



US007846635B2

(12) **United States Patent**  
Niimi

(10) **Patent No.:** **US 7,846,635 B2**  
(45) **Date of Patent:** **\*Dec. 7, 2010**

(54) **IMAGE FORMING APPARATUS, IMAGE FORMING METHOD AND PROCESS CARTRIDGE**

(75) Inventor: **Tatsuya Niimi**, Shizuoka-ken (JP)

(73) Assignee: **Ricoh Company, Ltd.**, Tokyo (JP)

(\*) Notice: Subject to any disclaimer, the term of this patent is extended or adjusted under 35 U.S.C. 154(b) by 897 days.

This patent is subject to a terminal disclaimer.

(21) Appl. No.: **11/669,957**

(22) Filed: **Feb. 1, 2007**

(65) **Prior Publication Data**

US 2008/0031653 A1 Feb. 7, 2008

(30) **Foreign Application Priority Data**

|               |      |       |             |
|---------------|------|-------|-------------|
| Feb. 6, 2006  | (JP) | ..... | 2006-028493 |
| Feb. 6, 2006  | (JP) | ..... | 2006-028494 |
| Jan. 12, 2007 | (JP) | ..... | 2007-004924 |
| Jan. 12, 2007 | (JP) | ..... | 2007-004925 |

(51) **Int. Cl.**

*G03G 5/087* (2006.01)  
*G03G 15/00* (2006.01)

(52) **U.S. Cl.** ..... **430/123.43; 430/123.4; 430/125.2; 430/57.2; 430/60; 399/159**

(58) **Field of Classification Search** ..... **430/125.2, 430/57.1, 123.4, 123.43, 60, 65, 57.2; 399/157, 399/159**

See application file for complete search history.

(56) **References Cited**

U.S. PATENT DOCUMENTS

|               |        |                  |       |          |
|---------------|--------|------------------|-------|----------|
| 4,959,288 A * | 9/1990 | Ong et al.       | ..... | 430/58.7 |
| 4,988,571 A * | 1/1991 | Ueda             | ..... | 430/59.6 |
| 5,378,570 A * | 1/1995 | Kobayashi et al. | ..... | 430/59.6 |

|                   |         |                |       |           |
|-------------------|---------|----------------|-------|-----------|
| 5,576,131 A *     | 11/1996 | Takai et al.   | ..... | 430/59.2  |
| 6,516,169 B2      | 2/2003  | Niimi et al.   | ..... |           |
| 6,803,162 B2      | 10/2004 | Niimi          | ..... |           |
| 2001/0014396 A1 * | 8/2001  | Tanaka et al.  | ..... | 428/402   |
| 2002/0028400 A1 * | 3/2002  | Shimada et al. | ..... | 430/58.05 |
| 2004/0002013 A1 * | 1/2004  | Bender et al.  | ..... | 430/58.65 |
| 2006/0292480 A1 * | 12/2006 | Niimi          | ..... | 430/124   |

FOREIGN PATENT DOCUMENTS

JP 2002-268255 9/2002

OTHER PUBLICATIONS

Tipaque® CR-EL Data Sheet < <http://www20.inetba.com/ishiharacorpusa/item416088.ctlg> > (retrieved Dec. 2, 2009).\*

(Continued)

*Primary Examiner*—Christopher RoDee

(74) *Attorney, Agent, or Firm*—Oblon, Spivak, McClelland, Maier & Neustadt, L.L.P.

(57) **ABSTRACT**

An image forming apparatus including an image bearing member for bearing a latent electrostatic image including a substrate, an intermediate layer containing a metal oxide and a photosensitive layer containing a charge transport layer and a charge generating layer containing an organic charge generating material, a charging device for charging the image bearing member, a writing device for writing the latent electrostatic image on the image bearing member by irradiating the image bearing member with light having a wavelength shorter than 450 nm which the metal oxide absorbs so that carriers can be generated, a developing device for developing the latent electrostatic image with a toner to form a visualized image, a transfer device for transferring the visualized image to a recording medium, a fixing device for fixing the transferred image on the recording image, and a discharging device for optically discharging residual charges on the image bearing member.

**17 Claims, 10 Drawing Sheets**



OTHER PUBLICATIONS

Diamond, Arthur S & David Weiss (eds.) *Handbook of Imaging Materials*, 2nd ed.. New York: Marcel-Dekker, Inc. (Nov. 2001) pp. 164-168.\*  
English language machine translation of JP 2002-268255 (Sep. 2002).\*

U.S. Appl. No. 11/625,873, filed Jan. 23, 2007, Niimi.

U.S. Appl. No. 11/611,179, filed Dec. 15, 2006, Niimi.

U.S. Appl. No. 11/855,553, filed Sep. 14, 2007, Inaba, et al.

\* cited by examiner

FIG. 1



FIG. 2



FIG. 3



FIG. 4



FIG. 5



FIG. 6



FIG. 7



FIG. 8



FIG. 9



FIG. 10



FIG. 11



FIG. 12



FIG. 13



FIG. 14



FIG. 15



FIG. 16



**IMAGE FORMING APPARATUS, IMAGE FORMING METHOD AND PROCESS CARTRIDGE**

**BACKGROUND OF THE INVENTION**

**1. Field of the Invention**

The present invention relates to an image forming apparatus, an image forming method and a process cartridge.

**2. Discussion of the Background**

Recently, the development of the information processing systems using electrophotography has been notably significant. Among these, optical printers, which convert information into digital signals to optically record the information, have been extremely improved in terms of the quality of printing and reliability. This digital recording technology is applied to not only printers but also typical photocopiers, which leads to the development of digital photocopiers. In addition, it is anticipated that a typical analogue photocopier using this digital recording technology is more and more demanded because such a photocopier has various kinds of information processing functions. Further, with the diffusion and the improvement of performance of home computers, the development of a digital color printer for outputting color images and documents increasingly speeds up.

In an electrophotographic image bearing member for use in these systems and devices, in general, a function separation type layered image bearing member is pervasively used, in which a charge generating layer is provided on a substrate with an optional intermediate layer therebetween and a charge transport layer is provided on the charge generating layer. Furthermore, to improve the mechanical or chemical resistance of an image bearing member, a surface protective layer can be formed as the surface layer thereof. When a surface charged image bearing member of this type is irradiated with light, the light transmits a charge transport layer and reaches a charge generating material in the charge generating layer. The charge generating material absorbs the light and generates charge carriers. The generated charge carriers are infused into the charge transport layer and transferred therein along the electric field generated by the charging to neutralize the surface charges of the image bearing member. As a result, a latent electrostatic image is formed on the surface of the image bearing member. Therefore, a combination of a charge generating material which absorbs near infrared and optical light and a charge transport material which does not hinder the transmission of the light absorbed in the charge generating material, i.e., absorbs optical light (yellow light range) and ultraviolet, is used for the function separation type layered image bearing member in most cases.

As a light source dealing with such a digital recording system, for example, small, inexpensive and reliable semiconductor lasers (LDs) and electroluminescence diodes (LEDs) are used in most cases. The oscillation wavelength of the most widely used LDs is in the near infrared range, i.e., from about 780 to about 800 nm. The luminous wavelength of a representative LED is 740 nm.

Recently, violet or blue LDs and LEDs having an oscillation wavelength shorter than 450 nm (i.e., from 375 to 450 nm) have been developed and introduced into the market as a writing light source dealing with the digital recording format for use in DVDs, etc. For example, when an LD having about a half oscillation wavelength in comparison with that of a typical near infrared LD is used as a writing light source, the spot diameter of the laser beam on an image bearing member can be theoretically significantly small as shown in the following relationship:  $d \propto (\pi/4) (\lambda f/D)$  (in the relationship, d

represents the spot diameter of a laser beam on an image bearing member,  $\lambda$  represents the wavelength of a laser beam, f represents the focusing length of an f0 lens and D represents the diameter of a lens). This is extremely advantagenous to improve the writing density, i.e., definition, of a latent electrostatic image.

When a light source having a wavelength shorter than 450 nm is used as a writing source, it is possible to irradiate an image bearing member with light having a beam (dot) spot of about 30  $\mu\text{m}$  corresponding to 1,200 dpi or about 15  $\mu\text{m}$  corresponding to 2,400 dpi while maintaining the clearness of the contour thereof.

Improvement on the quality of images and the durability, including colorization, is demanded for the printer and the photocopier mentioned above. There are two issues for the improvement on the quality of images for a digital apparatus. One is how to uniformly form a latent electrostatic image with fine dots. The other is how to reduce the occurrence of various kinds of abnormal images. The quality of images can be improved by using the light source mentioned above emitting light having a short wavelength. However, the occurrence of various kinds of abnormal images has been remained unsolved.

With regard to the improvement on durability, it is highly effective to elongate the life of an image bearing member.

There are various kinds of approaches to solve these issues. The thing common in both issues is how to restrain the deterioration of an image bearing member caused by electrostatic fatigue for use in these image forming apparatuses. To be specific, it is how to restrain the rise of the voltage at irradiated portions during repetitive use.

To restrain the rise of the voltage at irradiated portions, the design (composition, structure, etc.) of an image bearing member has been devised in the development so far. However, the electrostatic fatigue of an image bearing member greatly depends on the compositions thereof and the process conditions. From a point of development of an image bearing member, developers are required to deal with each process condition. Under these circumstances, the study on the electrostatic fatigue has hardly been made in terms of compositions of an image bearing member suitable for a short wavelength light source.

Published unexamined Japanese patent application No. (hereinafter referred to as JOP) 2002-268255 describes an image bearing member including a short wavelength light absorption layer, a photosensitive layer and a surface protective layer which are provided on a substrate. The short wavelength light absorption layer contains an N type like organic pigment and absorbs writing light having a wavelength of from 400 to 450 nm. Thereby, the occurrence of moiré is prevented. Due to this method, it is certain that the reflection from a substrate or a short wavelength light absorption layer does not occur so that the occurrence of moiré can be prevented.

However, this method involves a drawback in that an organic pigment is used. The short wavelength writing light source for use in the present invention has a large energy, which is equivalent to the second absorption band level energy of some of such organic materials. The mechanism of the generation of optical carriers of an organic material is described using the scheme shown in FIG. 1.

Most of the known mechanism so far is based on the reaction formed of the two steps (a first step from light excitation to generation of geminate pairs and a second step from the generation of geminate pairs to generation of free carriers) as shown in FIG. 1. The (A) charge generating material absorbs light and is excited to a higher excited state and the

geminate pairs are generated when the charge generating material is excited to a certain energy level. This certain energy level is the minimum excited singlet state ( $S_1$ ). Optical carriers are hardly produced by light having an energy smaller, which means light having a longer wavelength, than the difference between the ground level ( $S_0$ ) and the minimum excited singlet state ( $S_1$ ).

In contrast, in the case of the irradiation of light having an energy greater, which means light having a shorter wavelength, than the difference between the ground level ( $S_0$ ) and the minimum excited singlet state ( $S_1$ ), the energy state is excited to an energy level ( $S^*$ ) (an excited singlet state) than the minimum excited singlet state ( $S_1$ ) and rapidly relaxed to the minimum excited singlet state ( $S_1$ ) and the geminate pairs started to be formed. The energy corresponding to the difference between  $S^*$  and  $S_1$  is thermally relaxed (represented as extra energy shown in FIG. 1).

When this extra energy is extremely large, a reaction other than the thermal relaxing may occur directly at the excited state of a charge generating layer because the thermal relaxing is not sufficient to absorb the extra energy. For example, oxidization and decomposition of the material occur. When an organic pigment is used in a short wavelength light absorption layer, the organic pigment is used therein with a high density than in a charge generating layer to prevent reflection of the writing light almost perfectly. This has a large impact. Resultingly, the technology described in JOP 2002-268255 can prevent the occurrence of moiré but cannot continuously restrain the rise of the voltage at irradiated portion.

#### SUMMARY OF THE INVENTION

A need exists for an image forming apparatus and an image forming method by which the rise of the voltage at an irradiated portion can be restrained during repetitive use of an image bearing member to form fine and durable images.

Accordingly, an object of the present invention is to provide an image forming apparatus, an image forming method, and a process cartridge which can form fine images for an extended period of time.

Briefly this object and other objects of the present invention as hereinafter described will become more readily apparent and can be attained, either individually or in combination thereof, by an image forming apparatus including an image bearing member for bearing a latent electrostatic image including a substrate, an intermediate layer containing a metal oxide and a photosensitive layer formed of a charge transport layer and a charge generating layer containing an organic charge generating material, a charging device for charging the image bearing member, a writing device for writing the latent electrostatic image on the image bearing member by irradiating the image bearing member with light having a wavelength shorter than 450 nm which the metal oxide absorbs so that carriers can be generated, a developing device for developing the latent electrostatic image with a toner to form a visualized image, a transfer device for transferring the visualized image to a recording medium, a fixing device for fixing the transferred image on the recording image and a discharging device for optically discharging residual charges on the image bearing member.

It is preferred that, in the image forming apparatus mentioned above, the metal oxide is a non-surface treated metal oxide.

It is still further preferred that, in the image forming apparatus mentioned above, the metal oxide is a rutile type tita-

nium oxide and the writing device irradiates the image bearing member with light having a wavelength shorter than 410 nm.

It is still further preferred that, in the image forming apparatus mentioned above, the rutile type titanium oxide is a non-surface treated rutile type titanium oxide.

It is still further preferred that, in the image forming apparatus mentioned above, the transmission factor of the charge generating layer for the writing light is from 10 to 25%.

10 It is still further preferred that, in the image forming apparatus mentioned above, the transmission factor of the charge transport layer for the writing light is not less than 30%.

15 It is still further preferred that, in the image forming apparatus mentioned above, a protective layer is provided on the photosensitive layer.

It is still further preferred that, in the image forming apparatus mentioned above, the transmission factor of the protective layer for the writing light is not less than 30%.

It is still further preferred that, in the image forming apparatus mentioned above, the intermediate layer includes a charge blocking layer and a moiré prevention layer containing a metal oxide.

20 It is still further preferred that, in the image forming apparatus mentioned above, the charge blocking layer contains an insulating material and has a thickness of from 0.1 to less than 2.0  $\mu\text{m}$ .

25 It is still further preferred that, in the image forming apparatus mentioned above, the insulating material contains N-methoxymethylated nylon.

30 It is still further preferred that, in the image forming apparatus mentioned above, the moiré prevention layer further includes a binder resin and the ratio in volume of the metal oxide in the moiré prevention layer to the binder resin is from 1 to 3.

35 It is still further preferred that, in the image forming apparatus mentioned above, the discharging device includes a light source irradiating the image bearing member with light having a wavelength shorter than 450 nm which the metal oxide in the intermedia layer absorbs so that carriers can be generated.

40 It is still further preferred that the image forming apparatus mentioned above includes a plurality of image bearing members, charging devices, and writing devices.

45 It is still further preferred that the image bearing member, the charging device and the writing devices are integrally detachably attached to the image forming apparatus.

As another aspect of the present invention, an image forming method is provided which includes charging an image bearing member including a substrate, an intermediate layer 50 containing a metal oxide, a photosensitive layer formed of a charge transport layer and a charge generating layer containing an organic charge generating material, writing a latent electrostatic image on the image bearing member by irradiating the image bearing member with light having a wavelength shorter than 450 nm which the metal oxide absorbs so that carriers can be generated, developing the latent electrostatic image with a toner to form a visualized image, transferring the visualized image to a recording medium, fixing the transferred image on the recording medium, and discharging residual charges on the image bearing member.

55 It is preferred that, in the image forming method, the discharging device irradiates the image bearing member with light having a wavelength shorter than 450 nm which the metal oxide in the intermedia layer absorbs so that carriers can be generated.

60 It is still further preferred that the image forming method includes a plurality of charging processes and writing processes.

cesses. As another aspect of the present invention, a process cartridge is provided which includes an image bearing member for bearing a latent electrostatic image including a substrate, a photosensitive layer and an intermediate layer containing a metal oxide, a charging device for charging the image bearing member, and a writing device for writing the latent electrostatic image on the image bearing member by irradiating the image bearing member with light having a wavelength shorter than 450 nm which the metal oxide absorbs so that carriers can be generated.

These and other objects, features and advantages of the present invention will become apparent upon consideration of the following description of the preferred embodiments of the present invention taken in conjunction with the accompanying drawings.

#### BRIEF DESCRIPTION OF THE DRAWINGS

Various other objects, features and attendant advantages of the present invention will be more fully appreciated as the same becomes better understood from the detailed description when considered in connection with the accompanying drawings in which like reference characters designate like corresponding parts throughout and wherein:

FIG. 1 is a diagram illustrating the concept of the mechanism of photocarrier generation of an organic material;

FIG. 2 is a diagram illustrating the concept of the mechanism of photocarrier generation of an inorganic material;

FIG. 3 is a diagram illustrating an example of the layer structure of the image bearing member of the present invention;

FIG. 4 is a diagram illustrating another example of the layer structure of the image bearing member of the present invention;

FIG. 5 is a diagram illustrating another example of the layer structure of the image bearing member of the present invention;

FIG. 6 is a diagram illustrating the status of a liquid dispersion which is formed by a long dispersion time;

FIG. 7 is a diagram illustrating the status of a liquid dispersion which is formed by a short dispersion time;

FIG. 8 is a diagram illustrating the average particle diameter distribution and the particle size distribution of the liquid dispersions illustrated in FIGS. 6 and 7;

FIG. 9 is a schematic diagram illustrating an example of the present invention used for describing electrophotography process and an image forming apparatus;

FIG. 10 is a schematic diagram illustrating an example of the present invention used for describing a tandem type full color image forming apparatus;

FIG. 11 is a diagram illustrating an example of the process cartridge for use in the image forming apparatus of the present invention;

FIG. 12 is a diagram illustrating XD spectrum of titanyl phthalocyanine synthesized in Synthesis Example 1, which is described later;

FIG. 13 is a diagram illustrating SD spectrum of dried powder of water paste (wet cake);

FIG. 14 is a test shchart for use in Example 11, which is described later;

FIG. 15 is a test shchart for use in Example 16, which is described later; and

FIG. 16 is a test shchart for use in Example 33, which is described later.

#### DETAILED DESCRIPTION OF THE INVENTION

The present invention will be described below in detail with reference to several embodiments and accompanying drawings.

Embodiments of the present invention are about an image forming apparatus, an image forming method and a process cartridge containing or relating to an image bearing member having a photosensitive layer formed of a charge transport layer and a charge generating layer containing an organic charge generating material.

The present inventor has studied the electrostatic fatigue of an image bearing member, especially about the rise of the voltage at irradiated portion caused by strong irradiation, for example, by a laser beam during repetitive use of an image forming apparatus including the image bearing member.

With regard to the fatigue of an image bearing member during its repetitive use, generally the residual voltage of an image bearing member has been discussed. To evaluate residual voltage, the residual voltage, which has been defined as the voltage below which the surface voltage does not lower, is measured after several tens of seconds of irradiation of light having relatively low energy (about several  $\mu\text{W}/\text{cm}^2$  e.g., 4-7  $\mu\text{W}/\text{cm}^2$  on an image bearing member). This evaluation method is effective for an image forming apparatus using analogue light source, for example, a fluorescent lamp. Due to the analysis on the residual voltage of an image bearing member after its repetitive use, the result is obtained that the residual voltage is generated by a trap generated by the bulk of a charge transport layer. To reduce such a rise of the residual voltage, it is concluded that improvement of the design of a charge transport layer is desired.

However, in the case of an image forming apparatus using a digital light source as in the embodiments of the present invention, the amount of irradiation per unit time and unit area is extremely large (at least several hundreds of times when an LD is used for writing). Therefore, the characteristics of the optical extinction of an image bearing member is greatly different between the case of an analogue light source and the case of a digital light source. This difference has a large impact especially when a light source emitting light having a wavelength shorter than 450 nm is used for a high density writing with a small beam spot.

Under such a situation, the voltage at irradiated portions rises when an image bearing member having a substrate on which an intermediate layer, a charge generating layer and a charge transport layer are accumulated in this order is repetitively used. As a result of the analysis on this phenomenon, it is found that the response (transfer of positive and negative carriers) of the image bearing member to an extremely short writing in time is the key. With regard to the image bearing member, the development of a charge transport material contained in a charge transport layer has been in significant progress with the advance of size reduction and speed-up of an image forming apparatus. Currently used image bearing members can sufficiently deal with a high speed process, for example, a process of writing to development in 0.1 seconds or less. Therefore, among photocarriers generated in the charge generating layer, carriers (most thereof are positive holes) trespassing the charge transport layer are not a rate controlling factor of carrier transfer and hardly raise the voltage at irradiated portions during repetitive use.

On the other hand, carrier (most thereof are electrons) having a reversed polarity to the carriers infused into the charge transport layer are infused from the charge generating layer to the intermediate layer and transferred to the substrate.

Multiple functions are imparted to an intermediate layer contained in an image bearing member widely used in a current image forming apparatus. These are, for example, (i) transfer of photocarriers generated in a charge generating layer to a substrate, (ii) coverage of defects (scars, dirts, surface roughness, etc.) of a substrate, (iii) preventin of moiré (i.e., restraint of interference patterns caused by coherent light writing), (iv) prevention of infusion of charges having a reversed polarity to the polarity of a charged image bearing member from substrate, and (v) improvement on adhesibility between a photosensitive layer and a substrate.

In general, it is extremely difficult to have a good combination of the function of (i) and the function of (iv). In an organic photoconductor (OPC), in which an organic charge generating material is used in the charge generating layer, the surface of the organic photoconductor is negatively charged in operation. Therefore, the intermediate layer is required to transfer electrons among carriers generated in the charge generating layer. Also, it is desired to prevent infusion of positive holes from the substrate. In the intermediate layer, a material generally referred to as N type, which has a rectification property and transfers only electrons, is used. However, it is actually difficult to find a material having perfect N type property. Therefore, in most cases, either function of (i) or (iv) takes precedence over the other considering the balance thereof when designing an intermediate layer.

Most originals processed in the currently used negative positive development are monochrome with a writing ratio of 10% at most and most output image areas correspond to the background portion of an image bearing member. Therefore, when the functions of (i) and (iv) have a trade-off relationship, the function of (iv), i.e., the prevention of infusion of positive holes, is mainly considered when designing. This is because the portion corresponding to the background portion of an image bearing member occupies most of an image in the case of a monochrome original so that the image deficiency referred to as (the) background fouling occurs when the infusion of positive holes is not prevented. In addition, originals having gradation or solid images are rarely developed so that slight deterioration of the function of (i) (i.e., electron transport function) does not cause apparent reduction in image density.

The image forming apparatus of the present invention, which can produce quality images, is most effective in producing full color images. It is therefore desired to make a design suitable for full color image formation considering the feature. Different from monochrome images, full color images are developed with a relatively large writing ratio. Even a writing ratio of 100% is seen in some cases. Furthermore, gradation is frequently used in full color images so that color balance and color representation are more concerned than background fouling. However, image forming apparatuses are designed for both color images and monochrome images and background fouling is not still ignorable.

The present inventor has studied the behavior of electrons generated in a charge generating layer taking this point into consideration. From a structural reason of an image bearing member, an intermediate layer has a function of preventing infusion of positive holes from a substrate. It is deduced that infusion property of electron to an intermediate layer also deteriorates. The electron transport property of an intermediate layer is originally not so high but a poor electron infusion property thereof is considered to cause a rise in the voltage at irradiated portion for high density writing.

Generally, writing light is not completely absorbed in a charge generating layer. 10 to several 10s % thereof pass through a charge generating layer, which causes moiré

images. The present inventor thinks of using this passing light to generate photocarriers in an intermediate layer, by which the shortage of the number of electrons infusing from a charge generating layer can be compensated.

In embodiments of the present invention, the rise of the voltage at irradiated portion for high density writing can be restrained by an intermediate layer provided between a substrate and a photosensitive layer (a charge generating layer) and containing a metal oxide. The metal oxide absorbs writing light and photocarriers are generated in the intermediate layer.

FIG. 2 represents a schematic diagram illustrating the mechanism of generating photocarriers from an inorganic material. Generally, a band model is applied to the case of an inorganic material. The model shown in FIG. 2 formed of valence band and induction band is obtained. Electrons which obtain an energy corresponding to the band gap by light excitation can freely move at the valence band and are present as free carriers. In the conduction band area, electrons directly become free carriers. When an energy greater than the band gap is provided as shown in FIG. 1, carrier generation efficiency (ionic dissociation efficiency) is improved without producing extra energy. This is the significant difference between the mechanism of generating photocarriers from an organic image bearing member and that from an inorganic image bearing member. This accounts that the present invention is a technology produced based on a totally different idea from that described in JOP 2002-268255 including the stability against writing. The present invention was thus made.

The present invention is based on the knowledge mentioned above of the present inventor. Embodiment of the present invention include the following, but not limited thereto.

(1) An image forming apparatus including an image bearing member for bearing a latent electrostatic image, a charging device for charging the image bearing member, a writing device, a developing device, a transfer device for transferring the visualized image to a recording medium, a fixing device and a discharging device. The image bearing member includes a substrate, an intermediate layer containing a metal oxide and a photosensitive layer formed of a charge transport layer and a charge generating layer containing an organic charge generating material. The writing device writes the latent electrostatic image on the image bearing member by irradiating the image bearing member with light having a wavelength shorter than 450 nm which the metal oxide absorbs so that carriers can be generated. The developing device develops the latent electrostatic image with a toner to form a visualized image. The transfer device transfers the visualized image to a recording medium. The fixing device fixes the transferred image on the recording image. The discharging device optically discharges residual charges on the image bearing member.

(2) The image forming apparatus mentioned above, in which the metal oxide is a non-surface treated metal oxide.

(3) The image forming apparatus mentioned above, in which the metal oxide is a rutile type titanium oxide and the writing device irradiates the image bearing member with light having a wavelength shorter than 410 nm.

(4) The image forming apparatus mentioned above in (3), in which the rutile type titanium oxide is a non-surface treated rutile type titanium oxide.

(5) The image forming apparatus mentioned above, in which the transmission factor of the charge generating layer for the writing light is from 10 to 25%.

(6) The image forming apparatus mentioned above, in which the organic charge generating material is an azo pigment represented by the following chemical structure 1.



In the chemical structure 1, Cp<sub>1</sub> and Cp<sub>2</sub> individually represent coupler residue groups. R<sub>201</sub> and R<sub>202</sub> independently denote one of hydrogen atom, a halogen atom, an alkyl group, an alkoxy group, and cyano group. Cp<sub>1</sub> and Cp<sub>2</sub> are represented by the following chemical structure 2:



In the chemical structure 2, R<sub>203</sub> represents one of hydrogen atom, an alkyl group, for example, methyl group and ethyl group, and an aryl group, for example, phenyl group. R<sub>204</sub>, R<sub>205</sub>, R<sub>206</sub>, R<sub>207</sub> and R<sub>208</sub> independently represent one of hydrogen atom, nitro group, cyano group, a halogen atom, for example, fluorine atom, chlorine atom, bromium atom and iodine atom, an alkyl group, for example, methyl group and ethyl group, an alkoxy group, for example, methoxy group and ethoxy group, dialkyl amino group and hydroxyl group. Z represents an atom group forming a substituted or non-substituted aromatic carbon ring or a substituted or non-substituted aromatic heterocyclic ring.

(7) The image forming apparatus mentioned in (6), in which Cp<sub>1</sub> and Cp<sub>2</sub> are different substitutional groups from each other.

(8) The image forming apparatus mentioned above, in which the organic charge generating material is titanyl phthalocyanine crystal having a CuK $\alpha$  X ray diffraction spectrum having a wavelength of 1.542 Å such that a maximum diffraction peak is observed at a Bragg (20) angle of 27.2±0.2°, main peaks at a Bragg (20) angle of 9.4±0.2°, 9.6±0.2°, and 24.0±0.2°, and a peak at a Bragg (20) angle of 7.3±0.2° as the lowest angle diffraction peak, and having no peak between the peak of 9.4±0.2° peak and the peak of 7.3±0.2° and no peak at 26.3°.

(9) The image forming apparatus mentioned above, in which the transmission factor of the charge transport layer for the writing light is not less than 30%.

(10) The image forming apparatus mentioned above, in which a protective layer is provided on the photosensitive layer.

(11) The image forming apparatus mentioned in (10), in which the transmission factor of the protective layer for the writing light is not less than 30%.

(12) The image forming apparatus mentioned in (10) or (11), in which the protective layer contains at least one of an inorganic pigment and a metal oxide having a specific resistance of not less than 10<sup>10</sup> Ω·cm.

(13) The image forming apparatus mentioned above in (10) or (11), in which the protective layer is formed by curing a radical polymerizable monomer having at least three functional groups which does not have a charge transport structure and a radical polymerizable compound having one functional group which has a charge transport structure.

(14) The image forming apparatus mentioned above in (13), in which the radical polymeric compound having one functional group which has a charge transport structure for use in the protective layer is at least one kind represented by the following chemical structures 3 and 4:



In the chemical structures 3 and 4, R<sub>1</sub> represents hydrogen atom, a halogen atom, an alkyl group, an aralkyl group, an aryl group, cyano group, nitro group, an alkoxy group, —COOR<sub>7</sub>, wherein R<sub>7</sub> represents hydrogen atom, a substituted or non-substituted alkyl group, a substituted or non-substituted aralkyl group or a substituted or non-substituted aryl group, a halogenated carbonyl group or CONR<sub>8</sub>R<sub>9</sub>, wherein R<sub>8</sub> and R<sub>9</sub> independently represent hydrogen atom, a halogen atom, a substituted or non-substituted alkyl group, a substituted or non-substituted aralkyl group or a substituted or non-substituted aryl group, Ar<sub>1</sub> and Ar<sub>2</sub> independently represent a substituted or unsubstituted arylene group, Ar<sub>3</sub> and Ar<sub>4</sub> independently represent a substituted or unsubstituted aryl group, X represents a substituted or non-substituted alkylene group, a substituted or non-substituted cycloalkylene group, a substituted or non-substituted alkylene ether group, oxygen atom, sulfur atom or a vinylene group, Z represents a substituted or non-substituted alkylene group, a substituted or non-substituted alkylene ether divalent group or an alkyleneoxy carbonyl divalent group, and a represents 0 or 1, m and n represent an integer of from 0 to 3.

(15) The image forming apparatus mentioned in (13) or (14), in which the radical polymerizable compound having one functional group which has a charge transport structure for use in the protective layer is at least one kind represented by the following chemical structure 5:



In the chemical structure 5, u, r, p, q represent 0 or 1, s and t represent an integer of from 0 to 3, Ra represents hydrogen atom or methyl group, Rb and Rc independently represent an alkyl group having 1 to 6 carbon atoms, and Za represents methylene group, ethylene group,  $-\text{CH}_2\text{CH}_2\text{O}-$ ,  $-\text{CHCH}_3\text{CH}_2\text{O}-$ , or  $-\text{C}_6\text{H}_5\text{CH}_2\text{CH}_2-$ .

(16) The image forming apparatus mentioned in (13) to (15), in which the protective layer is cured by a thermal or light energy irradiation device.

(17) The image forming apparatus mentioned above, in which the intermediate layer includes a charge blocking layer and a moiré prevention layer containing a metal oxide.

(18) The image forming apparatus mentioned in (17), in which the charge blocking layer contains an insulating material and has a thickness of from 0.1 to less than 2.0  $\mu\text{m}$ .

(19) The image forming apparatus mentioned in (18), in which the insulating material contains N-methoxymethylated nylon.

(20) The image forming apparatus mentioned in (17) or (19), in which the moiré prevention layer further contains a binder resin and a ratio in volume of the metal oxide in the moiré prevention layer to the binder resin is from 1 to 3.

(21) The image forming apparatus mentioned above, in which the discharging device includes a light source irradiating the image bearing member with light having a wavelength shorter than 450 nm which the metal oxide in the intermedia layer absorbs so that carriers can be generated.

(22) The image forming apparatus mentioned above, which includes a plurality of image bearing members, charging devices, and writing devices.

(23) The image forming apparatus mentioned above, in which the image bearing member, the charging device and the writing devices are integrally detachably attached to the image forming apparatus.

(24) An image forming method including: charging an image bearing member including a substrate, an intermediate layer containing a metal oxide, a photosensitive layer including a charge transport layer and a charge generating layer containing an organic charge generating material; writing a latent electrostatic image on the image bearing member by irradiating the image bearing member with light having a wavelength shorter than 450 nm which the metal oxide absorbs so that carriers can be generated; developing the latent electrostatic image with a toner to form a visualized image; transferring the visualized image to a recording medium; fixing the transferred image on the recording medium; and discharging residual charges on the image bearing member.

(25) The image forming method mentioned above, in which the discharging device includes a light source irradiating the image bearing member with light having a wavelength shorter than 450 nm which the metal oxide in the intermedia layer absorbs so that carriers can be generated.

(26) An image forming method including: charging an image bearing member including a substrate, an intermediate layer containing a rutile type titanium oxide, a photosensitive layer including a charge transport layer and a charge generating layer containing an organic charge generating material; writing a latent electrostatic image on the image bearing member by irradiating the image bearing member with light having a wavelength shorter than 410 nm; developing the latent electrostatic image with a toner to form a visualized image; transferring the visualized image to a recording medium; fixing the transferred image on the recording medium; and discharging residual charges on the image bearing member.

(27) The image forming method mentioned in (26), in which the light source for use in the discharging device emits light having a wavelength shorter than 410 nm.

30 (28) The image forming method mentioned above, which includes a plurality of charging processes and writing processes.

(29) A process cartridge includes an image bearing member including a substrate, a photosensitive layer and an intermediate layer containing a metal oxide, a charging device for charging the image bearing member and a writing device for writing a latent electrostatic image by irradiating the image bearing member with light having a wavelength shorter than 450 nm which the metal oxide absorbs so that carriers can be generated.

(30) A process cartridge includes an image bearing member including a substrate, a photosensitive layer and an intermediate layer containing a rutile type titanium oxide, a charging device for charging the image bearing member and a writing device for writing a latent electrostatic image by irradiating the image bearing member with light having a wavelength shorter than 410 nm.

The wavelength of the writing light mentioned in embodiments of the present invention that is absorbed by the metal oxide so that carriers can be generated is defined as the wavelength of light having an energy greater than the energy corresponding to the width (referred to as energy gap or band gap between the conduction band and the valence band) of the 50 forbidden band of a metal oxide. When a rutile type titanium oxide is used, the energy gap is 3.0 eV, which is about 410 nm in wavelength conversion. This wavelength is the longest wavelength of writing light which can be absorbed by the 55 rutile type titanium oxide. Namely, light having a wavelength shorter than 410 nm can be absorbed by the rutile type titanium oxide and can generate carriers.

The wavelength of writing light which a metal oxide can absorb so that carriers can be generated is defined as the wavelength of light having a larger energy than the energy gap as described above. The method of measuring the energy gap is described below. In general, there are three methods therefore.

The first method is a method in which the spectroscopic reflective spectrum of an intermediate layer is measured to obtain the absorption end on the long wavelength side. This can be easily measured with a spectroscopic absorption spectrum device in the market. This method is used in Examples and Comparative Examples of the present invention. The wavelength of light which can be absorbed by an intermediate layer is obtained as the wavelength on the shorter wavelength side than the absorption end obtained by this method.

The second method is a method in which, after the spectroscopic absorption spectrum and the luminescence spectrum of an intermediate layer are obtained, both spectra are plotted in the same graph to obtain the wavelength of the intersection thereof. These can be measured by a spectrophotometer and a spectrophotofluorometer in the market. The wavelength of light which can be absorbed by an intermediate layer is obtained as the wavelength on the shorter wavelength side than the wavelength (intersection) obtained by the method.

The third method is a method in which the difference between measured energy levels of the electroconductive band and of the valance band is obtained as the energy gap. This method requires an exclusive device and is not prevalent. The wavelength of light which can be absorbed by an intermediate layer is obtained as the wavelength on the shorter wavelength side than the wavelength obtained by converting the energy gap (the unit of which is energy) in the wavelength unit.

The writing light having a wavelength shorter than 450 nm for use in embodiments of the present invention represents light which does not substantially (ignorably) or completely include light having a wavelength not shorter than 450 nm. Similarly, the discharging light having a wavelength shorter than 450 nm for use in embodiments of the present invention represents light which does not substantially (ignorably) or completely include light having a wavelength not shorter than 450 nm. The same applies to the discharging light having a wavelength shorter than 410 nm.

The mechanism of how the rise of the residual voltage of an image bearing member during repetitive use thererof can be restrained by using discharging light which can be absorbed by a metal oxide is not clear in detail. Currently, the considerable mechanism is described as follows.

When writing is performed by using light having a wavelength longer than the wavelength of light which can be absorbed by a metal oxide during repetitive use of an image bearing member, all the photocarriers generated in the image bearing member are produced in the charge generating layer. The positive holes produced are infused into the charge generating layer and the electron produced are infused into the intermediate layer. Each thereof is transferred to either of the surface of the image bearing member or the substrate thereof to cancel the surface charges or induced charges (the charges induced on the substrate side during the main charging). In the high speed process targeted by the present invention, the electron transport speed in the intermediate layer is slower than the positive hole transport speed in the charge generating layer. Therefore, electrons are accumulated in the intermediate layer during repetitive use. In addition, the infusion property of electrons from the charge generating layer to the intermediate layer is not sufficient so that electrons are accumulated in the interface between the charge generating layer and the intermediate layer.

In contrast, when writing is performed by using light which can be absorbed by the metal oxide, photocarriers are produced in a charge generating layer but the writing light is not completely absorbed in the charge generating layer and a part

thereof reaches an intermediate layer. When the intermediate layer contains a metal oxide which can absorb the writing light, the metal oxide in the intermediate layer absorbs the writing light and produces photocarriers via a photoexcitation state. Since the photocarriers are produced in the intermediate layer, there is no infusion process of photocarriers from the charge generating layer, resulting in good efficiency. The photocarriers produced in the intermediate layer cancel the residual charges (electrons) accumulated at or before the prior image formation so that the rise of the residual voltage can be restrained.

In addition, a typical organic charge generating material for use in a charge generating layer absorbs optical light and passes writing light having a wavelength shorter than 450 nm in some extent so that a sufficient amount of light reaches an intermediate layer and can produce photocarriers therein. In addition, the organic charge generating material does not completely absorb light having a wavelength shorter than 450 nm due in terms of the structure thereof. Therefore, since a sufficient amount of photocarriers can be produced in the charge generating layer as in the case of writing light having a wavelength of not shorter than 450 nm, the writing light having a wavelength shorter than 450 nm does not have an adverse impact on optical writing itself.

To sufficiently obtain this effect, it is desired that the discharging light reaches the intermediate layer in an image bearing member in a sufficient amount. To achieve this, the discharging light having a wavelength shorter than 450 nm passes through the charge generating layer and the charge transport layer, which are provided on or above the intermediate layer, in a sufficient amount.

In the charge generating layer, a transmission ratio for writing light that is too large may cause reduction of the occurrence of carriers. When a transmission ratio for writing light is too small, the writing light may not reach the intermediate layer. Namely, there is a suitable range therefor, which is from 10 to 25%. In this range, a balanced designing is possible.

With regard to the charge transport layer, when the charge transport layer absorbs writing light, various kinds of side effects occur. For example, writing light does not reach the charge generating layer and the intermediate layer which are located under the charge transport layer and the charge generating material contained therein rapidly deteriorate. Therefore, the transmission ratio of the charge transport layer for writing light is preferably not less than 30%, more preferably not less than 50% and further preferably not less than 85%.

Some of the materials suitably used as the charge transport materials for use in an image bearing member absorb light having a wavelength shorter than 450 nm. The effect of the present invention may be not sufficiently obtained with such materials. In addition, it is not possible to secure the stability of electrostatic characteristics of an image bearing member during repetitive use thereof even with a material which passes light having a wavelength shorter than 450 nm when the material does not have a sufficient charge transport ability.

Thereofre, the desired characteristics of the charge transport material for use in the present invention are, for example; (1) the light having a wavelength shorter than 450 nm passes through the charge transport material in the state in which a charge transport layer is formed. To be specific, it is preferred that at least 30% of the discharging light passes through the charge transport material; (2) the charge transport material has good compatibility, for example, energy matching, with an organic charge generating material. Thereby, the photocarriers generated in the charge generating layer can be smoothly infused; and (3) the charge transport material has a stability

during repetitive use of an image bearing member as a material. Specific examples thereof include the durability against oxidation gasses produced by a charging device and the stability against conduction for an extended period of time.

The effect of the present invention is all the more apparent by having a structure satisfying the conditions described above. An embodiment of the present invention is a durable image forming apparatus including an image bearing member having an intermediate layer containing a metal oxide, a photosensitive layer containing a charge transport layer and a charge generating layer containing an organic charge generating material and using a light source emitting light having a wavelength shorter than 450 nm which the metal oxide absorbs so that carriers can be generated as the writing light source. Thereby, the present invention can provide an image forming apparatus, an image forming method and a process cartridge which can solve typical problems in related arts.

#### Image Forming Apparatus and Image Forming Method

The image forming apparatus includes an image bearing member, an image forming device, a charging device, a writing device, a transfer device, a fixing device and a discharging device and can have optional other devices, for example, a cleaning device, a recycling device and a controlling device. The image bearing member includes a substrate on or above which an intermediate layer containing a metal oxide and a layered photosensitive layer are provided. The layered photosensitive layer includes a charge generating layer containing an organic charge generating material and a charge transport layer. The writing device includes a light source emitting light having a wavelength shorter than 450 nm which the metal oxide absorbs so that carriers can be generated.

The image forming method of the present invention includes, a charging process, a writing process, a developing process, a transfer process, a discharging process and a fixing process, and can optionally have other processes, for example, a cleaning process, a recycling process and a controlling process. In the writing process, a light source emitting light having a wavelength shorter than 450 nm which a metal oxide can absorb so that carriers are generated is used. The image forming method of the present invention can be suitably performed by the image forming apparatus of the present invention. The charging process can be performed by the charging device. The writing process can be performed by the writing device mentioned above. The developing process can be performed by the developing device mentioned above. The developing process can be performed by the developing device mentioned above. The transfer process can be performed by the transfer device mentioned above. The discharging process can be performed by the discharging device mentioned above. The fixing process can be performed by the fixing device mentioned above. The other processes can be performed by the other devices mentioned above.

The image forming apparatus of the present invention includes an image bearing member, a charging device for charging the image bearing member, a writing device for writing a latent electrostatic image thereon, a developing device for developing the latent electrostatic image with a toner to visualize the image, a transfer device for transferring the visualized image to a recording medium, a discharging device for discharging the image bearing member to remove residual charges thereon and a fixing device for fixing the transferred image transferred on the recording medium. The writing device includes a light source irradiating the image bearing member with writing light having a wavelength shorter than 450 nm which a metal oxide can absorb so that carriers can be generated.

#### Image Bearing Member

As long as a metal oxide is contained in the intermediate layer and an organic charge generating material is contained in the charge generating layer, there is no specific limit to the image bearing member with regard to its composition, form, structure, size, etc. Any known image bearing member can be selected for use. As for the substrate, an electroconductive substrate is preferred.

Next, the image bearing member for use in the present invention is described in detail with reference to drawings.

FIG. 3 is a cross section illustrating an example of the structure of the image bearing member for use in the present invention. The structure is a layered structure in which an intermediate layer 39, a charge generating layer 35 and a charge transport layer 37 are provided on or above a substrate 31. The charge generating layer 35 and the charge transport layer 37 form a photosensitive layer 38. The intermediate layer 39 contains a metal oxide. The charge generating layer 35 contains an organic charge generating material as the charge generating material. The main content of the charge transport layer 37 is a charge transport material.

FIG. 4 is a cross section illustrating another example of the structure of the image bearing member for use in the present invention. The intermediate layer 39 includes a charge blocking layer 43 and a moiré prevention layer 45 containing a metal oxide. The charge generating layer 35 containing an organic charge generating material as the charge generating material and the charge transport layer 37 containing a charge transport material as its main component form the photosensitive layer 38 and are accumulated on the intermediate layer 39.

FIG. 5 is a cross section illustrating yet another example of the structure of the image bearing member for use in the present invention. There are provided on the substrate 31 the intermediate layer 39 containing a metal oxide, the charge generating layer 35 containing an organic charge generating material as the charge generating material, the charge transport layer 37 containing a charge transport material as its main component. The charge generating layer 35 and the charge transport layer 37 form a photosensitive layer 38. Furthermore, a protective layer 41 is provided on the charge transport layer 37.

Materials having a volume resistance of not greater than  $10^{10} \Omega \cdot \text{cm}$  can be used as a material for the substrate 31. For example, there can be used plastic or paper having a film form or cylindrical form covered with a metal, for example, aluminum, nickel, chrome, nichrome, copper, gold, silver, and platinum, or a metal oxide, for example, tin oxide and indium oxide by depositing or sputtering. Also a board formed of aluminum, aluminum alloy, nickel, or stainless metal can be used. Further, a tube which is manufactured from the board mentioned above by a crafting technique, for example, extruding and extracting, and surface-treatment, for example, cutting, super finishing and glinding, is also usable. In addition, an endless nickel belt and an endless stainless belt can be used as the substrate 31.

An electroconductive substrate can be formed by applying to the substrate 31 a liquid of application in which electroconductive powder is dispersed in a suitable binder resin can be used as the electroconductive substrate for use in the present invention.

Specific examples of such electroconductive powder include carbon black, acetylene black, metal powder, for example, powder of aluminum, nickel, iron, nichrome, copper, zinc and silver, and metal oxide powder, for example, electroconductive tin oxide powder and ITO powder.

Specific examples of the binder resins which are used together with the electroconductive powder include thermoplastic resins, thermosetting resins, and optical curing resins, for example, a polystyrene, a styrene-acrylonitrile copolymer, a styrene-butadiene copolymer, a styrene-anhydride maleic acid copolymer, a polyester, a polyvinyl chloride, a vinyl chloride-vinyl acetate copolymer, a polyvinyl acetate, a polyvinylidene chloride, a polyarylate (PAR) resin, a phenoxy resin, polycarbonate, a cellulose acetate resin, an ethyl cellulose resin, a polyvinyl butyral, a polyvinyl formal, a polyvinyl toluene, a poly-N-vinyl carbazole, an acrylic resin, a silicone resin, an epoxy resin, a melamine resin, an urethane resin, a phenol resin, and an alkyd resin. Such an electroconductive layer can be formed by dispersing the electroconductive powder and the binder resins mentioned above in a suitable solvent, for example, tetrahydrofuran (THF), dichloromethane (MDC), methyl ethyl ketone (MEK), and toluene and applying the resultant to a substrate.

Also, an electroconductive substrate formed by providing a heat contraction tube on a suitable cylindrical substrate as an electroconductive layer can be used as the substrate 31 of the present invention. The heat contraction tube can be formed of a material, for example, polyvinyl chloride, polypropylene, polyester, polystyrene, polyvinylidene chloride, polyethylene, chloride rubber, and TEFLON® in which the electroconductive powder mentioned above is contained.

Among these, an aluminum cylindrical substrate, which can be easily subject to anodic oxidization film forming treatment, is most preferred for use. The aluminum means solid aluminum or aluminum alloy. To be specific, aluminum or aluminum alloy of JIS 1000 to 1999, 3000 to 3999 and 6,000 to 6,999 are most suitable. Anodic oxidized film is formed by anodic oxidizing various kinds of metals and alloyed metals in an electrolyte solution. Among these, a film referred to as alumite formed by anodic oxidizing aluminum or aluminum alloy in an electrolyte solution is most suitable for an image bearing member. Especially, this film is excellent in preventing the point deficiency (black spot and background fouling) which occurs when the reversal development (negative and positive development) is used.

Anodic oxidization treatment is conducted in acid bathing using, for example, chromium acid, sulfuric acid, oxalic acid, phosphoric acid, acidum boricum and sulfamic acid. Among these, sulfuric acid bathing is most preferred. For example, the anodic oxidization treatment is conducted under the conditions of the density of sulfuric acid of from 10 to 20%, bathing temperature of from 5 to 25°C., electricity density of from 1 to 4 A/dm<sup>2</sup>, electrolyzation voltage of from 5 to 30 V and treatment time of from about 5 to about 60 minutes but is not limited thereto. The thus formed anodic oxidized film is porous and has a high insulation property so that the surface of the film is extremely unstable. Therefore, the physicality of the anodic oxidized film tends to change over time. To avoid this change, the anodic oxidized film is preferably subject to sealing treatment. There are methods of sealing, for example, a method of dipping an anodic oxidized film in an aqueous solution containing nickel fluoride and nickel acetate, a method of dipping an anodic oxidized film in boiling water, and a method of using pressurized vapor. Among these, the method of dipping an anodic oxidized film in an aqueous solution containing nickel acetate is most preferred. Washing treatment of the anodic oxidized film follows the sealing treatment. This treatment is to remove excessive materials, for example, metal salts, attached while in the sealing treatment. When these excessive materials remain on the surface of a substrate (i.e., an anodic oxidized film), such materials may have an adverse impact on the quality of the layer formed

on the substrate and cause background fouling because the materials have a low resistance in general. The washing treatment can be done with purified water only once but normally is performed through multiple stages. It is preferred to use water as clean (deionized) as possible for the last washing treatment. In addition, it is also preferred that abrasive washing using an abrasive member is included in the multiple washing stages. The thus obtained anodic oxidized film preferably has a thickness of from about 5 to about 15 µm. An anodic oxidized film that is too thin tends to have an insufficient barrier effect and an anodic oxidized film that is too thick tends to have too large a time constant as an electrode so that the residual voltage may rise and the response of an image bearing member worsen.

Next, the intermediate layer 39 is described. The intermediate layer for use in the present invention contains a metal oxide. In general, an intermediate layer is mainly formed of a resin. Considering the case in which a photosensitive layer is formed on the intermediate layer (i.e., resin) using a solvent, the resin is preferably hardly soluble in a typically used organic solvent. Specific examples of such resins include water soluble resins, for example, polyvinyl alcohol, casein, and sodium polyacrylate, alcohol soluble resins, for example, copolymerized nylon and methoxymethylized nylon and curing resins, for example, polyurethane, melamine resins, phenol resins, alkyd-melamine resins and epoxy resins, which form a three-dimensional mesh structure.

In addition, the intermediate layer 39 contains a metal oxide to reduce the residual voltage and to prevent the occurrence of moiré in addition. The absorption wavelength range of the metal oxide varies depending on impurities contained therein. Therefore, as mentioned before, the absorption wavelength range is obtained by actually measuring the energy gap of the used material or an intermediate layer containing the material. Specific examples of the metal oxide include titanium oxides, silica, alumina, zirconium oxides, tin oxides and indium oxides. Among these, titanium oxides and tin oxides are effectively used. Among the titanium oxides, rutile type titanium oxides are preferred. Anatase type titanium oxides can be also used. Considering that photocarriers are generated and light the anatase type titanium oxide can absorb has a wavelength shorter than that of light the rutile type titanium oxide can absorb, the writing light is preferred to have a short wavelength for the anatase type titanium oxide. Taking into account the spectroscopic transmission factor of a charge generating layer, the selection of the charge generating material may be relatively limited in the case of the anatase type titanium oxide when compared with the rutile type titanium oxide. Therefore, the rutile type titanium oxide is more preferred.

In addition, it is preferred to use a non-surface treated metal oxide as the metal oxide. This is because non-surface treated surface area of a metal oxide decreases with surface treatment, which has an adverse impact on the transport of carriers produced by the metal oxide, resulting in the deterioration of the effect of the present invention. When a surface treated metal oxide is used to improve, for example, dispersion stability, the degree of the sufface treatment is limited to the minimal level.

These intermediate layers 39 can be formed by using a suitable solvent and a suitable coating method, which are described later. The thickness of the intermediate layer 39 is preferably from 0.1 to 5 µm.

The intermediate layer 39 has at least two functions in addition to the generation of photocarriers at the time of writing. One is a function of preventing charges having a reverse polarity induced at the electrode when an image bear-

ing member is charged from infusing into the photosensitive layer **38**. The other is a function of preventing the production of moiré images which may occur when writing is performed with a coherent light, for example, a laser beam. It is effective to use a function separation type intermediate layer in which these two functions are independently provided by two or more layers for an image bearing member for use in the present invention. The charge blocking layer **43** and the moiré prevention layer **45** of a function separation type intermediate layer are described below.

The charge blocking layer **43** has a function of preventing charges having a reverse polarity induced at the electrode (substrate **31**) when an image bearing member is charged from infusing from the substrate **31** to the photosensitive layer **38**. In the case of negative charging, induced positive holes are prevented by this function. When positively charged, induced electrons are prevented thereby. As specific examples of the charge blocking layer, there are an anodic oxidized film represented by aluminum oxidized layer, an insulating layer formed by inorganic material represented by SiO, a layer formed by glassy network of a metal oxide, a layer formed of polyphosphazene, a layer formed of an aminosilane reactive product, a layer formed of an insulating binder resin, and a layer formed of a curing resin. Among these, the layer formed of an insulating binder resin or a curing resin, which can be formed by a wet application method, can be preferably used. When the moiré prevention layer **45** and the photosensitive layer **38** are formed on or above the charge blocking layer **43** by a wet application method, the charge blocking layer is desired to be formed by a material or a composition insoluble in the liquid of application for use in the wet application method.

Specific examples of the binder resin include thermoplastic resins, for example, polyamides, polyesters, and copolymers of vinyl chlorides and vinyl acetates, and thermocuring resins, for example, a thermocuring resin formed by thermally polymerizing a compound having multiple active hydrogens (hydrogens contained in —OH group, —NH<sub>2</sub> group, —NH group, etc.), a compound having multiple isocyanate groups, and optionally a compound having multiple epoxy resins. Specific examples of the compound having multiple active hydrogens include polyvinyl butyral, phenoxy resins, phenol resins, polyamides, polyesters, polyethylene glycols, polypropylene glycols, polybutylene glycol, and acrylic resins containing a hydroxyl ethyl methacrylate group containing active hydrogens. Specific examples of the compound having multiple isocyanate groups include tolylene diisocyanate, hexamethylene diisocyanate, and diphenyl methane diisocyanate and their polymers. Specific examples of the compound having multiple epoxy groups include bisphenol A type epoxy resins. Among these, in terms of film forming property, environmental stability and anti-chemical property, polyamides resins are most preferred. Among the polyamides, N-methoxy methylated nylon is most suitable. N-methoxy methylated nylon can be obtained by modifying a polyamide containing polyamide 6 as its comopnsnt by the method proposed by, for example, T. L. Cairns (J. Am. Chem. Soc. 71. P 651, published in 1949). N-methoxy methylated nylon is obtained by substituting the hydrogen in the amide linkage of the original polyamide with methoxymethyl group. The substitution ratio can be determined from a wide range according to the modification condition. The ratio is preferably not less than 15 mol % and more preferably not less than 35 mol % to restrain the hydroscopic property in some degree and have a good affinity for alcohol and environmental stability. In addition, as the amide substitution ratio (the degree of N—N-methoxy methylation) increases, alco-

hol solution affinity increases. However, since the influence of side chain groups on the bulk side around the main chain becomes strong, the relaxed state of the main chain, the coordination state between the main chains, etc. change. Thereby, the hydroscopic property increases while the crystallization property decreases, which leads to the drop of the melting point and the deterioration of the mechanical strength and elasticity. Therefore, the substitution ratio is preferably not greater than 85 mol % and more preferably not greater than 70 mol %. As the result of the study, it is found that nylon 6 is preferred and then nylon 66 is next preferred but copolymerized nylon of nylons 6, 66 and 610 is not so preferred contrary to the description in JOP H09-265202.

In addition, a thermoplastic resin formed by thermally polymerizing an oil free alkyd resin and an amino resin, for example, butylated melamin resins, and a photocuring resin formed of a combination of a resin having an unsaturated linkage, for example, a polyurethane having an unsaturated linkage and/or an unsaturated polyester, and a photopolymerization initiator, for example, a thioxanthone based compound and methylbenzyl formate can be used as the binder resin.

It is also good to have a function of restraining the infusion of charges from a substrate by adding an electroconductive polymer having a rectification property and/or an acceptor or donor resin/compound selected according to the charging polarity.

Furthermore, the thickness of the charge blocking layer is from 0.1 to less than 2.0  $\mu\text{m}$  and preferably from 0.3 to less than 2.0  $\mu\text{m}$ . When a charge blocking layer that is too thick is used, the residual voltage tends to significantly rise due to repetitive charging and irradiation especially in a low temperature and low humidity environment. When a charge blocking layer that is too thin is used, the blocking effect tends to be reduced. A charge blocking layer can be formed on a substrate by a known method, for example, a blade coating method, a dip coating method, a spray coating method, a beat coating method and a nozzle coating method. Medicines, solvents, additives, curing promoting agents, etc., can be added, if desired. Subsequent to coating, curing or drying treatment by, for example, drying, heating, and/or light, is conducted.

The moiré prevention layer **45** is a layer having a function of preventing the production of moiré images caused by optical coherence inside the photosensitive layer **38** when writing is performed by a coherent light, for example, a laser beam. To form a function separation type intermediate layer, the moiré prevention layer **45** contains a metal oxide so that the moiré prevention layer **45** can have a function of generating photo-carriers upon application of discharging light. Fundamentally, the moiré prevention layer **45** has a function of scattering the writing light mentioned above. Therefore, it is effective for the moiré prevention layer **45** to contain a material having a large refraction index.

When the intermediate layer **39** is structured by the charge blocking layer **43** and the moiré prevention layer **45**, the effect is significantly increased by contacting the moiré prevention layer **45** with the charge generating layer **35**, which is one of the most effective structures of an image bearing member.

In addition, an image bearing member having a function separation type intermediate layer prevents the infusion of charges from the substrate **31** at the charge blocking layer **43**. It is preferred that the moiré prevention layer **45** has a function of at least transporting charges having the same polarity as the charges on the surface of the image bearing member in terms of prevention of the rise of the residual voltage. For example, in the case of a negatively charged image bearing member, it

is preferred to impart electroconductivity to the moiré prevention layer 45. Therefore, it is preferred to use a metal oxide having electron conductivity or an electroconductive metal oxide. The effect of the present invention can be significantly improved by using an electron conductive material, for example, an acceptor, in the moiré prevention layer 45.

The same binder resins as those for use in the charge blocking layer 43 can be used for the moiré prevention layer 45. Considering that the photosensitive layer 38 (the charge generating layer 35 and the charge transport layer 37) is provided on the moiré prevention layer 45, it is desired to use a binder resin which is insoluble in the liquid of application for use in the photosensitive layer 38.

As the binder resin, thermocuring resins are suitably used. Especially, a mixture of an alkyd resin and a melamine resin is most suitably used. The mixing ratio of alkyd resin to melamine resin in weight is a significant factor for determining the structure and the characteristics of the moiré prevention layer 45 and preferably from 5/5 to 8/2. A ratio of the melamine resin that is too great is not preferred because the volume contraction tends to be large, which may lead to the occurrence of layer application deficiency and the rise of the residual voltage. A ratio of the alkyd resin that is too great is not preferred because the bulk resistance is excessively low, which may lead to deterioration of the background fouling despite of the effect on the reduction of the residual voltage of an image bearing member.

In the moiré prevention layer 45, the volume ratio of the metal oxide to the binder resin has a significant importance. It is desired that the volume ratio of the metal oxide to the binder resin is from 1/1 to 3/1. When the ratio is too low, not only does the moiré prevention function tend to deteriorate, but also the rise of the residual voltage tends to increase during repetitive use. To the contrary, when the ratio is too high, the binding ability of the binder resin tends to be inferior and the surface property of the layer tends to deteriorate, which may have an adverse impact on the property of the photosensitive layer 38, which is provided on or above the moiré prevention layer 45. This impact can be significant when the photosensitive layer 38 is a layered type and a thin layer, for example, the charge generating layer 45, is formed therein. When the volume ratio is too high, the binder resin may not completely cover the surface of the metal oxide. Thereby, the metal oxide and a charge generating material directly contact each other, which leads to the increase of the probability of production of thermocarriers, resulting in an adverse impact on the anti-background fouling property.

Further, by using two kinds of metal oxides having different particle diameters in the moiré prevention layer 45, it is possible to improve the covering ability to the substrate 31 and restrain the production of moiré images. Also, pinholes, which cause the production of abnormal images, can be removed thereby. The ratio (D2/D1) of the average particle diameters of the two metal oxides, i.e., a metal oxide T1 having a large particle diameter D1 and a metal oxide T2 having a small diameter D2, is desired to satisfy the following relationship:  $0.2 < D2/D1 \leq 0.5$ . When the particle diameter ratio is too small, the activity at the surface of the metal oxides increases, which may lead to significant deterioration of the electrostatic stability of the image bearing member containing the metal oxides. In addition, when the particle diameter ratio is too large, the ability to cover the substrate 31 deteriorates so that production of moiré and/or abnormal images may not be restrained. The average particle diameter is obtained from the particle diameter distribution obtained when a strong dispersion is performed in an aqueous medium.

In addition, the average particled diameter D2 of the metal oxide T2 has a significant importance and D2 preferably satisfies the following relationship:  $0.05 \mu\text{m} < D2 < 0.20 \mu\text{m}$ . When D2 is too small, the covering ability deteriorates, which may cause moiré images. To the contrary, when D2 is too large, the filling ratio of the metal oxides in the moiré prevention layer 45 is decreased so that the effect of restraining the background fouling is not sufficient.

Also, the mixing ratio (by weight) of the two metal oxides 10 is another significant factor and it is preferred to satisfy the following relationship:  $0.2 \leq T2/(T1+T2) \leq 0.8$ . When the ratio of T2/(T1+T2) is too small, the filling ratio of the metal oxides is not greatly large so that the effect of restraining the background fouling is not sufficient. When the ratio of T2/(T1+T2) is too large, the covering ability deteriorates, which 15 may cause moiré images.

In addition, the thickness of the moiré prevention layer 45 is from 1 to 10  $\mu\text{m}$  and preferably from 2 to 5  $\mu\text{m}$ . When the 20 layer thickness is too low, the effect is not sufficient. When the layer thickness is too high, the residual voltage rises, which is not preferred.

The metal oxides are dispersed with a solvent and a binder resin by a known method using, for example, a ball mill, a sand mill and an attritor. The liquid dispersion is applied to a 25 substrate by a known method, for example, a blade coating, a dip coating, a spray coating, a bead coating and a nozzle coating with optional agents, solvents, additives, curing promotion agents, etc., desired for curing (cross linking). Subsequent to coating, the layer is dried or cured by treatment of 30 drying, heating, light, etc.

Next, the photosensitive layer 38 is described. The photosensitive layer 38 is formed of the charge generating layer 35 containing an organic charge generating material as the charge generating material and the charge transport layer 37 35 containing a charge transport material as its main component.

The charge generating layer 35 is formed by dispersing the organic charge generating material with an optional binder resin in a suitable solvent by using a ball mill, an attritor, a sand mill and/or supersonic and applying the liquid dispersion 40 to the intermediate layer 39 followed by drying.

Specific examples of the optional binder resins for use in the charge generating layer 35 include polyamides, polyurethanes, epoxy resins, polyketones, polycarbonates, silicone resins, acrylic resins, polyvinyl butyral, polyvinyl formals, 45 polyvinyl ketones, polystyrenes, polysulfones, poly-N-vinyl carbazoles, polyacrylamides, polyvinyl benzals, polyesters, phenoxy resins, copolymers of vinylchloride-vinyl acetates, polyvinyl acetates, polyphenylene oxides, polyvinyl pyridines, cellulose-based resins, caseine, polyvinyl alcohols, and polyvinyl pyrrolidones. The content of the optional binder resin is from 0 to 500 parts by weight and preferably from 10 to 300 parts by weight based on 100 parts by weight of a charge generating material.

Specific examples of the solvents include isopropanol, 55 acetone, methylethylketone, cyclohexane, tetrahydrofuran, dioxane, ethylcellosolve, ethyl acetate, methyl acetate, dichloromethane, dichloroethane, monochlorobenzene, cyclohexane, toluene, xylene, and ligroin. Usable methods of coating a liquid of application are, for example, a dip coating method, a spray coating method, a bead coating method, a nozzle coating method, a spinner coating method and a ring coating method. The layer thickness of the charge generating layer 35 is from about 0.01 to about 5  $\mu\text{m}$  and preferably from 0.1 to 2  $\mu\text{m}$ .

60 In addition, it is preferred that the transmission factor of the charge generating layer 35 at the wavelength of writing light is from 10 to 25%. When the charge generating layer 35 does

not have a light transmission property for the writing light sufficiently, the writing light does not sufficiently reach the intermediate layer 39. When the transmission factor is too large, the optical extinction at the time of forming a latent electrostatic image is not sufficient. Therefore, there is a suitable range of the transmission factor as mentioned above.

As the charge generating material, organic charge generating materials can be used.

Specific examples thereof include phthalocyanine based pigments, for example, metal phthalocyanine and non-metal phthalocyanine, azulenium salt pigments, methine squaric acid pigments, azo pigments having carbazole skeleton, azo pigments having triphenylamine skeleton, azo pigments having dibenzothiophene skeleton, azo pigments having fluorenone skeleton, azo pigments having oxadiazole skeleton, azo pigments having bisstilbene skeleton, azo pigments having distyryl oxadiazole skeleton, azo pigments having distyryl carbazole skeleton, perylene based pigments, anthraquinone based or polycyclic quinone based pigments, quinone imine pigments, diphenyl methane based pigments, triphenyl methane based pigments, benzoquinone based pigments, naphthoquinone based pigments, cyanine based pigments, azomethine based pigments, indigoid based pigments, and bisbenzimidazole pigments. These charge generating materials can be used alone or in combination.

Among these, the azo pigments represented by the following chemical structure 1 are effectively used as the charge generating material of the present invention. Especially, asymmetric azo pigments having  $Cp_1$  and  $Cp_2$  which are different from each other are effectively used because the asymmetric azo pigments have a large carrier generation efficiency.



In the chemical structure 1,  $Cp_1$  and  $Cp_2$  individually represent coupler residue groups.  $R_{201}$  and  $R_{202}$  independently denote one of hydrogen atom, a halogen atom, an alkyl group, an alkoxy group, and cyano group.  $Cp_1$  and  $Cp_2$  are represented by the following chemical structure 2:



In the chemical structure II,  $R_{203}$  represents one of hydrogen atom, an alkyl group, for example, methyl group and

ethyl group, and aryl group, for example, phenyl group.  $R_{204}$ ,  $R_{205}$ ,  $R_{206}$ ,  $R_{207}$  and  $R_{208}$  independently represent one of hydrogen atom, nitro group, cyano group, a halogen atom, for example, fluorine atom, chlorine atom, bromium atom and iodine atom, an alkyl group, for example, methyl group and ethyl group, an alkoxy group, for example, methoxy group and ethoxy group, dialkyl amino group and hydroxyl group.  $Z$  represents an atom group forming a substituted or non-substituted aromatic carbon ring or a substituted or non-substituted aromatic heterocyclic ring.

Titanyl phthalocyanines can be effectively used as the charge generating material of the present invention. Among these, titanyl phthalocyanine having a crystal form having a  $CuK\alpha$  X ray diffraction spectrum having a wavelength of 1.542 Å such that a maximum diffraction peak is observed at a Bragg (20) angle of  $27.2 \pm 0.2^\circ$ , main peaks at a Bragg (20) angle of  $9.4 \pm 0.2^\circ$ ,  $9.6 \pm 0.2^\circ$ , and  $24.0 \pm 0.2^\circ$ , and a peak at a Bragg (20) angle of  $7.3 \pm 0.2^\circ$  as the lowest angle diffraction peak, and having no peak between the peak of  $9.4 \pm 0.2^\circ$  peak and the peak of  $7.3 \pm 0.2^\circ$  and no peak at  $26.3^\circ$  efficiently produces carriers and can be used as the charge generating material of the present invention. The Bragg  $\theta$  ( $^\circ$ ) is a half angle of the angle of 20 formed between the incident X ray and the diffracted Xray to the crystal.

With regard to the organic charge generating material contained in the image bearing member for use in the present invention, the effect thereof appears by making the particle size thereof small. The average particle diameter is preferably not greater than 0.25  $\mu m$  and more preferably not greater than 0.2  $\mu m$ . The size of the charge generating material contained in the photosensitive layer 38 can be controlled by removing coarse particles having a particle diameter not less than 0.25  $\mu m$  after dispersion of the charge generating material.

The average particle diameter means the volume average particle diameter and is measured using an ultracentrifugal automatic particle size measuring device (CAPA-700, manufactured by Horiba Ltd.). The volume average particle diameter is calculated as the particle diameter (the median particle diameter) corresponding to the cumulative 50% particle diameter. However, since this method has a possibility that a minute quantity of coarse particles is not detected, it is desired to directly observe charge generating powder or a liquid dispersion thereof with an electron microscope to obtain an accurate size.

As a result of the study on the minute defect based on further observation of the liquid dispersion, the phenomenon is recognized as follows. In a typical method of measuring the average particle size, when particles having an extremely large size are present in an amount of not less than a couple percent, these particles can be detected. But the measuring device cannot detect large particles present in a small amount, for example, about not greater than 1% based on the total amount. Consequently, such large particles cannot be detected by simply measuring the average particle size, which makes understanding the minute defect mentioned above difficult.

FIGS. 6 and 7 are photographs illustrating the states of two kinds of a liquid dispersion formed under the same dispersion conditions except for the dispersion time. FIG. 6 is a photograph of a liquid dispersion formed in a short dispersion time. Black particles, which represent remaining coarse particles, are observed in the photograph of FIG. 6 as compared with the photograph of a liquid dispersion of FIG. 7, which is formed in a relatively long dispersion time.

The average particle diameter and the particle size distribution of these two kinds of liquid dispersions are measured by a known method using a marketed ultracentrifugal auto-

matic particle size measuring device (CAPA-700, manufactured by Horiba Ltd.). The results are shown in FIG. 8. A in FIG. 8 corresponds to the particle diameter and the particle size of the liquid dispersions of FIG. 6 and B in FIG. 8 corresponds to the particle diameter and the particle size of the liquid dispersions of FIG. 7. When both are compared, there is actually no difference with regard to the particle size distribution. The average particle diameters of A and B are 0.29  $\mu\text{m}$  and 0.28  $\mu\text{m}$ , respectively. Considering the measuring error, it is difficult to determine that there is a difference between A and B.

Therefore, it is difficult to detect a minute quantity of large particles remaining in a liquid dispersion simply by a known method for measuring an average particle size. Therefore, it is understood that such a method is not sufficient to obtain particles suitable for the current negative-positive development having a high definition. Such large particles existing in a minute quantity can be recognized only when the liquid of application is observed with a microscope.

Next, a method of removing coarse particles after dispersing organic charge generating material is described.

In the method, after preparing a liquid dispersion in which particles are made to be as fine as possible, the liquid dispersion is filtered with a suitable filter.

A liquid dispersion can be prepared by a known method. The organic charge generating material and an optional binder resin are dispersed in a suitable solvent with a ball mill, an attritor, a sand mill, a bead mill or supersonic. The binder resin can be selected based on the electrostatic characteristics of an image bearing member and the solvent can be selected based on the wettability to a pigment and the dispersability thereof.

In this method, it is possible to remove large particles present in a minute amount which cannot be observed or detected by particle size measurement. In addition, the method is also extremely effective in light of obtaining a sharp particle size distribution. Specifically, the liquid dispersion prepared as described above is subject to filtration with a filter having an effective mesh size of not greater than 5  $\mu\text{m}$  and preferably not greater than 3  $\mu\text{m}$ . A liquid dispersion containing only organic charge generating material having a small particle size, i.e., not greater than 0.25  $\mu\text{m}$  and preferably not greater than 0.2  $\mu\text{m}$ , can be prepared by this method. When an image bearing member using this titanyl phthalocyanine is installed in an image forming apparatus, the effects of the present invention is further significant.

A particle size of the filtered liquid dispersion that is too large or a particle size distribution thereof that is too broad may increase the loss by the filtration and cause clogging during the filtration, which leads to making the further filtration impossible. Therefore, with regard to the liquid dispersion before filtration, it is desired to perform the dispersion by which the average particle size is not greater than 0.3  $\mu\text{m}$  with a standard deviation of 0.2  $\mu\text{m}$ . When the average particle size is too large, the loss of the filtration tends to increase and when the standard deviation is too large, the filtration may take long.

The charge generating material for use in the present invention has an extremely strong hydrogen bond force, which is characteristic to a charge generating material having a high sensitivity. Thereby, the interaction among dispersed pigment particles is extremely strong. Consequently, charge generating material particles dispersed by a dispersion device are highly likely to reagglomerate by dilution so that, as described above, such agglomerated materials can be removed by using a filter having a mesh not larger than a particular size. Since the liquid dispersion is in a thixotropy

state, particles having a particle diameter smaller than that of the effective mesh diameter of the filter are also removed. In addition, it is possible to change structural viscosity liquid to a state close to Newtonian by filtration. When coarse particles of the charge generating material are removed as described above, the effect of the present invention can be extremely improved.

Selection of the filters for filtering a liquid dispersion depends on the size of coarse particles to be removed. According to the study by the inventors of the present invention, it is found that coarse particles having a size of about 3  $\mu\text{m}$  have an adverse effect on images when such coarse particles exist in an image bearing member for use in an image forming apparatus performing image formation with a definition of about 600 dpi. Therefore, a filter used preferably has an effective mesh size not greater than 5  $\mu\text{m}$  and more preferably not greater than 3  $\mu\text{m}$ . With regard to the effective mesh size, it is more effective to remove large particles with a small effective mesh size. But when the effective mesh size is too small, the desired pigment particles may be filtered as well. Therefore, there is a suitable effective mesh size. In addition, when the effective mesh size is too small, there are problems such that it takes a long time to complete filtration, the filter is clogged, and the burden is too heavy when a pump, etc., is used to send liquid. A filter is desirably made of a material insoluble in a solvent for use in a liquid dispersion to be filtered.

The charge transport layer 37 is mainly formed of a charge transport material and can be formed by dissolving or dispersing a charge transport material and a binder resin in a suitable solvent and applying the resultant liquid to the charge generating layer 35 followed by drying. It is possible to add a plastic agent, a leveling agent and an anti-oxidizing agent, if desired.

There are two types of the charge transport materials, which are a positive hole transport material and an electron transport material.

Specific examples of such positive hole transport materials include poly-N-vinyl carbazoles and their derivatives, poly- $\gamma$ -carbazolyl ethyl glutamates and their derivatives, pyrene-formaldehyde condensation compounds and their derivatives, polyvinyl pyrenes, polyvinyl phenanthrenes, polysilanes, oxazole derivatives, oxadiazole derivatives, imidazole derivatives, monoaryl amine derivatives, diaryl amine derivatives, triaryl amine derivatives, stilbene derivatives,  $\alpha$ -phenyl stilbene derivatives, benzidine derivatives, diaryl methane derivatives, triaryl methane derivatives, 9-styryl anthracene derivatives, pyrazoline derivatives, divinyl benzene derivatives, hydrazone derivatives, indene derivatives, butadiene derivatives, pyrene derivatives, bisstilbene derivatives, enamine derivatives and other known materials. These charge transport materials can be used alone or in combination. Specific examples of such electron transport material include electron acceptance materials such as chloranil, bromanil, tetracyanoethylene, tetracyanoquino dimethane, 2,4,5,7-trinitro-9-fluorenone, 2,4,5,7-tetranitro-9-fluorenone, 2,4,5,7-tetrinitroxanthone, 2,4,8-trinitrothioxanthone, 2,6,8-trinitro-4H-indeno[1,2-b]thiophene-4-one, 1,3,7-trinitrodibenzothiophene-5,5-dioxide, and benzoquinone derivatives.

Specific examples of the binder resins include thermal curing resins and thermal plastic resins, for example, polystyrenes, styrene-acrylonitrile copolymers, styrene-butadiene copolymers, styrene-maleic acid anhydride copolymers, polyesters, polyvinyl chlorides, vinyl chloride-vinyl acetate copolymers, polyvinyl acetates, polyvinyl vinylidene, polyarates, phenoxy resins, polycarbonates, cellulose acetate resins, ethyl cellulose resins, polyvinyl butyral, polyvinyl

formals, polyvinyl toluene, poly-N-vinylcarbazols, acrylic resins, silicone resins, epoxy resins, melamine resins, urethane resins, phenol resins, and alkyd resins.

The content of the charge transport material is from 20 to 300 parts by weight and preferably from 40 to 150 parts by weight based on 100 parts by weight of a binder resin. The layer thickness of the charge transport layer 37 is preferably from about 5 to about 100  $\mu\text{m}$ .

Specific examples of the solvents include tetrahydrofuran, dioxane, toluene, dichloromethane, monochlorobenzene, dichloroethane, cyclohexanone, methyl ethyl ketone, and acetone. Among these, to reduce the burden on the environment, the use of a non-halogenated solvent is preferred. Preferred specific examples thereof include cyclic ethers, for example, tetrahydrofuran, dioxolane and dioxane, aromatic hydrocarbons, for example, toluene and xylene and their derivatives.

In an embodiment of the present invention, the charge generating layer 35 and the charge transport layer 37 are formed on the intermediate layer 39. Therefore, it is preferred to select a suitable charge transport material to make writing light reach the intermediate layer 39 in a sufficient amount to suitably perform the writing function (i.e., generation of photocarriers in the intermediate layer 39). In addition, the charge transport layer 37 tends to deteriorate while the charge transport material repetitively absorbs discharging light, which may lead to the rise of the residual voltage to the contrary. In the structure described above, the transmission factor of the charge transport layer 37 for discharging light is not less than 30%, preferably not less than 50% and more preferably not less than 85%.

To obtain such a transmission factor, it is preferred to select a suitable charge transport material for writing light. Among the charge transport materials mentioned above, a charge transport material having triarylamine skeleton is preferred for the image bearing member for use in the present invention because such a charge transport material easily transmits writing light having a wavelength shorter than 450 nm and has a great transferability.

In the present invention, a plasticizing agent and a leveling agent can be contained in the charge transport layer 37, if desired.

Specific examples of the plasticizing agent include dibutyl phthalate and dioctyl phthalate, which are used for typical resins. The addition amount of the plasticizing agent is preferably from 0 to 30 weight % based on a binder resin.

Specific examples of the leveling agent include silicone oils, for example, dimethyl silicone oil and methyl phenyl silicone oil, and polymers or oligomers having perfluoroalkyl groups in its side chain. The addition amount of the leveling agent is preferably from 0 to 1 weight % based on a binder resin.

In the image bearing member for use in the present invention, the protective layer 41 can be optionally provided on or above the photosensitive layer 38 for protection. Recently, computers have been used in everyday life, and therefore, a high-speed printing and the size reduction are demanded for a printer. The protective layer 41 provided on or above a photosensitive layer can improve the durability of an image bearing member. Therefore, the image bearing member for use in the present invention having a high sensitivity can be fully utilized without defects.

There are two types of the protective layers 41 for use in the present invention. One is a layer in which a filler is added in a binder resin. The other is a layer in which a cross linking type binder is used.

The structure in which a filler is added is described first.

Specific examples of the materials for use in the protective layer 41 include ABS resins, ACS resins, olefin-vinyl monomer copolymers, chlorinated polyether, allyl resins, phenolic resins, polyacetals, polyamides, polyamideimides, polyallylsulfones, polybutylenes, polybutyleneterephthalates, polycarbonates, polyarylates, polyethersulfones, polyethylenes, polyethyleneterephthalates, polyimides, acrylic resins, polymethylpentenes, polypropylenes, polyphenyleneoxides, polysulfones, polystyrenes, AS resins, butadiene-styrene copolymers, polyurethanes, polyvinyl chlorides, polyvinylidene chlorides, epoxy resins, etc. Among these resins, polycarbonates and polyarylates are preferably used.

In addition, to improve the anti-abrasion property of the protective layer 41, fluorine-containing resins, for example, polytetrafluoroethylene, and silicone resins can be used therefor. Further, combinations of such resins and an inorganic filler, for example, a titanium oxide, a zinc oxide, a potassium titanate and silica or an organic filler can also be added thereto.

In addition, organic and inorganic fillers can be used in the protective layer 41. Suitable organic fillers include powders of fluorine-containing resins, for example, polytetrafluoroethylene, silicone resin powders, amorphous carbon powders, etc. Specific examples of the inorganic fillers include powders of metals, for example, copper, tin, aluminum and indium; metal oxides, for example, alumina, silica, tin oxide, zinc oxide, titanium oxide, alumina, zirconia, indium oxide, antimony oxide, bismuth oxide, calcium oxide, tin oxide doped with antimony and indium oxide doped with tin; and potassium titanate. In terms of the hardness of a filler, the inorganic fillers and metal oxides are especially preferred. In particular, silica, titanium oxide and alumina are effectively used.

The content of the filler in the protective layer 41 is preferably determined depending on the species of the filler used and the conditions of the electrophotographic process using the resultant image bearing member, but the content of a filler on the uppermost surface side of the protective layer 41 is preferably not less than 5% by weight, more preferably from 10 to 50% by weight, and even more preferably from 10 to 30% by weight, based on the total weight of the solid portion thereof.

The filler included in the protective layer 41 preferably has a volume average particle diameter of from 0.1 to 2  $\mu\text{m}$ , and more preferably from 0.3 to 1  $\mu\text{m}$ . When the average particle diameter is too small, the anti-abrasion property of the resultant image bearing member is not satisfactory. In contrast, when the average particle diameter is too large, the surface property of the resultant protective layer deteriorates or the protective layer 41 is not formed.

The average particle diameter of a filler described in the present invention means a volume average particle diameter unless otherwise specified, and is measured using an ultracentrifugal automatic particle size measuring device (CAPA-500, manufactured by Horiba Ltd.). The volume average particle diameter is calculated as the particle diameter (the median particle diameter) corresponding to the cumulative 50% particle diameter. In addition, it is preferred that the standard deviation of the particle diameter distribution curve of the filler used for the protective layer 41 is not greater than 1  $\mu\text{m}$ . When the standard deviation is too large (i.e., when the filler has too broad particle diameter distribution), the effect of the present invention may not be clearly obtained.

In addition, pH of a filler for use in the present invention has a large effect on the resolution of images produced and the dispersability of the filler. One of the thinkable reasons is as follows. Hydrochloric acid used in the preparation of a filler

(in particular, metal oxides) may remain therein. When the content of the remaining hydrochloric acid is large, the resultant image bearing member tends to produce blurred images. In addition, hydrochloric acid can have an adverse effect on the dispersibility of the filler depending on the remaining amount thereof.

Another reason is that the chargeability of a filler (in particular, a metal oxide) is greatly affected by the pH of the fillers. In general, particles dispersed in a liquid are positively or negatively charged and ions having the reverse polarities agglomerate for electric neutralization. As a result, electric double layers are formed and thereby the particles are stably dispersed in the liquid. As the distance from the particle increases, the potential (i.e., zeta potential) dwindles to zero in an electrically neutral area. As the absolute value of zeta potential increases, the repulsion among particles is strong, meaning that the stability of the dispersion is high. As the absolute value of zeta potential approaches to zero, the particles easily aggregate and are unstable. The zeta potential of a system greatly depends on the pH thereof. The zeta potential becomes zero at a particular pH, meaning that the system has an isoelectric point. Therefore, to stabilize a dispersion system, it is preferred to increase the absolute value of zeta potential by keeping away from the isoelectric point of the system.

It is preferred that the protective layer contains a filler having a pH of 5 or higher at the isoelectric point to prevent production of a blurred image. In other words, a filler having a highly basic property is preferably used in the image bearing member for use in the present invention to increase the prevention effect. A filler having a high basic property at an isoelectric point has a high zeta potential (i.e., the filler is stably dispersed) in an acidic system.

In this invention, the pH of a filler means the pH value of the filler at the isoelectric point, which is determined by the zeta potential of the filler. Zeta potential can be measured by a laser beam potential meter manufactured by Otsuka Electronics Co., Ltd.

In addition, to prevent production of blurred images, a filler having a high electric resistance (i.e., not less than  $1 \times 10^{10}$   $\Omega \cdot \text{cm}$  in resistivity) is preferably used. Further, a filler having a pH not less than 5 and a filler having a dielectric constant not less than 5 can be particularly preferably used. A filler having a dielectric constant not less than 5 and/or a pH not less than 5 can be used alone or in combination. In addition, a filler having a pH not less than 5 and a filler having a pH less than 5, or a filler having a dielectric constant not less than 5 and a filler having a dielectric constant less than 5 can also be used in combination. Among these fillers,  $\alpha$ -alumina, which has a high insulating property, a high thermal stability and an anti-abrasion property due to its hexagonal close-packed structure, is particularly preferred in terms of prevention of formation of blurred images and improvement of anti-abrasion property of the resultant image bearing member.

In the present invention, the specific resistivity of a filler is defined as follows. The specific resistivity of a powder such as a filler fluctuates depending on the filling factor thereof. Therefore, it is desired to measure the specific resistivity under a constant condition. In the present invention, the resistivity is measured by a device having a similar structure to that of the device illustrated in FIG. 1 of JOP H05-113688. The surface area of the electrodes of the device is  $4.0 \text{ cm}^2$ . Before the specific resistivity of a sample powder is measured, a load of 4 kg is applied to one of the electrodes for 1 minute and the amount of the sample powder is adjusted such that the distance between the two electrodes is 4 mm.

The specific resistivity of the sample powder is measured while the sample powder is under pressure of the weight (i.e., 1 kg) of the upper electrode without any other load. The voltage applied to the sample powder is 100V. HIGH RESISTANCE METER (manufactured by Yokogawa Hewlett-Packard Co.) is used to measure the resistivity not less than  $10^6$   $\Omega \cdot \text{cm}$ . A digital multimeter (manufactured by Fluke Corp.) is used to measure the specific resistivity less than  $10^6$   $\Omega \cdot \text{cm}$ . The thus obtained resistivity is defined as the resistivity in embodiments of the present invention.

The dielectric constant of a filler is measured as follows. A cell similar to that used in measuring the specific resistivity is also used to measure the dielectric constant. After a load is applied to a sample powder, the electric capacity of the sample powder is measured using a dielectric loss measuring instrument (manufactured by Ando Electric Co., Ltd.) to determine the dielectric constant of the powder.

These fillers can be subject to surface treatment using at least one surface treatment agent to improve the dispersion property of the fillers in a protective layer. When a filler is poorly dispersed in a protective layer, the following problems occur:

- (1) the residual potential of the resultant image bearing member increases;
- (2) the transparency of the resultant protective layer decreases;
- (3) coating defects occur in the resultant protective layer; and
- (4) the anti-abrasion property of the protective layer deteriorates.

These problems can lead to a large problem restraining the improvement on the quality of images and the duration property of the resultant image bearing member.

Suitable surface treatment agents include known surface treatment agents. Among these, surface treatment agents which can maintain the highly insulative property of a filler used are preferred.

As the surface treatment agents, titanate coupling agents, aluminum coupling agents, zirconium coupling agents, higher fatty acids, combinations of these agents with a silane coupling agent,  $\text{Al}_2\text{O}_3$ ,  $\text{TiO}_2$ ,  $\text{ZrO}_2$ , silicones, aluminum stearate, and the like, can be preferably used to improve the dispersibility of fillers and to prevent formation of blurred images. These materials can be used alone or in combination.

When a filler treated with a silane coupling agent is used, the resultant image bearing member tends to produce blurred images. However, when a silane coupling agent is used in combination with one of the surface treatment agents mentioned above, the effect of the silane coupling is possibly restrained.

The coating weight of a surface treatment agents is preferably from 3 to 30% by weight, and more preferably from 5 to 20% by weight, based on the weight of the treated filler although the weight is determined depending on the average primary particle diameter of the filler.

When the content of the surface treatment agent is too low, the dispersibility of the filler is not improved. In contrast, when the content is too high, the residual potential of the resultant image bearing member significantly increases.

These fillers can be used alone or in combination. With regard to the definition of the content of the surface treatment for a filler, the ratio in weight of the content of a surface treatment agent to the content of the filler is used as mentioned above.

These fillers can be dispersed using a proper dispersion machine. In this case, the fillers are preferably dispersed to an

## 31

extent that aggregated particles of the filler are dissociated to primary particles to improve the transmission factor of the resultant protective layer.

In addition, a charge transport material can be contained in the protective layer 41 to enhance the photo-responsive property and to reduce the residual potential of the resultant image bearing member. The charge transport materials mentioned above for use in the charge transport layer 37 and known charge transport material can also be used for the protective layer 41.

When a low molecular weight charge transport material is used in the protective layer 41, the concentration of the charge transport material may be gradated in the thickness direction of the protective layer 41 with the surface side being thinner. Specifically, it is preferred to reduce the concentration of the charge transport material at the surface portion of the protective layer 41 to improve the anti-abrasion property of the resultant image bearing member. The concentration of the charge transport material means the ratio of the weight of the charge transport material to the total weight of the protective layer 41.

It is extremely advantageous to use a charge transport polymer in the protective layer 41 to improve the durability of the image bearing member.

Furthermore, known charge transport polymers can be used as the binder resin contained in the protective layer 41. The effects of using such a known charge transport polymer are the improvement on anti-abrasion property and the charge transport speed.

Typical application methods are adopted as a method of forming the protective layer 41. The layer thickness of the protective layer 41 is suitably from 0.1 to 10  $\mu\text{m}$ .

Next, the protective layer 41 having a cross linking structure (hereinafter referred to as cross linking type protective layer 41) as the binder structure thereof is described.

With regard to the formation of cross linking structure, three dimensional mesh structure is formed by conducting cross linking reaction using a reactive monomer having multiple cross linking functional groups in one molecular by using optical and/or thermal energy. A binder resin having this mesh structure can have a high anti-abrasion property.

In addition, it is extremely effective to use a monomer partially or entirely having a charge transport function as the reactive monomer mentioned above. By using such a monomer, charge transport portions are formed in the mesh structure, which makes the protective layer 41 properly function. A reactive monomer having triarylamine structure can be effectively used as the monomer having the charge transport function.

The protective layer 41 having such a mesh structure has a high anti-abrasion property but the volume constriction thereof is also large. Therefore, a protective layer that is too thick may cause cracking inside. To solve this problem, the protective layer 41 can have a layered structure formed of a first protective layer of a low molecular dispersion polymer and a second protective layer having a cross linking structure on the first protective layer.

Among cross linking type protective layers 41, the protective layer 41 having a particular structure is especially effectively used.

The protective layer 41 having a particular structure is a protective layer formed by curing a radical polymerizable monomer having at least 3 functional groups which does not have a charge transport structure and a radical polymerizable monomer having a functional group which has a charge transport structure.

## 32

In the cross-linking type protective layer 41, a three-dimensional mesh structure is developed because the protective layer 41 has a cross-linking structure formed by curing a radical polymerizable monomer having at least 3 functional groups. Therefore, the resultant surface layer has an extremely high cross linking density with a high hardness and a high elasticity. Further, the surface is uniform and smooth and obtains a high anti-abrasion property and a high anti-damage property. As described above, it is desired to increase 10 the cross-linking density of the surface, i.e., the number of the cross-linkings per unit area. However, an internal stress increases due to the volume contraction since a number of linkings are formed instantly during curing reaction. This internal stress increases as the layer thickness of the cross-linking type protective layer 41 thickens. Therefore, curing 15 the entire protective layer 41 tends to invite cracking and peeling-off thereof. This phenomenon may not occur initially. But while electrophotography processes, for example, charging, developing, transferring and cleaning are repetitively 20 performed, such cracking and peeling-off tend to occur due to cleaning hazard, thermal fluctuation, etc. over time.

There are the following methods for solving this problem: (1) introducing a polymerizable component in the cross-linking layer and the cross-linking structure, (2) using a radical 25 polymerizable monomer having one or two functional groups in a large amount, and (3) using a monomer having multi-functional groups having a plasticity group. The cured resin layer can be flexible by these methods. However, the cross-linking density is thin in either of these methods and the 30 anti-abrasion property is not significantly improved. To the contrary, the image bearing member for use in the present invention has a cross linking type protective layer 41 having a charge transport structure with a high cross linking density provided on the charge transport layer 37. The cross linking 35 type protective layer 41 has a layer thickness of from 1 to 10  $\mu\text{m}$  in which a three-dimensional structure is developed. Thereby, such cracking and peeling-off do not occur to the image bearing member for use in the present invention and further, an extremely high anti-abrasion property is obtained.

40 When the layer thickness of the cross linking type protective layer 41 is from 2 to 8  $\mu\text{m}$ , the margin against the problem mentioned above is wide. In addition, a material having a high cross-linking density can be selected to further improve the anti-abrasion property.

45 The reason the image bearing member for use in the present invention can restrain the occurrence of cracking and peeling-off is, for example, that the internal stress can be limited because the cross linking type protective layer 41 can be made to be thin. Another reason is that the internal stress in the cross linking type protective layer 41 forming the surface can be relaxed because the photosensitive layer 38 or the charge 50 transport layer 37 is provided under the cross linking type protective layer 41. Thereby, the cross linking type protective layer 41 does not necessarily contain a polymerizable material in a large amount, which leads to the reduction of incompatibility of a cured compound produced during the reaction between the polymerizable material and a radical polymerizable composition (radical polymerizable monomer or a radical polymerizable compound having a charge transport structure). Therefore, scars and toner filming ascribable to the 55 incompatibility hardly occur. Further, when the protective layer 41 is entirely cured upon application of optical energy, light transmission inside the charge transport layer 37 is limited due to the absorption thereof by the charge transport structure. Thereby, there is a possibility that the curing reaction is not fully and uniformly conducted inside the layer. In the cross linking type protective layer 41 for use in the present

invention, the curing reaction uniformly proceeds inside the layer because the layer is thin, i.e., preferably not greater than 10  $\mu\text{m}$ . Therefore, the layer can have a good anti-abrasion property therein as on the surface. Further, the cross linking protective layer **41** is formed of a radical polymerizable compound having a functional group in addition to the radical polymerizable monomer having three functional groups mentioned above. The radical polymerizable compound having a functional group and a charge transport structure is trapped in the cross linking when the radical polymerizable monomer having three functional groups is cured. In contrast, when a low molecular weight charge transport material having no functional group is contained in the cross linking surface layer, the low molecular weight charge transport material precipitates or clouding phenomenon occurs due to its low compatibility. Further, the mechanical strength of the surface of the cross-linking layer deteriorates. On the other hand, when a charge transport material having at least two functional groups is mainly used, the charge transport material is trapped in multiple linkages, which leads to improvement on the cross linking density. However, the charge transport structure is extremely bulky, which greatly distorts the structure of the resultant curing resin. This can be a cause of increasing the internal stress in the cross linking type charge transport layer **41**.

Further, the image bearing member for use in the present invention has good electric characteristics and therefore has a good stability for repetitive use, which leads to high durability and stability. This is because a radical polymerizable compound having a functional group and a charge transport structure is used as a composition material forming the cross linking type protective layer **41** and is fixed between the cross linkings in a pendant manner. As described above, a low molecular weight charge transport material having no functional group precipitates or white turbidity phenomenon occurs, which leads to significant deterioration of the electric characteristics, for example, deterioration of the sensitivity and the rise of the residual voltage, during repetitive use. When a charge transport compound having at least two functional groups is mainly used, the charge transport compound is fixed in the cross linking structure with multiple linkings. Therefore, the structure of the intermediary body (cation radical) during charge transport is not stable, which may lead to deterioration of the sensitivity and the rise of the residual voltage by charge entrapment. The deterioration of the electric characteristics results in the decrease in the image density and an image with thinned lines. Further, the design of a typical image bearing member, which is designed to have a high transportability with less charge entrapment, can be applied to an undercoating layer of the image bearing member for use in the present invention. Therefore, the electric side effects of the cross linking type protective layer **41** having a charge transport structure can be limited to the minimal level.

Further, the cross linking type protective layer **41** for use in the present invention is insoluble in an organic solvent during the formation of the cross linking type protective layer **41**. Therefore, the cross linking type protective layer is highly anti-abrasive. The cross linking type protective layer **41** for use in the present invention is formed by curing a radical polymerizable monomer having three functional groups without having a charge transport structure and a radical polymerizable compound having a functional group and a charge transport structure. A three-dimensional mesh structure is developed in the cross linking type protective layer **41** and therefore the density of the cross-linking structure therein is high. However, depending on the other components (addi-

tives, for example, a monomer having one or two functional groups, a polymerizable binder, an anti-oxidation agent, a leveling agent and a plasticizer and a dissolved component commingling from the layer disposed under the protective layer **41**) other than the polymerizable monomers and the compounds mentioned above and the curing conditions, the cross linking density may locally be thin or a collective body of fine cured cross-linked materials having a high density is formed. In this type of cross linking type protective layer, the linkage force among cured materials is weak and soluble in an organic agent. Further, during repetitive use in the electro-photography process, the cross linking type charge transport layer tends to be locally abraded and the cured material is easily detached into minute pieces. As in the present invention, when the cross linking type protective layer **41** is insoluble in an organic solvent, the proper three-dimensional mesh structure is developed with a high density. In addition, since the chain reaction proceeds in a wide area and the cured material grows and has a high molecular weight, the anti-abrasion property is highly improved.

Next, the material composition of the liquid of application for the cross linking type protective layer related to the present invention is described.

The radical polymerizable monomer having at least 3 functional groups which does not have a charge transport structure related to the present invention contains at least 3 radical polymerizable functional group but does not contain a positive hole structure, for example, triaryl amine, hydrazone, pyrazoline and carbazole nor an electron transport structure, for example, an electron suction aromatic ring having, for example, a condensed polycyclic quinone, a diphenoquinone, cyano group and nitro group. The radical polymerizable functional group is any radical polymerizable group having carbon and carbon double linking. Specific examples of the radical polymerizable functional groups include 1-substituted ethylene functional group and 1,1-substituted ethylene functional group as follows:

A specific example of 1-substituted ethylene functional groups is the functional group represented by the following chemical formula 1:



wherein  $\text{X}_1$  represents an arylene group, for example, a substituted or non-substituted phenylene group and naphthylene group, a substituted or non-substituted alkenylene group,  $-\text{CO}-$ ,  $-\text{COO}-$ ,  $-\text{CON}(\text{R}_{10})-$  ( $\text{R}_{10}$  represents hydrogen atom, an alkyl group, for example, methyl group and ethyl group, an aralkyl group, for example, benzyl group, naphthyl methyl group, and an aryl group, for example, phenethyl group and naphthyl group), or  $-\text{S}-$ ).

Specific examples of such functional groups include vinyl group, styryl group, 2-methyl-1,3-butadienyl group, vinyl carbonyl group, acryloyloxy group, acryloyl amide group, and vinylthio ether group.

A specific example of 1,1-substituted ethylene functional groups is the functional group represented by the following chemical formula 2:



wherein  $\text{Y}$  represents a substituted or non-substituted alkyl group, a substituted or non-substituted aralkyl group, an aryl group, for example, a substituted or non-substituted phenyl group and naphthyl group, a halogen atom, cyano group, nitro group, an alkoxy group, for example, methoxy group and ethoxy group,  $-\text{COOR}_{11}$  ( $\text{R}_{11}$  represents hydrogen atom, an alkyl group, for example, a substituted or non-substituted methyl group or ethyl group, an aralkyl group, for example, a

substituted or non-substituted benzyl group and a substituted or non-substituted phenyl group, an aryl group, for example, a substituted or non-substituted phenyl group and a substituted or non-substituted naphthyl group, or  $-\text{CONR}_{12}\text{R}_{13}$  ( $\text{R}_{12}$  and  $\text{R}_{13}$  independently represent a hydrogen atom, an alkyl group, for example, a substituted or non-substituted methyl group or a substituted or non-substituted ethyl group, an aralkyl group, for example, a substituted or non-substituted benzyl group, a substituted or non-substituted naphthyl methyl group, and a substituted or non-substituted phenethyl group, or an aryl group, for example, a substituted or non-substituted phenyl group and a substituted or non-substituted naphthyl group).  $\text{X}_2$  represents the same substitution group as  $\text{X}_1$  in the chemical formula 1 or an alkylene group and  $\text{d}$  represents 0 or 1. At least one of  $\text{Y}$  and  $\text{X}_2$  is an oxycarbonyl group, cyano group, an alkenylene group or an aromatic ring.

Specific examples of these functional groups include  $\alpha$ -cyanoacryloyloxy group, methacryloyloxy group,  $\alpha$ -cyanoethylene group,  $\alpha$ -cyanoacryloyloxy group,  $\alpha$ -cyanophenylene group and methacryloyl amino group.

Specific examples of the substitution groups further substituted to the substitution groups of  $\text{X}_1$ ,  $\text{X}_2$  and  $\text{Y}$  include halogen atom, nitro group, cyano group, an alkyl group, for example, methyl group and ethyl group, an alkoxy group, for example, methoxy group and ethoxy group, an aryloxy group, for example, phenoxy group, an aryl group, for example, phenyl group and naphthyl group, and an aralkyl group, for example, benzyl group and phenetyl group.

Among these radical polymerizable functional groups, an acryloyloxy group and a methacryloyloxy group are particularly suitable. A compound having at least three acryloyloxy groups can be obtained by performing ester reaction or ester conversion reaction using, for example, a compound having at least three hydroxyl groups therein and an acrylic acid (salt), a halide acrylate and an ester of acrylate. Similarly, a compound having at least three methacryloyloxy groups can be obtained. In addition, the radical polymerizable functional groups in a monomer having at least three radical polymerizable functional groups can be the same or different from each other.

The radical polymerizable monomer having three functional groups without having a charge transport structure are specifically the following compounds but not limited thereto.

Specific examples of the radical polymerizable monomer mentioned above for use in the present invention include trimethylol propane triacrylate (TMPTA), trimethylol propane trimethacrylate, trimethylol propane alkylene modified triacrylate, trimethylol propane ethyleneoxy modified (hereinafter referred to as EO modified) triacrylate, trimethylol propane propyleneoxy modified (hereinafter referred to as PO modified) triacrylate, trimethylol propane caprolactone modified triacrylate, trimethylol propane alkylene modified triacrylate, pentaerythritol triacrylate, pentaerythritol tetraacrylate (PETTA), glycerol triacrylate, glycerol epichlorohydrin modified (hereinafter referred to as ECH modified) triacrylate, glycerol EO modified triacrylate, glycerol PO modified triacrylate, tris(acryloxyethyl)isocyanurate, dipentaerythritol hexacrylate (DPHA), dipentaerythritol caprolactone modified hexacrylate, dipentaerythritol hydroxyl dipentaacrylate, alkylized dipentaerythritol tetracrylate, alkylized dipentaerythritol triacrylate, dimethylol propane tetracrylate (DTMPTA), pentaerythritol ethoxy tetracrylate, phosphoric acid EO modified triacrylate, and 2,2,5,5-tetrahydroxy methyl cyclopentanone tetracrylate. These can be used alone or in combination. In addition, the radical polymerizable monomer having three functional groups without having

a charge transport structure for use in the present invention preferably has a ratio (molecular weight/the number of functional groups) of the molecular weight to the number of functional groups in the monomer is not greater than 250 to 5 form a dense cross linking in the cross linking type protective layer 41. Further, when the ratio (molecular weight/the number of functional groups) is too large, the cross linking type protective layer 41 formed of such a monomer is soft and the anti-abrasion property thereof tends to deteriorate in some degree. Therefore, among the monomers mentioned above, it is not preferred to singly use a monomer having an extremely long modified (EO, PO, caprolactone modified) group. In addition, the content ratio of the radical polymerizable monomer having three functional groups without having a charge transport structure is from 20 to 80% by weight and preferably from 30 to 70% by weight based on the total weight of the cross linking type protective layer 41 having a charge transport structure. When the monomer content ratio is too small, the density of three-dimensional cross linking in the cross linking type protective layer 41 tends to be small. Therefore, the anti-abrasion property thereof is not drastically improved in comparison with the case in which a typical thermal plastic binder resin is used. When the monomer content ratio is too large, the content of a charge transport compound decreases, which may cause the deterioration of the electric characteristics. Desired electric characteristics and anti-abrasion property vary depending on the process and the layer thickness of the cross linking type protective layer 41 for use in the present invention varies. Therefore, it is difficult to jump to any conclusion but considering the balance, the range of from 30 to 70% by weight is preferred.

The radical polymerizable compound having a functional group and a charge transport structure for use in the cross linking type protective layer 41 represents a compound having a radical polymerizable functional group and a positive hole structure, for example, triaryl amine, hydrazone, pyrazoline, and carbazole, or an electron transport structure, for example, condensed polycyclic quinone, diphenoquinone and electron absorbing aromatic ring having cyano group, a nitro group, etc. As the radical polymerizable functional group, the radical polymerizable functional group mentioned in the radical polymerizable monomer mentioned above can be suitably used. Especially, acryloyloxy group and methacryloyloxy group are suitable. In addition, a triaryl amine structure is highly effective as the charge transport structure. Among these, when a compound having the structure represented by the following chemical structures 3 and 4 is used, the electric characteristics, for example, the sensitivity and the residual voltage, are preferably maintained.

[Chemical structure 3]



[Chemical structure 4]



wherein,  $\text{R}_1$  represents hydrogen atom, a halogen atom, an alkyl group, an aralkyl group, an aryl group, a cyano group, a nitro group, an alkoxy group,  $-\text{COOR}_7$ , wherein  $\text{R}_7$  represents hydrogen atom, a substituted or non-substituted alkyl

37

group, a substituted or non-substituted aralkyl group or a substituted or non-substituted aryl group, a halogenated carbonyl group or  $\text{CONR}_8\text{R}_9$ , wherein  $\text{R}_8$  and  $\text{R}_9$  independently represent hydrogen atom, a halogen atom, a substituted or non-substituted alkyl group, a substituted or non-substituted aralkyl group or a substituted or non-substituted aryl group,  $\text{Ar}_1$  and  $\text{Ar}_2$  independently represent a substituted or unsubstituted arylene group,  $\text{Ar}_3$  and  $\text{Ar}_4$  independently represent a substituted or unsubstituted aryl group,  $\text{X}$  represents a single bond, a substituted or non-substituted alkylene group, a substituted or non-substituted cycloalkylene group, a substituted or non-substituted alkylene ether group, oxygen atom, sulfur atom or a vinylene group,  $\text{Z}$  represents a substituted or non-substituted alkylene group, a substituted or non-substituted alkylene ether divalent group or an alkyleneoxy carbonyl divalent group, and  $\text{a}$  represents 0 or 1,  $\text{m}$  and  $\text{n}$  represent an integer of from 0 to 3.

Specific examples of the structure represented by the chemical structures 3 and 4 are as follows.

In the chemical structures 3 and 4, the alkyl group of  $\text{R}_1$  is, for example, methyl group, ethyl group, propyl group, and butyl group. The aryl group thereof is, for example, phenyl group and naphtyl group. The aralkyl group thereof is, for example, benzyl group, phenethyl group, and naphtyl methyl group. The alkoxy group thereof is, for example, methoxy group, ethoxy group and propoxy group. These can be substituted by a halogen atom, nitro group, cyano group, an alkyl group, for example, methyl group and ethyl group, an alkoxy group, for example, methoxy group and ethoxy group, an aryloxy group, for example, phenoxy group, an aryl group, for example, phenyl group and naphtyl group, and an aralkyl group, for example, benzyl group and phenethyl group.

Among these substitution groups of  $\text{R}_1$ , hydrogen atom and methyl group are especially preferred.

$\text{Ar}_3$  and  $\text{Ar}_4$  represent a substituted or non-substituted aryl group. Specific examples thereof include condensed polycyclic hydrocarbon groups, non-condensed ring hydrocarbon groups and heterocyclic groups.

The condensed polycyclic hydrocarbon group preferably forms a ring by 18 or less carbon atoms. Specific examples thereof include pentanyl group, indenyl group, naphtyl group, azulenyl group, heptalenyl group, biphenylenyl group, as-indacenyl group, s-indacenyl group, fluorenyl group, acenaphthylenyl group, pleiadetyl group, acenaphtentenyl group, phenalenyl group, phenanthryl group, anthryl group, fluorantennyl group, acephenantrirenyl group, aceantrirenyl group, triphenyl group, pyrenyl group, chrysanyl group, and naphthacenyl group.

Specific examples of the non-condensed ring hydrocarbon group include a single-valent group of monocyclic hydrocarbon compounds, for example, benzene, diphenyl ether, polyethylene diphenyl ether, diphenylthio ether and diphenylsulfone, a single-valent group of non-condensed polycyclic hydrocarbon compounds, for example, biphenyl, polyphenyl, diphenyl alkane, diphenyl alkene, diphenyl alkyne, triphenyl methane, distyryl benzene, 1,1-diphenyl cycloalkane, polyphenyl alkane and polyphenyl alkene or a single-valent group of ring aggregated hydrocarbon compounds, for example, 9,9-diphenyl fluorene.

Specific examples of the heterocyclic group include a single-valent group of, for example, carbazol, dibenzofuran, dibenzothiophene, oxadiazole, and thiadiazole.

The substituted or non-substituted aryl groups represented by  $\text{Ar}_3$  and  $\text{Ar}_4$  can have the following substitution groups.

- (1) a halogen atom, cyano group, and nitro group;
- (2) a straight chained or branch chained alkyl group having 1 to 12 carbon atoms, preferably 1 to 8 carbon atoms and

38

more preferably 1 to 4 carbon atoms. These alkyl groups can have fluorine atom, hydroxyl group, cyano group, an alkoxy group having 1 to 4 carbon atoms, phenyl group or a phenyl group substituted by a halogen atom, an alkyl group having 1 to 4 carbon atoms or an alkoxy group having 1 to 4 carbon atoms. Specific examples thereof include methyl group, ethyl group, n-butyl group, i-propyl group, t-butyl group, s-butyl group, n-propyl group, trifluoromethyl group, 2-hydroxy ethyl group, 2-ethoxyethyl group, 2-cyanoethyl group, 2-methoxyethyl group, benzyl group, 4-chlorobenzyl group, 4-methyl benzyl group and 4-phenyl benzyl group;

- (3) an alkoxy group ( $—\text{OR}_2$ ), wherein  $\text{R}_2$  represents the alkyl group defined in (2). Specific examples thereof include methoxy group, ethoxy group, n-propoxy group, i-propoxy group, t-butoxy group, n-butoxy group, s-butoxy group, i-butoxy group, 2-hydroxyethoxy group, benzyl oxy group and trifluoromethoxy group;
- (4) an aryloxy group: As an aryl group, for example, phenyl group and naphtyl group can be included. These can contain an alkoxy group having 1 to 4 carbon atoms, an alkyl group having 1 to 4 carbon atoms or a halogen atom as a substitution group. Specific examples thereof include phenoxy group, 1-naphtyloxy group, 2-naphtyloxy group, 4-methoxyphenoxy group, and 4-methylphenoxy group;
- (5) an alkyl mercapto group or an aryl mercapto group: Specific examples thereof include methylthio group, ethylthio group, phenylthio group, and p-methylphenylthio group;
- (6)

[Chemical structure 6]



In the chemical structure 6,  $\text{R}_3$  and  $\text{R}_4$  independently represent hydrogen atom, the alkyl group defined in (2), or an aryl group. Specific examples of the aryl group include phenyl group, biphenyl group, or naphtyl group. These can contain an alkoxy group having 1 to 4 carbon atoms, an alkyl group having 1 to 4 carbon atoms or a halogen group.  $\text{R}_3$  and  $\text{R}_4$  can form a ring together. Specific examples thereof include amino group, diethyl amino group, N-methyl-N-phenyl amino group, N,N-diphenyl amino group, N,N-di(tolyl) amino group, dibenzyl amino group, piperidino group, morpholino group, and pyrrolidino group;

- (7) an alkylene dioxy group or an alkylene dithio group, for example, methylene dioxy group and methylene dithio group; and
- (8) a substituted or non-substituted styryl group, a substituted or non-substituted  $\beta$ -phenyl styryl group, diphenyl aminophenyl group, ditolyl aminophenyl group, etc.

The arylene group represented by  $\text{Ar}_1$  and  $\text{Ar}_2$  are divalent groups derived from the aryl group represented by  $\text{Ar}_3$  and  $\text{Ar}_4$ .

$\text{X}$  represents a substituted or non-substituted alkylene group, a substituted or non-substituted cycloalkylene group, a substituted or non-substituted alkylene ether group, oxygen atom, sulfur atom or vinylene group.

Specific examples of the substituted or non-substituted alkylene group include a straight chained or branch chained alkylene group having 1 to 12 carbon atoms, preferably 1 to 8 carbon atoms and more preferably from 1 to 4 carbon atoms. These alkylene groups can further have fluorine atom, hydroxyl group, cyano group, an alkoxy group having 1 to 4

carbon atoms, phenyl group or a phenyl group substituted by a halogen atom, an alkyl group having 1 to 4 carbon atoms or an alkoxy group having 1 to 4 carbon atoms. Specific examples thereof include methylene group, ethylene group, n-butylene group, i-propylene group, t-butylene group, s-butylene group, n-propylene group, trifluoromethylene group,

Specific examples of the substituted or non-substituted divalent alkylene ether group include the same as the alkylen ether group described for X.

A specific example of the divalent alkyleneoxy carbonyl group includes a divalent caprolactone modified group.

In the present invention, the radical polymerizable compound having a functional group with a charge transport structure is more preferably the compound represented by the following chemical structure 5.

[Chemical structure 5]



2-hydroxy ethylene group, 2-ethoxyethylene group, 2-cyanoethylene group, 2-methoxyethylene group, benzylidene group, phenyl ethylene group, 4-chlorophenyl ethylene group, 4-methylphenyl ethylene group, and 4-biphenyl ethylene group.

Specific examples of the substituted or non-substituted cycloalkylene groups include cyclic alkylene group having 5 to 7 carbon atoms. These cyclic alkylene groups can have fluorin atom, a hydroxyl group, an alkyl group having 1 to 4 carbon atoms, and an alkoxy group having 1 to 4 carbon atoms. Specific examples thereof include cyclohexylidene group, cyclohexylene group, and 3,3-dimethyl cyclohexylidene group.

Specific examples of the substituted or non-substituted alkylene ether group include ethyleneoxy group, propyleneoxy group, ethylene glycol, propylene glycol, diethylene glycol, tetraethylene glycol, tripropylene glycol, etc. Alkylenes groups of the alkylene ether groups can have a substitution group, for example, hydroxyl group, methyl group, and ethyl group.

The vinylene groups represented by X are, for example, substitution groups represented by the following chemical structures 7 and 8:

[Chemical structure 7]



[Chemical structure 8]



In the chemical structures 7 and 8, R<sub>5</sub> independently represent hydrogen atom, an alkyl group (the same as the alkyl groups defined in (2)), an aryl group (the same as the aryl groups of Ar<sub>3</sub> and Ar<sub>4</sub> mentioned above), a represents 1 or 2 and b represents an integer of from 1 to 3.

Z represents a substituted or non-substituted alkylene group, a substituted or non-substituted divalent alkylene ether group or a divalent alkyleneoxy carbonyl group.

Specific examples of the substituted or non-substituted alkylene group include the same as the alkylen group described for X.

20 In the chemical structure 5, u, r, p, q independently represent 0 or 1. s and t independently represent an integer of from 0 to 3. Ra represents hydrogen atom or methyl group. Each of Rb and Rc independently represents an alkyl group having 1 to 6 carbon atoms. Za represents methylene group, ethylene group, —CH<sub>2</sub>CH<sub>2</sub>O—, —CHCH<sub>2</sub>CH<sub>2</sub>O—, or —C<sub>6</sub>H<sub>5</sub>CH<sub>2</sub>CH<sub>2</sub>—.

25 Among the compounds represented by Chemical structure illustrated above, the compounds having a methyl group or an ethyl group as a substitution group of each of Rb and Rc are preferred.

30 The radical polymerizable compound for use in the present invention having a functional group with a charge transport structure represented by the chemical structures 3, 4 and especially 5 is polymerized in such a manner that the double linkage of C and C is open to both ends. Therefore, the radical polymerizable compound is not present at the end but in the chained polymer. In a polymer in which a cross linking chain is formed with a radical polymerizable monomer having at 35 least 3 functional groups, the radical polymerizable compound is present in the main chains of the polymer and in a cross linking chain. There are two kinds of cross linking chains. One is referred to as inter-molecule cross linking, in which the cross linking chain is formed between a polymer and another polymer. The other is referred to as internal cross linking, in which the cross linking chain is formed between a portion in the main chain present in a polymer formed in a folded state and another portion deriving from the monomer which is polymerized at a position remote from that portion in 40 the main chain. Whether the radical polymerizable monomer having at least 3 functional groups is present in a main chain or in a cross linking chain, the triaryl amine structure suspending from the chain portion has at least three aryl groups disposed in the radial directions from the nitrogen atom 45 therein. Such a triaryl amine structure is bulky and does not directly bind with the chain portion but suspends from the chain portion via a carbonyl group, etc. That is, the triaryl amine structure is stereoscopically fixed in the polymer in a flexible state. Therefore, these triaryl amine structures can be 50 adjacent to each other with a moderate space in a polymer. Therefore, the structural distortion in a molecule is slight. In addition, when the structure is used in the surface layer of an image bearing member, it can be deduced that the internal 55 molecular structure can have a structure in which there are relatively few disconnections in the charge transport route.

60 Below are specific examples of the radical polymerizable compound for use in the present invention having a functional

**41**

group with a charge transport structure. But the radical polymerizable compounds are not limited thereto.

**42**

-continued

No. 5



No. 1

5

10

15

20



No. 2

25

30

35

No. 3

40

45

50

No. 4

55

60

65

**42**

-continued

No. 5



No. 6



No. 7



No. 8

43

-continued



$$\begin{array}{c}
 \text{CH}=\text{CH}_2 \\
 | \\
 \text{O}=\text{C} \\
 | \\
 \text{O} \\
 | \\
 \text{C}_6\text{H}_4 \\
 | \\
 \text{N} \\
 | \\
 \text{C}_6\text{H}_4
 \end{array}$$

CC(=O)Oc1ccc(cc1)N(c2ccccc2Cl)c3ccccc3

No. 9

5

10

No. 10

20

25

No. 11

40

45

No. 12

55

60

65

44

-continued

No. 13



45

-continued



No. 16

5

10

20

46

-continued



No. 19

№. 17 25

30

35

40

45

No. 20



No. 18 50

22

60

65

No. 21



**47**

-continued



No. 22

5

10

15

20

No. 23

25

30

35

40

45

No. 24

50

55

60

65

**48**

-continued

No. 25



No. 26



No. 27



49

-continued



No. 28

5

10

No. 29

20

25

30

No. 30

40

45

50

No. 31

60

65

50

-continued



No. 32

No. 33



No. 34



No. 35





53

-continued



54

-continued

No. 43

5



No. 44

25



30

35

40

45

No. 47



No. 48

No. 45

50

55

60

65



No. 46

**55****56**

57

-continued



No. 55

5

10

15

20

25

No. 56

30

35

40

No. 57

45

50

55

60

65

58

-continued

No. 58



No. 59



59

60

-continued



No. 61

5

10

20

25

30

35

40

45

No. 63

50

55

60

65

No. 64

-continued



30



No. 65

CH<sub>3</sub>



No. 63

50

55

60

65

**61**

-continued



No. 67

5

10

15

20

25

30

35

40

**62**

-continued



No. 69

5



10



15



20



25

30

35

40

No. 68

45



50



55



60



65

No. 70

**63****64**

No. 73



No. 71

5

10

15

20

No. 72

30

35

40

No. 73

50

55

60

No. 74

No. 75

No. 76

**65**

-continued



No. 77

5

10

15

20



No. 78

25

30

35

40

45

**66**

-continued



No. 80

No. 79

50

55

60

65



No. 81



No. 82

**67**

-continued



No. 83

5

10

15

20

No. 84

25

30

35

40

45

No. 85

50

55

60

65

**68**

-continued

No. 86



No. 84

25

30

35

40

45

No. 85

50

55

60

65

No. 87



No. 88



69

-continued



No. 89

5

10

20

25

35

40

70

-continued



No. 91

30

35

40

No. 92

No. 90

45

50

55

60



**71**

-continued



No. 93

5

10

15

20

25

30

35

40

**72**

-continued

No. 95



No. 93

5

10

15

20

25

30

35

40

No. 94

45

50

55

60

65



No. 96

73

-continued



5

10

15

20

25

30

35

40



No. 98

45

50

55

60

65

74

-continued

No. 99



No. 97

5

10

15

20

25

30

35

40

No. 100





77

-continued



No. 105

5

10

15

20

25

30

35

40

78

-continued

No. 107



No. 106

45

50

55

60

65

No. 108



79

-continued



80

-continued

No. 109



No. 111

No. 112

No. 113

No. 110



81

-continued



82

-continued

No. 117



No. 114

5

10

20

30

40

N 116

45

50

55

60

No. 118



45

55

60

**83**

-continued



5

10

20

25

30

**84**

-continued

No. 121



35

40



No. 120

45

50

55

60

65



No. 122

**85****86**

No. 124



No. 126



87

-continued



No. 127

5

10

20

25

30

40

No. 129

50

55

60

88

-continued



No. 130

No. 131

No. 132

89

90

-continued

No. 133



5

No. 134



20

30

35

No. 135



40

50

No. 136



55

60

65

-continued

No. 137



No. 138



No. 139



**91**

-continued

No. 140

**92**

-continued

No. 142



No. 141 45



No. 144



No. 145

93

-continued



-continued



The radical polymerizable compound for use in the present invention having a functional group with a charge transport structure imparts a charge transport function to the cross linking type protective layer **41**. The content of the cross

No. 156

linking type protective layer **41** is from 20 to 80% by weight, and preferably from 30 to 70% by weight. When the content is too small, the charge transport function of the cross linking type protective layer **41** is not maintained, which may lead to the deterioration of the electric characteristics, for example, the decrease in the sensitivity and the rise in the residual voltage, during repetitive use. When the content is too large, the content of the radical polymerizable monomer having at least three functional groups without a charge transport structure decreases. That is, the cross linking density decreases, resulting in the shortage of the anti-abrasion property. Desired electric characteristics and anti-abrasion property vary depending on the process, which affects the layer thickness of the cross linking type protective layer **41** of the image bearing member. Therefore, it is difficult to jump to any conclusion but considering the balance of both characteristics and property, the addition amount is most preferably from 30 to 70% by weight.

The cross linking type protective layer **41** forming the image bearing member for use in the present invention is formed by curing at least a radical polymerizable monomer having at least three functional groups which does not have a charge transport structure and a radical polymerizable compound having one functional group which has a charge transport structure. In addition to this, a radical polymerizable monomer having one or two functional groups, functional monomers, and a radical polymerizable oligomer can be used to provide functions, for example, adjusting the viscosity upon coating, relaxing the stress in the cross linking type protective layer **41**, decreasing the surface energy, and reducing the friction index, etc. Any known radical polymerizable monomers and oligomers can be used.

Specific examples of the radical polymerizable monomer having one functional group include monomers of 2-ethylhexyl acrylate, 2-hydroxyethyl acrylate, 2-hydroxypropyl acrylate, tetrahydrofurfuryl acrylate, 2-ethylhexyl carbitol acrylate, 3-methoxybutyl acrylate, benzyl acrylate, cyclohexyl acrylate, isoamyl acrylate, isobutyl acrylate, methoxy triethylene glycol acrylate, phenoxy tetraethylene glycol acrylate, cetyl acrylate, isostearyl acrylate, stearyl acrylate, and styrene.

Specific examples of the radical polymerizable monomer having two functional groups include 1,3-butandiol diacrylate, 1,4-butane diol diacrylate, 1,4-butane diol dimethacrylate, 1,6-hexane diol diacrylate, 1,6-hexane diol dimethacrylate, diethylene glycol diacrylate, neopentyl glycol diacrylate, bisphenol A-EO modified diacrylate, bisphenol F-EO modified diacrylate and neopentyl glycol diacrylate.

Specific examples of the functional monomer include monomers in which a fluorine atom of, for example, octafluoro pentyl acrylate, 2-perfluoroctyl ethyl acrylate, 2-perfluorooctyl ethyl methacrylate and 2-perfluoroisononyl ethyl acrylate is substituted, and vinyl monomers, acrylates and methacrylates having polysiloxane groups, for example, acryloyl polydimethyl siloxane ethyl, methacryloyl polydimethyl siloxane ethyl, acryloyl polydimethyl siloxane propyl, acryloyl polydimethyl siloxane butyl and diacryloyl polydimethyl siloxane diethyl having 20 to 70 siloxane repeating units set forth in JPPs H05-60503 and H06-45770.

Specific examples of the radical polymerizable oligomer include epoxyacrylate based, urethane acrylate based, and polyester acrylate based oligomers.

When a radical polymerizable monomer and/or a radical polymerizable oligomer having one or two functional groups are contained in a large amount, the three dimensional cross linking density of the cross linking type protective layer **41** substantially decreases, which invites the deterioration of the

anti-abrasion property. Therefore, the content of these monomers and oligomers is not greater than 50 parts by weight and preferably not greater than 30 parts by weight based on 100 parts by weight of the radical polymerizable monomer having at least three functional groups.

The cross linking type protective layer **41** for use in the present invention is formed by curing at least a radical polymerizable monomer having at least three functional groups which does not have a charge transport structure and a radical polymerizable compound having one functional group which has a charge transport structure. A polymerization initiator can be added, if desired, in a liquid of application for the cross linking type protective layer **41** to effectively conduct the curing reaction.

Specific examples of thermal polymerization initiator include peroxide-based initiators, for example, 2,5-dimethylhexane-2,5-dihydroperoxide, dicumyl peroxide, benzoyl peroxide, t-butyl cumyl peroxide, 2,5-dimethyl-2,5-di(peroxybenzoyl)hexyne-3, di-t-butyl peroxide, t-butylhydroperoxide, cumene hydroperoxide, lauroyl peroxide and 2,2-bis(4,4-di-t-butyl peroxy cyclohexy)propane, and azo based initiators, for example, azobis isobutylnitrile, azo-biscyclohexane carbonitrile, azobis methyl isobutyric acid, azobis isobutyl amidine hydrochloride salts, and 4,4'-azobis-4-cyano valeric acid.

Specific examples of photo polymerization initiators include acetophenone based or ketal based photo polymerization initiators, for example, diethoxy acetopenone, 2,2-dimethoxy-1,2-diphenylethane-1-one, 1-hydroxy cyclohexyl phenylketone, 4-(2-hydroxyethoxy)phenyl-(2-hydroxy-2-propyl)ketone, 2-benzyl-2-dimethylamino-1-(4-morpholinophenyl)butanone-1,2-hydroxy-2-methyl-1-phenylpropane-1-one, 2-methyl-2-morpholino(4-methylthiophenyl)propane-1-one, and 1-phenyl-1,2-propane dione-2-(o-ethoxycarbonyl)oxime; benzoin ether based photo polymerization initiators, for example, benzoine, benzoine methyl ether, benzoin ethyl ether, benzoine isobutyl ether and benzoine isopropyl ether; benzophenone based photo polymerization initiators, for example, benzophenone, 4-hydroxy benzophenone, o-benzoyl benzoic acid methyl, 2-benzoyl naphthalene, 4-benzoyl biphenyl, 4-benzoyl phenyl ether, acrylated benzophenone and 1,4-benzoyl benzene; and thioxanthone based photo polymerization initiators, for example, 2-isopropyl thioxanthone, 2-chloro thioxanthone, 2,4-dimethyl thioxanthone, 2,4-diethyl thioxanthone, and 2,4-dichloro thioxanthone.

Other photo polymerization initiators are, for example, ethylanthraquinone, 2,4,6-trimethyl benzoyl diphenyl phosphine oxide, 2,4,6-trimethyl benzoyl phenyl ethoxy phosphine oxide, bis(2,4,6-trimethyl benzoyl)phenyl phosphine oxide, bis(2,4-dimethoxy benzoyl)-2,4,4-trimethyl pentyl phosphine oxide, methylphenyl glyoxy esters, 9,10-phenanthrene, acridine based compounds, triazine based compounds, and imidazole based compounds. In addition, compounds having photo polymerization promotion effect can be used alone or in combination with the photo polymerization initiators mentioned above. Specific examples thereof include triethanol amine, methyl diethanol amine, 4-dimethylamino ethyl benzoate, 4-dimethylamino isoamile benzoate, benzoic acid (2-dimethylamino)ethyl, and 4,4'-dimethylamino benzophenone.

These polymerization initiators can be used alone or in combination. The addition amount of the polymerization initiator is from 0.5 to 40 parts by weight and preferably from 1 to 20 parts by weight based on 100 parts by weight of the total weight of the radical polymerizable compound.

Furthermore, a liquid of application for the cross linking type protective layer **41** can contain additives, for example, various kinds of a plasticizing agent (to relax stress and improve adhesibility), a leveling agent, and a low molecular weight charge transport material which is not radical polymerizable, if desired. Known additives can be used. Specific examples of the plasticizing agent include compounds, for example, dibutyl phthalate and dioctyl phthalate, which are used for typical resins. The addition amount of the plasticizing agent is not greater than 20% by weight and more preferably not greater than 10% by weight based on all the solid portion of the liquid of application. Specific examples of the leveling agent include silicone oils, for example, dimethyl silicone oil, and methylphenyl silicone oil, and polymers or oligomers having a perfluoroalkyl group in its branch chain. The addition amount of the leveling agent is not greater than 3% by weight based on all the solid portion of the liquid of application.

The cross-linking type protective layer **41** for use in the present invention is formed by coating and curing on the charge transport layer **37** a radical polymerizable monomer having three functional groups without having a charge transport structure and a radical polymerizable compound having a functional group and a charge transport structure. When a radical polymerizable monomer contained in a liquid of application is liquid, it is possible to coat the liquid of application in which other components are dissolved. In addition, a liquid of application can be diluted in a suitable solvent before coating, if desired. Specific examples of such solvents include an alcohol based solvent, for example, methanol, ethanol, propanol and butanol; a ketone based solvent, for example, acetone, methyl ethyl ketone, methyl isobutyl ketone, and cycle hexanone; an ester based solvent, for example, ethyl acetate and butyl acetate; an ether based solution, for example, tetrahydrofuran dioxane and propyl ether; a halogen based solvent, for example, dichloromethane, dichloroethane, trichloroethane and chlorobenzene; an aromatic series based solvent, for example, benzene, toluene and xylene; and a cellosolve based solvent, for example, methyl cellosolve, ethyl cellosolve and cellosolve acetate. These solvents can be used alone or in combination. The dilution ratio by these solvents depends on the solubility and the coating method of a composition, and a desired layer thickness. A dip coating method, a spray coating method, a beat coating method, a ring coating method, etc., can be used for application.

In the present invention, subsequent to the application of a liquid of application, the cross-linking type protective layer **41** is cured upon application of external energy, for example, heat, light and radiation ray. A method of applying heat energy can be used in which the cross-linking type protective layer **41** is heated from the application surface side or the substrate side using a gas, for example, air and nitrogen, vapor, or various kinds of heat media, infra-red radiation and electromagnetic wave. The heating temperature is not lower than 100°C. and preferably not higher than 170°C. When the heating temperature is too low, the reaction speed tends to be slow so that the curing reaction may not be complete. When the heating temperature is too high, the curing reaction is not uniformly conducted. Thereby, the protective layer **41** is significantly distorted inside, non-reaction groups may remain therein and three-dimensional mesh structure is not developed completely. To uniformly conduct the curing reaction, it is effective to heat the cross-linking type protective layer **41** at a relatively low temperature, for example lower than 100°C., followed by heating at a relatively high temperature, for example, higher than 100°C. to complete the curing reaction.

As light energy, a UV irradiation light source, for example, a high pressure mercury lamp or a metal halide lamp having an emission wavelength mainly in the ultraviolet area can be used. A visible light source can be selected according to the absorption wavelength of a radical polymerizable compound and a photopolymerization initiator. The irradiation light amount is preferably from 50 mW/cm<sup>2</sup> to 1,000 mW/cm<sup>2</sup>. When the irradiation light amount is too small, it takes a long time to complete the curing reaction. When the irradiation light amount is too large, the reaction is not uniformly conducted, resulting in the occurrence of wrinkle on the surface of the protective layer 41 and a significant amount of non-reacted groups and polymerization terminated ends. In addition, the internal stress in the protective layer 41 increases due to such rapid cross-linking, which causes cracking and peeling thereof. As radiation ray energy, electron beam can be used. Among these forms of energies, thermal or light energy is suitably used in terms of easiness of reaction speed control and simplicity of a device.

The layer thickness of the cross-linking protective layer of the present invention is preferably from 1 to 10 µm, and more preferably from 2 to 8 µm. When the layer thickness is too thick, cracking and peeling easily occur as described above. When the layer thickness is in the preferred range, the safety margin is improved so that the density of cross-linking can be increased. Further, it is possible to select a material and set a curing condition for a high anti-abrasion property. On the other hand, the radical polymerization reaction is vulnerable to oxygen inhibition. That is, on the surface, which contacts air, cross-linking tends to not proceed at all or uniformly due to the radical trap caused by oxygen. This radical trap has a significant effect on the portion having a depth not greater than 1 µm from the surface. Therefore, in the cross-linking type protective layer 41 having a thickness not greater than 1 µm, the anti-abrasion property may deteriorate and non-uniform abrasion may occur. In addition, when the layer thickness of the cross-linking type protective layer 41 is too thin, contaminants may diffuse in the entire layer, which leads to the inhibition of the curing reaction and the decrease of the density of cross-linking. Considering these, the cross-linking type protective layer 41 having a layer thickness not less than 1 µm has a good anti-abrasion property and anti-damage property. But when the cross-linking type protective layer 41 is locally ground to the charge transport layer 37 provided under the protective layer 41 during repetitive use, the ground portion is further abraded, resulting in the production of a half tone image with uneven density due to the fluctuation of chargeability and sensitivity. Therefore, to obtain a durable image bearing member and improve the image quality, the layer thickness of the cross-linking type protective layer 41 is preferably at least 2 µm.

In the structure of the image bearing member for use in the present invention in which the intermediate layer 39 (the charge blocking layer 43 and the moiré prevention layer 45), the photosensitive layer 38 (the charge generating layer 35 and the charge transport layer 37) and the cross-linking type protective layer 41 are accumulated on the substrate 31 in this order, when the cross-linking type protective layer 41 provided uppermost is insoluble in an organic solvent, the anti-abrasion property and the anti-damaging property can be significantly improved. A method of testing the solubility in an organic solvent is as follows: drop on the surface of an image bearing member a droplet of an organic solvent, for example, tetrahydrofuran and dichloromethane having a high solubility for a polymer, and subsequent to natural dry, observe the change in the form of the surface of the image bearing member with a microscope. In the case of an image

bearing member having a high solubility therein, the following phenomenon can be observed: the center portion on the image bearing member where the droplet has been dropped is dented and the portion therearound rises; the charge transport layer 37 precipitates, causing white turbidity or clouding due to the crystallization thereof; and wrinkled portion is observed as a result of swelling of the surface and contraction thereafter. To the contrary, an image bearing member insoluble in the organic solvent does not change at all and these phenomena are not observed.

In the structure of the present invention, to make the cross linking type protective layer 41 insoluble in an organic solvent, the following measures can be taken: (1) controlling the compositions and their content ratio of the liquid of application for the cross-linking type protective layer 41; (2) controlling the diluting solvent and the density of the solid portion of the cross linking type protective layer 41; (3) selecting the method of coating the cross linking type protective layer 41; (4) controlling the curing conditions of the cross linking type protective layer 41; and (5) making the charge transport layer 37 hardly soluble in an organic solvent. Each factor has an impact and desired to be used in combination.

When a binder resin having no radical polymerizable functional group and an additive such as an anti-oxidization agent and a plasticizer in a large amount are contained in a large amount in the composition of the cross linking type protective layer 41 in addition to the radical polymerizable monomer having at least three functional groups without having a charge transport structure and the radical polymerizable compound having a functional group and a charge transport structure mentioned above, the density of cross linking decreases, and the phase separation occurs between the cured material obtained as the result of the reaction and the additives. Consequently, the composition may be soluble in an organic solvent. Specifically, it is desired to restrain the content of the additives within not greater than 20% by weight based on the total solid portion of the liquid of application. In addition, not to reduce the cross linking density, it is also desired to restrain the total content of a radical polymerizable monomer having one or two monomers, a reactive oligomer, and a reactive polymer within not greater than 20% by weight based on the radical polymerizable monomer having three functional groups. Further, when a radical polymerizable compound having a charge transport structure having at least two functional groups is contained in a large amount, bulky structural bodies are fixed in multiple bondings in the cross linking structure, which may cause distortion. Therefore, such a structure tends to become an agglomeration of minute cured materials which may make the cross linking type protective layer 41 soluble in an organic solvent. Although it depends on structures, it is preferred to restrain the content of a radical polymerizable compound having a charge transport structure having at least two functional groups within not greater than 10% by weight based on the radical polymerizable compound having a charge transport structure and a functional group.

With regard to the dilution solvent for a liquid of application for the cross linking type protective layer 41, when a solvent having a slow evaporation speed is used, the remaining solvent may inhibit the curing reaction or increase the content of contaminants from the layer provided under the cross linking type protective layer 41, which causes non-uniform curing and the decrease in the curing density. Therefore, the protective layer 41 tends to be soluble in an organic solvent. Suitable specific examples of the dilution solvents include tetrahydrofuran, a mixture solvent of tetrahydrofuran and methanol, ethyl acetate, methylethyl ketone and ethylcellosolve. These are selected in combination with a coating

## 101

method. When the density of solid portion in a liquid of application is too low, the cross linking type protective layer 41 formed thereof tends to be dissolved in an organic solvent due to the same reason as described above. In contrast, on account of the restraint on the layer thickness and the viscosity of a liquid of application, the density has an upper limit. Specifically, the density is preferred to be from 10 to 50% by weight. As a method of coating a liquid of application for the cross linking type protective layer, as described above, a method is preferred in which the content of the solvent during coating is small and the contact time of the solvent is short. To be specific, a spray coating method or a ring coating method in which the amount of a liquid of application is regulated is preferred. In addition, to restrain the amount of the components infused from the layer provided under the protective layer 41, it is effective to use a charge transport polymer for the charge transport layer 37 and provide the intermediate layer 39 insoluble in a liquid of application for the cross linking type protective layer 41 between the photosensitive layer 38 (or the charge transport layer 37) and the cross linking type protective layer 41.

With regard to the curing conditions of the cross linking type protective layer 41, when the heating energy or light irradiation energy is too low, the curing reaction is not conducted completely. Thereby, the solubility thereof in an organic solvent increases. To the contrary, extremely high energy causes non-uniform curing reaction, which leads to the increase of non-cross linked portions and radical terminated portions and formation of an agglomeration of cured materials. The cross linking type protective layer 41 tends to be dissolved in an organic solvent. To make the cross linking type protective layer 41 insoluble in an organic solvent, heat curing is preferably performed at a temperature from 100 to 170° C. and for 10 minutes to 3 hours. UV irradiation curing is preferably performed at a range of from 50 to 1,000 mW/cm<sup>2</sup> for 5 seconds to 5 minutes while restraining the rise of the temperature within 50° C. Thereby, non-uniform curing reaction can be prevented.

Below are example methods of making the cross linking type protective layer 41 forming the image bearing member for use in the present invention insoluble in an organic solvent. For example, when an acrylate monomer having three acryloyloxy groups and a triaryl amine compound having an acryloyloxy group are used as a liquid of application, the content ratio of the acrylate monomer to the triaryl amine is 3/7 to 7/3 and an polymerization initiator is added in an amount of 3 to 20% by weight based on the total amount of the acrylate compound followed by an addition of a solvent to prepare the liquid of application. When a triaryl amine based doner and polycarbonate as a binder resin are used in the charge transport layer 37 provided under the cross linking type protective layer 41 and the surface thereof is formed by a spray coating method, it is preferred to use tetrahydrofuran, 2-butanone or ethyl acetate as the solvent mentioned above for the liquid of application, the content of which is 3 to 10 times as much as the total weight of the acrylate compound.

Next, for example, the liquid of application prepared as described above is applied with, for example, a spray, on an image bearing member in which the intermediate layer 39, the charge generating layer 35 and the charge transport layer 37 are accumulated on the substrate 31, for example, an aluminum cylinder. Subsequent to natural drying or drying at a relatively low temperature (25 to 80° C.) for a short time (1 to 10 minutes), the liquid of application is cured by UV ray irradiation or heat.

## 102

In the case of UV ray irradiation, a metal halide lamp, etc., is used for preferably about 5 seconds to about 5 minutes while the drum temperature is controlled not to be high than 50° C.

5 In the case of heat curing, the heating temperature is preferably from 100 to 170° C. An air supply oven is used as a heating device and when the heating temperature is set at 150° C., the liquid of application is heated for 20 minutes to 3 hours.

10 After the curing reaction is complete, to reduce the amount of the remaining solvent, the liquid of application is heated at 100 to 150° C. for 10 to 30 minutes and thus the image bearing member of the present invention is obtained.

In addition to a filler for use in forming the protective layer 15 41 or the cross linking type protective layer 41, it is also possible to use known materials, for example, a-C and a-SiC formed by a method of forming vacuum thin layer to form the protective layer 41.

20 As described above, when the protective layer 41 is formed on the photosensitive layer 38, it is preferred to select a suitable protective layer to make writing light and/or discharging light reach the photosensitive layer 38 in a sufficient amount to obtain the writing light and/or discharging function. In addition, the protective layer 41 tends to deteriorate while the protective layer 41 repetitively absorbs writing light and/or discharging light, which leads to the rise of the residual voltage. In each case of the protective layers 41 described above, the transmission factor of the protective layer 41 for writing light and/or discharging light is not less than 30%, preferably not less than 50% and more preferably not less than 85%.

30 The transmission factor of the protective layer 41 can be measured by the same method as for the charge transport layer 37. Spectral absorption of a protective layer which is singly formed for use in an image bearing member is measured by a spectral photometer available in the market. The transmission factor of light having a wavelength of writing light for use in an image forming apparatus can be obtained from the spectrum.

40 In addition, when an image bearing member having the protective layer 41 on the photosensitive layer 38 having the charge generating layer 35 and the charge transport layer 37 thereon is irradiated with discharging light from the surface of the image bearing member, the charge generating layer 35 is 45 irradiated with the discharging light which has transmitted through the protective layer 41 and the charge transport layer 37. Therefore, the transmission factors of the charge transport layer 37 and the protective layer 41 are of significant importance. The transmission factor of the discharging light for the charge transport layer 37 and the protective layer 41 in total is 50 not less than 30%, preferably not less than 50% and more preferably not less than 85%.

55 The transmission factor can be obtained by measuring the spectral absorption spectrum of the coated layer in which the charge transport layer 37 and the protective layer 41 are accumulated.

60 As described above, by providing the protective layer 41 on the surface of an image bearing member, the durability (anti-abrasion property) of the image bearing member is improved and a new effect which is not produced for a monochrome image forming apparatus can be provided for a tandem type full color image forming apparatus, which is described later.

65 In the present invention, to improve the environmental durability, especially to prevent the deterioration of the sensitivity and the rise in the residual voltage, an anti-oxidization agent can be suitably added in each layer of the protective

layer 41, the charge transport layer 37, the charge generating layer 35, the charge blocking layer 43, the moiré prevention layer 45, etc.

Specific examples of such anti-oxidization agents include the following:

phenol based compounds, for example, 2,6-t-butyl-p-cresol, butylated hydroxyl anisole, 2,6-di-t-butyl-4-ethylphenol, stearyl- $\beta$ -(3,5-di-t-butyl-4-hydroxyphehyl)propionate, 2,2'-methylene-bis(4-methyl-6-t-butylphenol), 2,2'-methylene-bis-(4-ethyl-6-t-butylphenol), 4,4'-thiobis-(3-methyl-6-t-butylphenol), 4,4'-butyldenebis-(3-methyl-6-t-butylphenol), 1,1,3-tris-(2-methyl-4-hydroxy-5-t-butylphenyl)butane, 1,3,5-trimethyl-2,4,6-tris(3,5-di-t-butyl-4-hydroxybenzyl) benzene, tetrakis-[methylene-3-(3',5'-di-t-butyl-4'-hydroxyphenyl)propionate]methane, bis[3,3'-bis(4'-hydroxy-3'-t-butylphenyl)butylic acid]glycol ester and tocopherols;

Paraphenylene diamines, for example, N-phenyl-N'-isopropyl-p-phenylene diamine, N,N'-di-sec-butyl-p-phenylene diamine, N-phenyl-N-sec-butyl-p-phenylene diamine, N,N'-di-isopropyl-p-phenylene diamine, and N,N'-dimethyl-N,N'-di-t-butyl-p-phenylene diamine;

Hydroquinones, for example, 2,5-di-t-octyl hydroquinone, 2,6-didodecyl hydroquinone, 2-dodecyl hydroquinone, 2-dodecyl-5-chloro hydroquinone, 2-t-octyl-5-methyl hydroquinone, 2-(2-octadecenyl)-5-methyl hydroquinone;

Organic sulfur compounds, for example, dilauryl-3,3-thiodipropionate, distearyl-3,3'-thiodipropionate, and ditetradecyle-3,3'-thiodipropionate; and

Organic phosphorus compounds, for example, triphenyl phosphine, tri(nonylphenyl)phosphine, tri(dinonylphenyl) phosphine, tricresyl phosphine and tri(2,4-dibutylphenoxy) phosphine.

These compounds are known as anti-oxidization agents for rubber, plastic, and oil and marketed products thereof can easily be obtained. The addition amount of the anti-oxidization agent in the present invention is from 0.01 to 10% by weight based on the total amount of the layer to which the anti-oxidization agent is added.

In the case of a full color image, various kinds of images including regular images are input. Proof marks in Japanese documents are one of such regular images. Images, for example, proof marks, are typically disposed at an edge of an image area and the usable color therefor is limited. In a state in which a random image is constantly written, writing, developing and transferring an image are averagely performed on and around the image bearing member in the image formation elements. However, when images are repeatedly written on a specific area many times or when only a specific image element is repeatedly used, the durability at the areas and of the image forming elements is thrown off balance. When an image bearing member having a surface the durability of which is physically, chemically and mechanically weak is used in such a state, the imbalance becomes significant among the elements, which leads to an image problem. To the contrary, when an image bearing member having a high durability is used, the local variation is small. Thereby, an abnormal image is hardly produced. Therefore, such an image bearing member has a high durability and the stability thereof is improved so that the image bearing member is extremely effective.

## Image Formation

The image formation mentioned above is performed by, for example, uniformly charring the surface of the image bearing member and thereafter irradiating the surface imagewise by the image forming device.

Image formation is performed by, for example, a charging device for uniformly charging the surface of the image bearing member and an irradiating device for irradiating the surface of the image bearing member imagewise.

## 10 Charging Device

There is no specific limit to the selection of the charging device. For example, there can be used a known contact type charging device having an electroconductive or semi-electroconductive roll, brush, film, and/or rubber blade and a known non-contact type charging device including a non-contact and vicinity type charging device having a space not greater than 100  $\mu\text{m}$  between the surface of an image bearing member and a charging device, for example, corotron and scorotorn, using corona discharging.

The electric field intensity applied to the image bearing member by the charging device is preferably from 20 to 60  $\text{V}/\mu\text{m}$  and more preferably from 30 to 50  $\text{V}/\mu\text{m}$ . The stronger the electric field intensity applied to the image bearing member is, the better the dot representation is. An electric field intensity that is too high may cause problems, for example, the insulation breakdown of an image bearing member and carrier attachment thereto during development.

The electric field intensity is represented by the following relationship:

$$\text{Electric field intensity } (\text{V}/\mu\text{m}) = SV/G$$

In the relationship, SV represents the absolute voltage (V) of the surface voltage at unirradiated portions on the image bearing member at the current position. G represents the layer thickness ( $\mu\text{m}$ ) of the photosensitive layer 38, i.e., at least the total thickness of the charge generating layer 35 and the charge transport layer 37.

## Writing Device

40 Writing can be performed by irradiating the surface of the image bearing member using the irradiating device. There is no specific limit to the selectin of the irradiating device as long as the irradiating device can emit light having a wavelength shorter than 450 nm. There can be used various kinds 45 of irradiating devices using, for example, a photocopying optical system, a rod lens array system, a laser optical system, and a liquid crystal shutter optical system. In the present invention, it is possible to adopt the bottom side irradiation by which an image bearing member is irradiated imagewise from the bottom side. As the light source for the irradiating device mentioned above, a light source securing a high brilliance, for example, a luminous diode (LED), a semi-conductor laser (LD), and an electroluminescence (EL), can be used.

50 There are technologies of oscillating laser in this wavelength range. One is a method in which the wavelength of a laser beam is halved by second harmonic generation (SHG) using a non-linear optical material (refer to JOPs H09-275242, H09-189930, H05-313033, etc.). In this system, it is possible to use GaAs LDs and YAG laser. These have been 55 established as technologies with high power output and long life. Another is a technology using a wide gap semiconductor, which can be reduced in size in comparison with a device using second harmonic generation (SHG).

55 LDs using ZnSe semiconductors (refer to JOPs H07-321409, H06-334272, etc.) or GaN semiconductors (refer to JOPs H08-88441, H07-335975, etc.) have been intensively 60 studied in light of luminance efficiency. Furthermore, as the

105

relatively leading edge technology, LDs (oscillation of 405 nm) using a GaN based semiconductor are marketed by Nichia Corporation. This technology contributes to the development of a highly advanced writing system in comparison with the other technologies described above and can be effectively used in the present invention. In addition, LED lamps using the materials mentioned above are marketed and also can be effectively used.

On the other hand, the lower limit is regulated by the following issue. That is, a charge transport material is used as a component forming an image bearing member, i.e., the charge transport layer 37 and the protective layer 41 existing on the writing light side. However, there is practically no charge transport material which not only has a high transport speed but also is sufficiently transparent to light having a wavelength less than about 350 nm. This is ascribable to the fact that most of the developed charge transport materials have a triaryl amine structure and the absorption end thereof on the long wavelength side is about from 300 to 350 nm. Therefore, when the wavelength of discharging light emitted by a light source can be shortened and the transparency (light absorption on the short wavelength side) of a charge transport material is improved, the oscillation of the light source for use in the present invention can advance to the short wavelength side.

According to the definition of a light source for writing light, the definition of a formed latent electrostatic image, resulting in a toner image, is determined. The higher the definition is, the clearer the image is. However, it takes a long time for writing with high definition so that when there is only one light source in an image forming apparatus, the writing is the rate controlling factor of the drum linear velocity (i.e., processing speed). Therefore, about 2,400 dpi is the upper limit of the definition when there is one light source for writing. When there are multiple light sources for writing, each thereof can irradiate just each corresponding writing area. Therefore, the upper limit of the definition is regulated by  $(2,400 \text{ dpi}) \times (\text{the number of light sources for writing})$ . Among these light sources mentioned above, a luminous diod and a semi-conductor laser have a high irradiation energy and can be effectively used.

#### Developing Device

Development can be performed by developing a latent electrostatic image with a toner to form a visualized image. A toner having the same polarity as the charging polarity of an image bearing member is used and the latent electrostatic image is developed using the reverse development (negative-positive development). There are two development systems. One is a single component development system using only a toner and the other is a two component development system using a toner and a carrier. Both can be suitably applied.

#### Transfer Device

The visualized image is transferred by a transfer device. There are two kinds of transfer methods. One is a method in which the visualized image is directly transferred from the surface of an image bearing member to a recording medium. The other is a method in which the visualized image is primarily transferred to an intermediate transfer body and then secondarily transferred to a recording medium. Both methods are applicable but when the transfer has an adverse impact on the improvement of the quality of images, the former method (direct transfer method) is preferred.

Transferring the visualized image can be performed by, for example, charging an image bearing member with a transfer charging device and with the transfer device mentioned above. There is no specific limit to the transfer device and any

106

known device can be suitably used. For example, a transfer conveyor belt, which can simultaneously transfer a recording medium, can be suitably used.

5 The transfer device (a primary transfer device and a secondary transfer device) preferably has a transfer charging device by which the visualized image formed on an image bearing member is charged and detached to a recording medium. The transfer device can be plural. There can be used a corona transfer device using corona discharging, a transfer belt, a transfer roller, a pressure transfer roller and an adhesive transfer device as the transfer charging device. The recording medium has no specific limit to its selection and can be selected from any known recording medium (paper).

10 In addition, a transfer belt and a transfer roller can be used as the transfer charging device but it is preferred to use a contact type transfer belt or a contact type transfer roller which less produces ozone. It is possible to use either of a constant voltage system and a constant electric current system as the voltage/electric current applying system during transfer. The constant electric current system is preferred because the constant electric current system can constantly hold the amount of transfer charges and is more stabilized than the other. Known transfer devices can be used as long as the structure can satisfy the present invention.

15 20 25 30 35 The amount of charges passing through an image bearing member per image formation cycle greatly varies depending on the surface voltage (surface voltage when entering into the discharging portion) of the image bearing member after transfer. A large surface voltage has a significant influence on the electrostatic fatigue of an image bearing member during repetitive use.

35 40 45 50 The amount of charges passing through an image bearing member corresponds to the amount of charge trespassing along the layer thickness direction of the image bearing member. An image bearing member is charged (negatively charged in most cases) at a preferred charging voltage by a main charging device and optical writing is performed based on the input signals according to an original. Photocarriers are generated at the optically written portions and the surface charges are neutralized (potentially decayed). The charges flow in the layer thickness of the image bearing member depending on the amount of the generation of photocarriers. On the other hand, the non-optically written portion advances to the discharging portion after the developing process and the transfer process (and optionally a cleaning process). When the surface voltage of the image bearing member is close to the voltage charged by the main charging device (excluding the darkness decayed amount), the charges having almost the same amount as that corresponding to the optically written portions flow in the layer thickness of the image bearing member. In general, the writing ratio in an original is so low that almost all of the amount of charges passing through the image bearing member in this system is generated in the discharging process. For example, 90% of the total electric current flows in the discharging process when the writing ratio is 10%.

55 60 65 The charges passing through the image bearing member has a great adverse impact on the characteristics of the image bearing member, for example, causing the deterioration of the materials for use in the image bearing member. As a result, especially the residual voltage of the image bearing member rises depending on the amount of the charges passing through the image bearing member. When the residual voltage of the image bearing member rises, the image density decreases in the negative or positive development for use in the present invention, which is a large problem. Therefore, to achieve a long life (high durability) of an image bearing member for use

107

in an image forming apparatus, how to make the charges passing through an image bearing member small is of a significant importance.

To the contrary, an idea of not performing optical discharging is thinkable. But a main charging device is preferred to have a large charging ability to secure the charging, otherwise a problem, for example, residual images, may occur. Passing of charges through an image bearing member of charges is the transfer of the photocarriers generated by the electric field caused by the voltage charged at the surface of the image bearing member and optical irradiation. Therefore, when the surface voltage can be decayed by a means other than light, the amount of charges passing through an image bearing member per one rotation of the image bearing member (i.e., one cycle of image formation) is reduced.

The amount of charges can be effectively adjusted by adjusting the transfer bias in the transfer process. An image bearing member is charged by a main charging device and non-written portions thereon sustain a voltage (excluding the amount caused by darkness decay) close to the charging voltage and enter into the transfer process. When the absolute value on the polarity of charges charged by the main charging device is reduced to not greater than 100 V, the photocarriers and charges passing through the image bearing member are hardly generated when the image bearing member enters into the following discharging process. This absolute value is more preferred when the value is closer to zero. Furthermore, when a transfer bias is applied to an image bearing member through adjustment of the transfer bias such that the surface voltage thereof has a polarity reverse to the polarity imparted by the main charging, the photocarrier is never produced, which is more preferred. However, under the condition such that the surface voltage of an image bearing member has the reverse polarity, transfer debris may be produced in a large amount and the main charging in the next image formation cycle may not be performed in time. This may cause a problem of producing residual images. Therefore, the absolute value of the surface voltage of an image bearing member by a transfer bias is preferred to be not greater than 100 V.

The adjustment mentioned above makes the effect of the present invention clear and is preferably used.

#### Fixing Device

The visualized image transferred to a recording medium is fixed by a fixing device. Fixing can be performed when each color toner is transferred to the recording medium or performed simultaneously after each color toner is accumulated on the recording medium.

There is no specific limit to the fixing device and a known heating and pressing fixing device is suitably used. A combination of a heating roller and a pressing roller and a combination of a heating roller, a pressing roller and an endless belt can be applicable. The temperature of a heating and pressing fixing device is preferably from 80 to 200°C. In the present invention, for example, a known optical fixing device can be used in place of such fixing devices.

#### Discharging Device

Any known discharging device can be suitably selected as long as the discharging device can perform discharging an image bearing member. For example, a semi-conductor laser (LD) and an electroluminescence (EL) can be used. In addition, the effect of the present invention is all the more clear when a light source emitting light having a wavelength shorter than 450 nm (i.e., wavelength of light which can be absorbed by the metal oxide contained in the intermediate layer 39 of the image bearing member) is used to discharge the image bearing member.

108

As the light source having such a wavelength, there can be used a semiconductor laser (LD) or an electroluminescence (EL) which can oscillate light having a wavelength shorter than 450 nm and a combination of a fluorescent lamp, a tungsten lamp, a halogen lamp, a mercury lamp, a sodium lamp or a xenon lamp with an optical filter which can restrain the luminescence in the range of a wavelength shorter than 450 nm. As the optical filter, various kinds of filters, for example, a sharp cut filter, a band-pass filter, a near infrared filter, a dichroic filter, a coherent filter and a color conversion filter, can be used for irradiation of light having a wavelength in a preferred range (i.e., shorter than 450 nm).

#### Others

There is no specific limit to the cleaning device. Any known cleaning device can be used as long as the toner remaining on an image bearing member can be removed. For example, a magnetic brush cleaner, an electrostatic brush cleaner, a magnetic roller cleaner, a blade cleaner, a brush cleaner and a web cleaner can be suitably used.

The recycling process is a process of returning the toner removed by the cleaning device to the developing device for recycle use. Any known transport system can be used as the recycling system.

The controlling process is a process of controlling each process mentioned above by a controlling device.

There is no specific limit to the selection of the controlling device and any known controlling device can be suitably selected as long as the controlling device can control the behavior of each device. For example, devices, for example, a sequencer and a computer, can be used.

An embodiment of the image forming apparatus of the present invention is described with reference to FIG. 9.

FIG. 9 is a schematic diagram illustrating the image forming apparatus of the present invention. The variations described later are within the scope of the present invention.

In FIG. 9, an image bearing member 1 has an intermediate layer containing a metal oxide and a layered photosensitive layer including a charge generating layer containing an organic charge generating material and a charge transport layer containing a charge transport material on a substrate. The image bearing member 1 has a drum form but a sheet form or an endless form is also allowed.

A charging device having a wire system or a roller form is used as a charging device 3. When a high speed charging is desired, a charging device of a scorotron system is preferably used. In an image forming apparatus of a compact size or of a tandem type using plurality of the image bearing members described later, a charging device having a roller form which can restrain the production of acidic gasses (e.g., NO<sub>x</sub> and SO<sub>x</sub>) and ozone is effectively used. The charging device 3 charges the image bearing member 1. Since the dot representation is improved as the electric field intensity applied to the image bearing member 1 increases, the electric field intensity is preferably not less than 20 V/μm. However, this may cause problems, for example, the insulation breakdown of the image bearing member 1 and carrier attachment thereto during development. Therefore, the upper limit of the electric field intensity is about 60 V/μm and preferably 50 V/μm.

A light source, for example, a luminous diode (LED), a semi-conductor (LD) and an electroluminescence (EL), which can secure high brightness and can write with light having a wavelength shorter than 450 nm which can be absorbed by the metal oxide contained in the intermediate layer 39, is used in an image irradiation portion 5. The definition of a formed latent electrostatic image, resultingly a toner image, is determined by the definition of a light source

109

for writing light. The higher the definition is, the more clear the image is. However, it takes a long time for writing with high definition so that when there is only one light source in an image forming apparatus, the writing is the rate controlling factor of the drum linear velocity (i.e., processing speed). Therefore, about 2,400 dpi is the upper limit of the definition when there is one light source for writing. When there are multiple light sources for writing, each thereof can irradiate just each corresponding writing area. Therefore, the upper limit of the definition is regulated by  $(2,400 \text{ dpi}) \times (\text{the number of light source for writing})$ . Among these light sources mentioned above, a luminous diode and a semi-conductor laser have a high irradiation energy and can be effectively used.

A developing unit 6 functioning as a developing device has at least one developing sleeve.

In the developing unit 6, a toner having the same polarity as that of the image bearing member 1 and a latent electrostatic image is developed by the reverse development (negative and positive development). Although it depends on the light source for use in the image irradiation portion 5, to elongate the life of the light source, the reverse development system in which toner development is performed for written portions is advantageous in the case of a digital light source which have been recently used in reflection of the low image area ratio in general. There are two development systems. One is a single component development system using only a toner and the other is a two component development system using a toner and a carrier. Both can be suitably applied.

A transfer belt and a transfer roller can be used as a transfer charging device 10, but it is preferred to use a contact type transfer belt and a contact type transfer roller which less produce ozone. It is possible to use either of a constant voltage system and a constant electric current system as the voltage/electric current applying system during transfer. The constant electric current system is preferred because the constant electric current system can constantly hold the amount of transfer charges and is more stabilized than the other. Especially, a method is preferred in which the electric current to the image bearing member 1 is controlled by subtracting the electric current which does not flow in the image bearing member 1 but in portions related to transfer members from the electric current output from a high voltage power supply for providing charges to the transfer members.

The transfer electric current is an electric current by which toner electrostatically attached to the image bearing member 1 is detached and transferred to a transfer body (e.g., transfer medium 9 or an intermediate transfer body). To avoid poor transfer performance, for example, remaining transfer, it is desired to have a large transfer electric current. However, in the case of the reverse development (negative or positive development), the charges having a polarity reverse to the charging polarity of the image bearing member 1 are provided so that the image bearing member 1 is electrostatically fatigued significantly. It is true that a large transfer electric current is advantageous to provide an amount of charges having a stronger force than the electrostatic attachment force between the image bearing member 1 and the toner. However, a transfer electric current that is larger than a threshold causes discharging between the transfer members and the image bearing member 1, resulting in scattering of a finely developed toner image. The threshold is a value below which the discharging does not occur and varies depending on the distance (space) between the transfer members and the image bearing member 1 and the materials forming the transfer members and the image bearing member 1. The discharging can be avoided below about 200  $\mu\text{A}$  so that the upper limit of the transfer electric current is about 200  $\mu\text{A}$ .

110

In addition, there are two methods for transferring the toner image formed on the image bearing member 1 to the transfer medium (paper) 9. One is the direct transfer in which a toner image developed on the image bearing member 1 is directly transferred as in FIG. 9. The other is a method in which a toner image developed on the image bearing member 1 is transferred to the transfer medium 9 via an intermediate body. Both methods can be suitably used in the present invention.

Any known transfer member can be used as long as the transfer member satisfies the structure of the present invention.

When the surface voltage at non-irradiated portions by the writing light of the image bearing member 1 after transfer is reduced by controlling the transfer electric current as described above, the amount of charges passing through the image bearing member 1 per cycle of image formation can be reduced. This can be effectively used in the present invention.

There is no specific limit to the selection of the light source for use in a discharging lamp 2 as long as the light source can discharge the image bearing member and any known discharging device can be selected. For example, a semiconductor laser (LD) and electroluminescence (EL) are suitably selected. In particular, the effect of the present invention is all the more clear when a light source emitting light having a wavelength shorter than 450 nm (i.e., wavelength of light which can be absorbed by the metal oxide contained in the intermediate layer 39 of the image bearing member) is used to discharge the image bearing member.

As the light source for a semiconductor laser (LD), electroluminescence (EL), etc., for example, there can be used a semiconductor laser or an electroluminescence (EL) which can oscillate light having a wavelength shorter than 450 nm and a combination of a fluorescent lamp, a tungsten lamp, a halogen lamp, a mercury lamp, a sodium lamp or a xenon lamp with an optical filter which can restrain the luminescence in the range of a wavelength shorter than 450 nm. As the optical filter, various kinds of filters, for example, a sharp cut filter, a band-pass filter, a near infrared filter, a dichroic filter, a coherent filter and a color conversion filter, can be used for the irradiation of light having a wavelength in a preferred range (i.e., shorter than 450 nm).

In FIG. 9, 8 represents a pair of registration rollers, 11 represents a separation charging device, and 12 represents a separation claw.

In addition, the toner developed on the image bearing member 1 by the developing unit 6 is transferred to the transfer medium 9. Toner remaining on the image bearing member 1 is removed by a fur brush 14 and a cleaning blade 15. Cleaning can be performed only by a cleaning brush. Known cleaning brushes, for example, a fur brush and a magfur brush, can be used as the cleaning brush 14.

FIG. 10 is a schematic diagram illustrating an example of the tandem type full color image forming apparatus of the present invention. The variations described later are also within the scope of the present invention.

In FIG. 9, each of 16Y, 16M, 16C and 16K represents a drum image bearing member. Each image bearing member has an intermediate layer containing a metal oxide and a layered photosensitive layer including a charge generating layer containing an organic charge generating material and a charge transport layer containing a charge transport material on a substrate.

These image bearing members 16Y, 16M, 16C and 16K can rotate in the direction indicated by the arrows in FIG. 9. Around the image bearing members 16Y, 16M, 16C and 16K, charging devices 17Y, 17M, 17C and 17K, developing devices 19Y, 19M, 19C and 19K having a developing sleeve,

## 111

cleaning devices 20Y, 20M, 20C and 20K, and discharging devices 27Y, 27M, 27C and 27K are arranged along the rotation direction of the image bearing members 16Y, 16M, 16C and 16K. The charging devices 17Y, 17M, 17C and 17K, are charging devices for uniformly charging the surface of the image bearing members 16Y, 16M, 16C and 16K. Irradiating devices 18Y, 18M, 18C and 18K irradiate the surface of the image bearing members 16Y, 16M, 16C and 16K with a laser beam having a wavelength shorter than 450 nm from between the charging devices 17Y, 17M, 17C and 17K and the developing devices 19Y, 19M, 19C and 19K to form latent electrostatic images on the image bearing members 16Y, 16M, 16C and 16K. Four image forming elements 25Y, 25M, 25C and 25K having the image bearing members 16Y, 16M, 16C and 16K as main components are arranged along a transfer belt 22. The transfer belt 22 are brought into contact with the image bearing members 16Y, 16M, 16C and 16K between the developing devices 19Y, 19M, 19C and 19K and cleaning devices 20Y, 20M, 20C and 20K. Transfer brushes 21Y, 21M, 21C and 21K for applying a transfer bias are arranged on the opposite side of the transfer belt 22 relative to the image bearing members 16Y, 16M, 16C and 16K. Each of the image forming elements 25Y, 25M, 25C and 25K have the same structure except for the color of the toner contained therein.

The image formation is performed in the full color image forming apparatus having the structure illustrated in FIG. 10 as follows.

First, latent electrostatic images are formed on the image bearing members 16Y, 16M, 16C and 16K in each of the image forming elements 25Y, 25M, 25C and 25K. Then the image bearing members 16Y, 16M, 16C and 16K rotate and are charged by the charging devices 17Y, 17M, 17C and 17K. To form a fine latent electrostatic image, the electric field intensity of the image bearing members 16Y, 16M, 16C and 16K is from 20 to 60 V/μm and preferably to 50 V/μm.

Next, the irradiating devices 18Y, 18M, 18C and 18K arranged outside the image bearing members 16Y, 16M, 16C and 16K perform writing with a laser beam having a wavelength shorter than 450 nm which can be absorbed by the metal oxide contained in the intermediate layer 39 with a definition not less than 1,200 dpi, preferably not less than 2,400 dpi to form latent electrostatic images corresponding to each color formed image. As described above, any light source suitable for the image bearing members 16Y, 16M, 16C and 16K can be used as the light source for writing light. The upper limit of the definition of a light source for writing light is about 2,400 dpi.

Next, the developing devices 19Y, 19M, 19C and 19K develop latent electrostatic images and form corresponding toner images. The developing devices 19Y, 19M, 19C and 19K are developing devices developing latent images with toners of Y (Yellow), M (Magenta), C (Cyan) and K (Black) and respective color toner images formed on four image bearing members 16Y, 16M, 16C and 16K are overlapped on a transfer medium 26. The transfer medium 26 is sent out from a tray by paper feeding rollers (not shown), temporarily held at a pair of registration rollers 23 and transferred to the transfer belt 22 synchronously with a timing of image formation on the image bearing members 16Y, 16M, 16C and 16K. The transfer medium 26 held on the transfer belt 22 is transferred and each color toner image is transferred thereto at the contact point (transfer point) of the transfer medium 26 and the image bearing members 16Y, 16M, 16C and 16K.

The toner images on the image bearing members 16Y, 16M, 16C and 16K are transferred to the transfer medium 26

## 112

by the potential between the transfer bias applied to the transfer brushes 21Y, 21M, 21C and 21K and the image bearing members 16Y, 16M, 16C and 16K. The transfer medium 26 on which four color toner images are overlapped while passing through the four transfer points is transferred to a fixing device 24, where the toner is fixed, and output to a medium discharging portion (not shown).

In addition, the toner which has not been transferred at the transfer points and remains on the image bearing members 16Y, 16M, 16C and 16K is retrieved by the cleaning devices 20Y, 20M, 20C and 20K.

Next, the extra residual charges on the image bearing members 16Y, 16M, 16C and 16K are removed by the discharging devices 27Y, 27M, 27C and 27K. Thereafter, the image bearing members 16Y, 16M, 16C and 16K are again charged by the charging devices 17Y, 17M, 17C and 17K to start the next image formation.

In addition, in the example illustrated in FIG. 10, the image forming elements 25Y, 25M, 25C and 25K are arranged in this order from the upstream to the downstream of the transfer belt 22 relative to the transfer direction of the transfer medium 26 but can be arranged in any order. It is especially effective to provide a mechanism by which the image forming elements 25Y, 25M and 25C forming color images other than black images are suspended when a black color image is formed.

In addition, as described above, the surface of the image bearing members 16Y, 16M, 16C and 16K after transfer is preferably charged to have a voltage not greater than 100 V with the same polarity as that of the image bearing members 16Y, 16M, 16C and 16K charged by the charging devices 17Y, 17M, 17C and 17K, more preferably with the polarity reverse thereto and especially preferably a voltage not greater than 100 V with the reverse polarity. Thereby, the rise of the residual voltage of the image bearing members 16Y, 16M, 16C and 16K during repetitive use can be reduced.

The devices mentioned above relating to the image formation can be fixedly incorporated in a photocopier, a facsimile machine or a printer or take a form of a process cartridge, which is incorporated therein as a whole. The process cartridge is a device (part) including an image bearing member and at least one of the devices, for example, an image forming device, a developing device, a transfer device, a cleaning device and a discharging device. The process cartridge can be freely designed. A general example thereof is as illustrated in FIG. 11. An image bearing member 101 includes a substrate on which an intermediate layer containing a metal oxide and a layered photosensitive layer including a charge generating layer containing an organic charge generating material and a charge transport layer containing a charge transport material.

An image irradiating portion 103 preferably uses a light source which can write with light having a wavelength shorter than 450 nm which can be absorbed by the metal oxide contained in the intermediate layer 39. Any charging device can be used as a charging device 102. In FIG. 11, 104 represents a developing device including at least one developing sleeve, 105 represents a transfer body, 106 represents a transfer device, and 107 represents a cleaning device and 108 represents a discharging device.

Having generally described preferred embodiments of this invention, further understanding can be obtained by reference to certain specific examples which are provided herein for the purpose of illustration only and are not intended to be limiting. In the descriptions in the following examples, the numbers represent weight ratios in parts, unless otherwise specified.

## EXAMPLES

Below are the detailed descriptions of the present invention with reference to Examples but the present invention is not limited thereto.

First, the methods of synthesizing azo pigments and titanyl phthalocyanine having a crystal form for use in the present invention are described.

The azo pigment for use in Examples is manufactured in accordance with the methods described in examined published Japanese patent application No. (hereinafter referred to as JPP) S60-29109 and JP 3026645. The titanyl phthalocyanine having a crystal form is manufactured in accordance with the methods described in JOPs 2001-19871 and 2004-83859.

## Synthesis of Titanyl Phthalocyanine having Crystal Form

## Synthesis Example 1

A titanyl phthalocyanine having a crystal form is manufactured in accordance with Synthesis Example 1 in JOP 2001-19871. That is: Mix 29.2 g of 1,3-diiminoisoindoline and 200 ml of sulforan and drop 20.4 g of titanium tetrabuthoxide to the resultant liquid in nitrogen atmosphere; Subsequent to the drop, gradually heat the resultant liquid to 180° C. followed by 5 hour stirring while keeping the reaction temperature between 170 to 180° C.; After standing to cool, filter the precipitated material and wash the resultant powder with chloroform until the color thereof shows blue; Wash the resultant with methanol several times and thereafter with hot water of 80° C. several times; Subsequent to drying, coarse titanyl phthalocyanine is obtained; Dissolve the coarse titanyl phthalocyanine in concentrated sulfuric acid having an amount 20 times as much as the amount of the coarse titanyl phthalocyanine and drop the resultant to iced water in an amount 100 times as much as that of the resultant while stirring; Filter the precipitated crystal and repetitively wash the crystal with deionized water (pH: 7.0 and specific conductivity: 1.0  $\mu$ S/cm) until the washing water shows neutral (pH: 6.8 and specific conductivity: 2.6  $\mu$ S/cm) and wet cake (water paste) of titanyl phthalocyanine pigment is thus obtained; and place 40 g of the wet cake in 200 g of tetrahydrofuran followed by 4 hour stirring, filtering and drying and thereby powder of titanyl phthalocyanine is obtained as Pigment No. 1.

The density of the solid portion of the wet cake is 15% by weight. The amount of the crystal conversion solvent is 33 times in weight ratio based on the amount of the wet cake. The raw material of Synthesis Example 1 does not contain a halogen containing compound.

The obtained titanyl phthalocyanine powder has a CuK $\alpha$  X ray diffraction spectrum having a wavelength of 1.542 Å with a market product of an X ray diffraction device (manufactured by Rigaku Corporation such that a maximum diffraction peak is observed at a Bragg (20) angle of 27.2±0.2°, main peaks at a Bragg (21) angle of 9.4±0.2°, 9.6±0.2°, and 24.0±0.2°, and a peak at a Bragg (20) angle of 7.3±0.2° as the lowest angle

diffraction peak, and having no peak between the peak of 9.4°±0.2° peak and the peak of 7.3°±0.2° and no peak at 26.3° when measured under the following conditions:

## 5 X Ray Diffraction Spectrum Measuring Conditions

X ray tube: Cu

Voltage: 50 kV

Current: 30 mA

## 10 Scanning speed: 2°/min

Scanning area: 3 to 40°

Time constant: 2 seconds

The result is shown in FIG. 12.

15 In addition, part of the water paste obtained in Synthesis Example 1 is dried for 2 days with a reduced pressure of 5 mm Hg at 80° C. to obtain titanyl phthalocyanine powder having a low crystalline property. X ray diffraction spectrum of the dried powder of the water paste is shown in FIG. 13.

## 20 Synthesis Example 2

25 A water paste of titanyl phthalocyanine pigment is synthesized in accordance with the method of Synthesis Example 1 of JOP 2004-83859 and crystal converted as follows to obtain titanyl phthalocyanine crystal having a primary particle diameter smaller than that of Synthesis Example 1:

30 Add 400 parts by weight of tetrahydrofuran to 60 parts of the water paste before crystal conversion obtained in Synthesis Example 1 and violently stir the resultant with HOMO-MIXER (Mark II Model, manufactured by Kenis, Ltd.) at 2,000 rpm at room temperature; When the color of the paste changes from indigo to light blue (after about 20 minutes stirring), stop the stirring and immediately filter the resultant with a reduced pressure; Wash the crystal obtained on the filtering device with tetrahydrofuran to obtain a wet cake of the pigment; and dry the wet cake for 2 days at 70° C. with a reduced pressure of 5 mmHg to obtain 8.5 parts by weight of 35 titanyl phthalocyanine crystal, which is Pigment No. 2. The raw material of Synthesis Example 2 does not contain a halogen containing compound. The density of the solid portion of the wet cake is 15% by weight. The amount of the 40 crystal conversion solvent is 44 times in weight ratio based on the amount of the wet cake.

45 Dilute part of the titanyl phthalocyanine (water paste) before crystal conversion manufactured in Synthesis Example 1 with deionized water to obtain a 1% by weight solution; Scrape the solution with a copper net the surface of 50 which is electric conductively treated; and observe the particle diameter of titanyl phthalocyanine with a transmission electron microscope (TEM)(H-9000NAR, manufactured by Hitachi Ltd.) with a magnifying power of 75,000. The average particle diameter is obtained as follows:

55 The TEM image as observed above is photographed as a TEM photograph. 30 titanyl phthalocyanine particles, which have a form similar to a needle, are arbitrarily selected in the TEM photograph and the major axis of each particle is measured. The arithmetical mean of the major axes of the 30 particles are calculated and determined as the average particle diameter. The average particle diameter of the water paste (wet cake) of Synthesis Example 1 as measured above is 0.06  $\mu$ m.

60 In addition, titanyl phthalocyanine crystal just before filtration in Synthesis Example 1 and 2 is diluted with tetrahydrofuran to obtain a 1% by weight solution and observed by

## 115

the same method as mentioned above. The average particle diameters obtained as described above are shown in Table 1. Titanyl phthalocyanine crystals manufactured in Synthesis Example 1 and 2 do not necessarily have the same crystal form. For example, there are forms similar to a triangle and a square. The longest diagonal of the crystal is measured as the major axis for calculation.

TABLE 1

|                                        | Average particle size (μm) | Memo                                                                             |
|----------------------------------------|----------------------------|----------------------------------------------------------------------------------|
| Synthesis Example 1<br>(Pigment No. 1) | 0.31                       | Contains particles having a large particle diameter of about 0.3 to about 0.4 μm |
| Synthesis Example 2<br>(Pigment No. 2) | 0.12                       | Sizes of crystal are almost uniform                                              |

The X-ray diffraction spectrum of Pigment No. 2 manufactured in Synthesis Example 2 is measured in the same method as mentioned above. As a result, the X-ray diffraction spectrum thereof matches the spectrum of Pigment No. 1 manufactured in Synthesis Example 1.

## Liquid Dispersion Manufacturing Example 1

A liquid dispersion 1 is prepared by using Pigment No. 1 manufactured in Synthesis Example 1 with the following

## 116

5 dispersion Manufacturing Example 1 is replaced with Pigment No. 2 prepared in Synthesis Example 2.

## Liquid Dispersion Manufacturing Example 3

10 A liquid dispersion 3 is prepared by filtering the liquid dispersion 1 prepared in Liquid Dispersion Manufacturing Example 1 with a cotton wind cartridge filter (TCW-1-CS, manufactured by Advantec Co., Ltd.) having an effective hole diameter of 1 μm. The filtration is performed using a pump with an increased pressure.

## Liquid Dispersion Manufacturing Example 4

15 A liquid dispersion 4 is prepared in the same manner as described in preparation of Liquid Dispersion Manufacturing Example 3 except that the filter used therein is replaced with 20 a cotton wind cartridge filter (TCW-3-CS, manufactured by Advantec Co., Ltd.) having an effective hole diameter of 3 μm.

## Liquid Dispersion Manufacturing Example 5

25 A liquid dispersion 5 is prepared by using the following receipe under the following condition as liquid of application for a charge generating layer.

Azo pigment represented by the following chemical structure:

5 parts



Polyvinyl butyral (BX-1, manufactured by Sekisui Chemical Co., Ltd.)  
Cyclohexanone  
2-butanone

2 parts  
250 parts  
100 parts

composition under the following condition as a liquid of application for a charge generating layer.

The liquid dispersion 5 is prepared by: placing all of the solvent in which polyvinyl butyral is dissolved and the azo pigments in a bead mill dispersing device with PSZ balls 50 having a particle diameter of 10 mm; and dispersing the solution for 7 days with a rotation speed of 85 rpm of the rotor.

|                                                                     |           |
|---------------------------------------------------------------------|-----------|
| Titanyl phthalocyanine pigment (Pigment No. 1)                      | 15 parts  |
| Polyvinylbutyral (BX-1, manufactured by Sekisui Chemical Co., Ltd.) | 10 parts  |
| 2-butanone                                                          | 280 parts |

55 The liquid dispersion 1 is prepared by: placing all of 2-butanone in which polyvinyl butyral is dissolved and Pigment No. 1 in a marketed bead mill dispersing device (DISPER-MAT: SL-05C1-EX) with PSZ balls having a particle diameter of 0.5 mm; and dispersing the solution for 30 minutes with a rotation speed of at 1,200 rpm of the rotor.

## Liquid Dispersion Manufacturing Example 2

60 A liquid dispersion 2 is prepared in the same manner as described in preparation of Liquid Dispersion Manufacturing Example 1 except that Pigment No. 1 for use in Liquid Dis-

## Liquid Dispersion Manufacturing Example 6

65 A liquid dispersion 6 is prepared in the same manner as described in preparation of Liquid Dispersion Manufacturing Example 5 except that the azo pigment used in Liquid Dispersion Manufacturing Example 5 is changed to the azo pigment represented by the following chemical structure:



The particle size distributions of the pigment particles in liquid dispersion prepared as described above are measured by CAPA-700, manufactured by Horiba Ltd. The results are shown in Table 2.

TABLE 2

|                     | Average particle diameter (μm) | Standard deviation (μm) |
|---------------------|--------------------------------|-------------------------|
| Liquid dispersion 1 | 0.29                           | 0.18                    |
| Liquid dispersion 2 | 0.19                           | 0.13                    |
| Liquid dispersion 3 | 0.22                           | 0.16                    |
| Liquid dispersion 4 | 0.24                           | 0.17                    |
| Liquid dispersion 5 | 0.26                           | 0.18                    |
| Liquid dispersion 6 | 0.27                           | 0.17                    |

#### Image Bearing Member Manufacturing Example 1

A liquid of application for an intermediate layer having the following composition, a liquid of application for a charge generating layer and a liquid of application for a charge transport layer are applied to an aluminum drum (JIS 1050)

15 having a diameter of 30 mm. Subsequent to drying, Image bearing member 1 (a layered image bearing member) having an intermediate layer having a thickness of 3.5 μm, a charge generating layer and a charge transport layer having a thickness of 25 μm are manufactured.

20 The layer thickness of the charge generating layer is adjusted as follows: apply a liquid for a charge generating layer to a substrate having an aluminum drum substrate prepared beforehand around which a polyethylene terephthalate film is wound in the same manner as described for preparing Image bearing member 1. The transmission factor of the 25 charge generating layer for light having a wavelength of 407 nm is measured by a marketed spectral photometer (UV-3100, manufactured by Shimadzu Corporation) while comparing with polyethylene terephthalate on which a liquid for charge generating layer is not coated. The layer thickness is 30 adjusted such that the result of the transmission factor is 20%.

The transmission factor of the charge transport layer is measured in the same manner. The result for the charge transport layer having a thickness of 407 nm having the following composition is 98%.

#### Liquid of Application for Intermediate Layer

|                                                                                                                                                    |            |
|----------------------------------------------------------------------------------------------------------------------------------------------------|------------|
| Non-surface treated rutile type titanium oxide having an average particle diameter of 0.25 μm (CR-EL, manufactured by Ishihara Industry Co., Ltd.) | 112 parts  |
| Alkyd resin (BECKOLITE M6401-50-S, manufactured by Dainippon Ink and Chemicals Incorporated, solid portion: 50%)                                   | 33.6 parts |
| Melamine resin (SUPERBECAKMINE L-121-60, manufactured by Dainippon Ink and Chemicals Incorporated, solid portion: 60%)                             | 18.7 parts |
| 2-butanone                                                                                                                                         | 260 parts  |
| Liquid of Application for Charging Generating Layer                                                                                                |            |

The liquid dispersion 1 is used.

#### Liquid of Application for Charge Transport Layer

|                                                                                                                                             |                     |
|---------------------------------------------------------------------------------------------------------------------------------------------|---------------------|
| Polycarbonate (TS2050, manufactured by Teijin Chemicals Ltd.)<br>Charge transport material represented by the following chemical structure: | 10 parts<br>7 parts |
|---------------------------------------------------------------------------------------------------------------------------------------------|---------------------|



Methylene chloride

80 parts

119

An intermediate layer is formed using the liquid of application mentioned above for intermediate layer on an aluminum board having a thickness of 1 mm in the same manner as described in manufacturing of the Image bearing member 1 using the liquid of application for the intermediate layer. The spectroscopic reflection spectrum of the intermediate layer is measured by a marketed spectral photometer (UV-3100, manufactured by Shimadzu Corporation). The absorption end (the upper limit of the wavelength of light which can be absorbed therein) of intermediate layer is obtained from the spectroscopic reflection spectrum. The result of the absorption end of the titanium oxide mentioned above is about 410 nm.

#### Image Bearing Member Manufacturing Example 2

Image bearing member 2 is manufactured in the same manner as in Image Bearing Member Manufacturing Example 1 except that the liquid of application for the intermediate layer used in Image Bearing Member Manufacturing Example 1 is changed to the following component.

#### Liquid of Application for Intermediate Layer

|                                                                                                                        |            |
|------------------------------------------------------------------------------------------------------------------------|------------|
| Surface treated rutile type titanium oxide                                                                             | 112 parts  |
| Alkyd resin (BECKOLITE M6401-50-S, manufactured by Dainippon Ink and Chemicals Incorporated, solid portion: 50%)       | 33.6 parts |
| Melamine resin (SUPERBECAKMINE L-121-60, manufactured by Dainippon Ink and Chemicals Incorporated, solid portion: 60%) | 18.7 parts |
| 2-butanol                                                                                                              | 260 parts  |

The surface treated rutile type titanium oxide is obtained by surface-treating the non-surface treated rutile type titanium oxide used in Image Bearing Member Manufacturing Example 1 with siloxane having 2 weight % based on the weight of the non-surface treated rutile type titanium oxide.

An intermediate layer is formed using the liquid of application mentioned above for intermediate layer on an aluminum board having a thickness of 1 mm in the same manner as described in manufacturing of the image bearing member 1. The spectroscopic reflection spectrum of the intermediate layer is measured by a marketed spectral photometer (UV-3100, manufactured by Shimadzu Corporation). The absorption end (the upper limit of the wavelength of light which can be absorbed therein) of the intermediate layer is obtained from the spectroscopic reflection spectrum. The result of the absorption end of the titanium oxide mentioned above is about 410 nm.

#### Image Bearing Member Manufacturing Example 3

Image bearing member 3 is manufactured in the same manner as in Image Bearing Member Manufacturing Example 1 except that the liquid of application for intermediate layer used in Image Bearing Member Manufacturing Example 1 is changed to the following component.

#### Liquid of Application for Intermediate Layer

|                                                                                                 |           |
|-------------------------------------------------------------------------------------------------|-----------|
| Non-surface treated zinc oxide (SAZEX #2000, manufactured by Sakai Chemical Industry Co., Ltd.) | 112 parts |
|-------------------------------------------------------------------------------------------------|-----------|

120

-continued

|                                                                                                                        |            |
|------------------------------------------------------------------------------------------------------------------------|------------|
| Alkyd resin (BECKOLITE M6401-50-S, manufactured by Dainippon Ink and Chemicals Incorporated, solid portion: 50%)       | 33.6 parts |
| Melamine resin (SUPERBECAKMINE L-121-60, manufactured by Dainippon Ink and Chemicals Incorporated, solid portion: 60%) | 18.7 parts |
| 2-butanol                                                                                                              | 260 parts  |

10 An intermediate layer is formed using the liquid of application mentioned above for intermediate layer on an aluminum board having a thickness of 1 mm in the same manner as described in manufacturing of the image bearing member 3 using the liquid of application for intermediate layer. The spectroscopic reflection spectrum of the intermediate layer is measured by a marketed spectral photometer (UV-3100, manufactured by Shimadzu Corporation). The absorption end (the upper limit of the wavelength of light which can be absorbed therein) of the intermediate layer is obtained from the spectroscopic reflection spectrum. The result of the absorption end of the titanium oxide mentioned above is about 388 nm.

#### Image Bearing Member Manufacturing Example 4

Image bearing member 4 is manufactured in the same manner as in Image Bearing Member Manufacturing Example 1 except that the layer thickness of the charge generating layer in Image Bearing Member Manufacturing Example 1 is changed such that the transmission factor is 12% for light having a wavelength of 407 nm.

#### Image Bearing Member Manufacturing Example 5

35 Image bearing member 5 is manufactured in the same manner as in Image Bearing Member Manufacturing Example 1 except that the layer thickness of the charge generating layer in Image Bearing Member Manufacturing Example 1 is changed such that the transmission factor is 8% for light having a wavelength of 407 nm.

#### Image Bearing Member Manufacturing Example 6

45 Image bearing member 6 is manufactured in the same manner as in Image Bearing Member Manufacturing Example 2 except that the layer thickness of the charge generating layer in Image Bearing Member Manufacturing Example 2 is changed such that the transmission factor is 12% for light having a wavelength of 407 nm.

#### Image Bearing Member Manufacturing Example 7

55 Image bearing member 7 is manufactured in the same manner as in Image Bearing Member Manufacturing Example 2 except that the layer thickness of the charge generating layer in Image Bearing Member Manufacturing Example 2 is changed such that the transmission factor is 8% for light having a wavelength of 407 nm.

#### Image Bearing Member Manufacturing Example 8

60 Image bearing member 8 is manufactured in the same manner as in Image Bearing Member Manufacturing Example 1 except that the charge transport material in Image Bearing Member Manufacturing Example 1 is changed to the material represented by the following chemical structure:



The transmission factor of the charge transport layer in Image Bearing Member Manufacturing Example 8 for light having a wavelength of 407 nm is 40% when measured and evaluated in the same manner as described above.

#### Image Bearing Member Manufacturing Example 9

Image bearing member 9 is manufactured in the same manner as in Image Bearing Member Manufacturing Example 8 except that the liquid of application for the charge transport layer in Image Bearing Member Manufacturing Example 8 is changed to the following receipt:

#### Liquid of Application for Charge Transport Layer

Polycarbonate (TS2050, manufactured by Teijin Chemicals Ltd.) 10 parts  
Charge transport material represented by the following chemical structure 10 parts



The transmission factor of the charge transport layer in Image Bearing Member Manufacturing Example 9 for light having a wavelength of 407 nm is 25% when measured and evaluated in the same manner as described above.

#### Example 1

The image bearing member 1 is implemented in an image forming apparatus as shown in FIG. 9. The irradiation light source is a semi-conductor laser (image writing by a polygon mirror) emitting light having a wavelength of 407 nm. A scorotron charger is used as the charging device. A transfer belt is used as the transfer device. A 380 nm LED, manufactured by Nichia Corporation, is as the discharging light source. The process conditions before the test of 50,000 continuous printing of a chart in which characters corresponding to about 6%

based on the total area of an A4 sheet are uniformly written are set as follows:

Charging device of image bearing member (non-irradiated portion): -900V

Developing bias: -650 V (negative/positive development)  
Surface voltage of irradiated portion by writing light: -120 V

Evaluation is made based on the measurement of the charging voltage of the image bearing member and the voltage at irradiated portion thereof before and after 50,000 image printing. The voltage is measured after 50,000 image printing while fixing the writing condition (amount of irradiation) to the value of the initial stage.

The surface voltage of the non-irradiated portions and irradiated portion at the development portion and the irradiation voltage are measured with a surface voltmeter placed on the developing position shown in FIG. 9 for solid image printing by the semi-conductor laser after -900 V charging on the image bearing member. The result is shown in Table 3.

20

#### Example 2

The evaluation is made in the same manner as in Example 1 except that a 502 nm LED (with a half value width of 15 nm, manufactured by Seiwa Electric Mfg. Co., Ltd.) is used as the discharging device instead of that in Example 1. The result is shown in Table 3.

#### Comparative Example 1

The evaluation is made in the same manner as in Example 2 except that the writing light source of Example 2 is changed to a light source of 440 nm LD (image writing by a polygon mirror). The result is shown in Table 3. The transmission factors of the charge generating layer and the charge transport layer for light having a wavelength of 440 nm are 38% and 98%, respectively.

#### Example 3

The evaluation is made in the same manner as in Example 1 except that the image bearing member 1 is replaced with the image bearing member 2. The result is shown in Table 3.

#### Example 4

The evaluation is made in the same manner as in Example 1 except that the writing light source of Example 1 is changed to a light source of 375 nm LD (image writing by a polygon mirror) and the image bearing member 1 is replaced with the image bearing member 3. The result is shown in Table 3. The transmission factors of the charge generating layer and the charge transport layer for light having a wavelength of 375 nm are 17% and 77%, respectively.

55

#### Comparative Example 2

The evaluation is made in the same manner as in Example 1 except that the image bearing member 1 is replaced with the image bearing member 3. The result is shown in Table 3.

#### Comparative Example 3

The evaluation is made in the same manner as in Comparative Example 1 except that the image bearing member 1 is replaced with the image bearing member 3. The result is shown in Table 3.

**123**

Example 5

The evaluation is made in the same manner as in Example 1 except that the image bearing member **1** is replaced with the image bearing member **4**. The result is shown in Table 3.

Example 6

The evaluation is made in the same manner as in Example 1 except that the image bearing member **1** is replaced with the image bearing member **5**. The result is shown in Table 3.

Example 7

The evaluation is made in the same manner as in Example 1 except that the image bearing member **1** is replaced with the image bearing member **8**. The result is shown in Table 3. The amount of writing light is set such that the voltage at the irradiated portion at the initial stage is the same as that of Example 1.

The evaluation is made in the same manner as in Example 1 except that the image bearing member **1** is replaced with the image bearing member **9**. The result is shown in Table 3. The amount of writing light is set such that the voltage at the irradiated portion at the initial stage is the same as that of Example 1.

10

**124**

Example 8

15 The evaluation is made in the same manner as in Example 3 except that the image bearing member **2** is replaced with the image bearing member **6**. The result is shown in Table 3.

Example 9

20 The evaluation is made in the same manner as in Example 3 except that the image bearing member **2** is replaced with the image bearing member **7**. The result is shown in Table 3.

Example 10

TABLE 3

|             | Writing light wavelength (nm) | Discharging light wavelength (nm) | Initial                                        |                                            | After 50,000 image printing                    |                                            |
|-------------|-------------------------------|-----------------------------------|------------------------------------------------|--------------------------------------------|------------------------------------------------|--------------------------------------------|
|             |                               |                                   | Surface voltage at non-irradiated portion (-V) | Surface voltage at irradiated portion (-V) | Surface voltage at non-irradiated portion (-V) | Surface voltage at irradiated portion (-V) |
| Example 1   | 407                           | 380                               | 900                                            | 120                                        | 900                                            | 135                                        |
| Example 2   | 407                           | 502                               | 900                                            | 120                                        | 900                                            | 150                                        |
| Comparative | 440                           | 502                               | 900                                            | 120                                        | 900                                            | 180                                        |
| Example 1   |                               |                                   |                                                |                                            |                                                |                                            |
| Example 3   | 407                           | 380                               | 900                                            | 120                                        | 900                                            | 150                                        |
| Example 4   | 375                           | 380                               | 900                                            | 125                                        | 900                                            | 140                                        |
| Comparative | 407                           | 380                               | 900                                            | 125                                        | 900                                            | 175                                        |
| Example 2   |                               |                                   |                                                |                                            |                                                |                                            |
| Comparative | 440                           | 502                               | 900                                            | 125                                        | 900                                            | 185                                        |
| Example 3   |                               |                                   |                                                |                                            |                                                |                                            |
| Example 5   | 407                           | 380                               | 900                                            | 110                                        | 900                                            | 125                                        |
| Example 6   | 407                           | 380                               | 900                                            | 105                                        | 900                                            | 145                                        |
| Example 7   | 407                           | 380                               | 900                                            | 120                                        | 900                                            | 150                                        |
| Example 8   | 407                           | 380                               | 900                                            | 120                                        | 900                                            | 165                                        |
| Example 9   | 407                           | 380                               | 900                                            | 120                                        | 900                                            | 150                                        |
| Example 10  | 407                           | 380                               | 900                                            | 120                                        | 900                                            | 155                                        |

## 125

As seen in Table 3, when the wavelength of writing light is set to be shorter than 450 nm and the writing light is absorbed by metal oxide (titanium oxide) contained in the intermediate layer as in Example 1, the rise of the voltage at irradiated portions after repetitive use is relatively small in comparison with that in the case in which the writing light is not absorbed by the metal oxide as in Comparative Example 1. This effect is greater when discharging light is absorbed by the intermediate layer as in Example 1 than when discharging light is not absorbed by the intermediate layer as in Example 2.

The effect of reducing the residual voltage is less when a surface treated titanium oxide is used as in Example 3 than when a non-surface treated titanium oxide is used as in Example 1.

It is found that, when the wavelength of writing light is set to be shorter than 450 nm and the writing light is absorbed by metal oxide (zinc oxide) contained in the intermediate layer as in Example 1, the rise of the voltage at irradiated portions after repetitive use is relatively small in comparison with that in the cases in which the writing light is not absorbed by the metal oxide as in Comparative Examples 2 and 3.

It is also found that when the transmission factor of the charge generating layer for the writing light is less than 10% as in Examples 6 and 10, the rise of the voltage at irradiated portions after repetitive use is relatively large in comparison with those in the cases in which the transmission factor thereof is not less than 10% as in Examples 1 and 5 and Comparative Examples 3 and 9.

It is also found that when the transmission factor of the charge transport layer for the discharging light is less than 30% as in Example 8, the rise of the voltage at irradiated portions after repetitive use is relatively large in comparison with those in the cases in which the transmission factor thereof is not less than 30% as in Examples 1 and 7.

## Example 11

The test of Example 11 is performed in the same manner as in Example 1 except that a chart shown in FIG. 14 having a white solid portion and a black solid portion which are divided from each other at the center of an A4 sheet in the longitudinal direction of the image bearing member is used instead of the chart in which characters corresponding to about 6% based on the total area of an A4 sheet. The voltages at the irradiated portion of the white solid portion and the black solid portion are measured after 50,000 printing. The results are shown in Table 4.

## Example 12

The test of Example 12 is performed in the same manner as in Example 2 except that a chart shown in FIG. 14 having a white solid portion and a black solid portion which are divided from each other at the center of an A4 sheet in the longitudinal direction of the image bearing member is used instead of the chart in which characters corresponding to about 6% based on the total area of an A4 sheet. The voltages at the irradiated portion of the white solid portion and the black solid portion are measured after 50,000 printing. The results are shown in Table 4.

TABLE 4

| Writing light wavelength (nm) | Discharging light wavelength (nm) | After 50,000 printing                                     |                                                           |
|-------------------------------|-----------------------------------|-----------------------------------------------------------|-----------------------------------------------------------|
|                               |                                   | Voltage at irradiated portion of white solid portion (-V) | Voltage at irradiated portion of black solid portion (-V) |
| Example 11                    | 407                               | 380                                                       | 135                                                       |
| Example 12                    | 407                               | 502                                                       | 155                                                       |

## 126

As seen in Table 4, when discharging light is absorbed by the metal oxide (titanium oxide) contained in the intermediate layer (as in Example 11) and an original having portions having an extremely large difference in image density as shown in FIG. 14 is used, there is no significant difference between the voltages at the irradiated portions.

However, when discharging light is not absorbed by the metal oxide (titanium oxide) contained in the intermediate layer (as in Example 12), there is a large difference between the voltages at the white solid portion and the black solid portion.

## Image Bearing Member Manufacturing Example 10

Image bearing member 10 is manufactured in the same manner as in Image Bearing Member Manufacturing Example 1 except that the liquid dispersion 2 is used as the liquid of application for charge generating layer. The layer thickness of the charge generating layer is adjusted such that the transmission factor thereof for writing light having a wavelength of 407 nm is 20%.

## Image Bearing Member Manufacturing Example 11

Image bearing member 11 is manufactured in the same manner as in Image Bearing Member Manufacturing Example 1 except that the liquid dispersion 3 is used as the liquid of application for charge generating layer. The layer thickness of the charge generating layer is adjusted such that the transmission factor thereof for writing light having a wavelength of 407 nm is 20%.

## Image Bearing Member Manufacturing Example 12

Image bearing member 12 is manufactured in the same manner as in Image Bearing Member Manufacturing Example 1 except that the liquid dispersion 4 is used as the liquid of application for charge generating layer. The layer thickness of the charge generating layer is adjusted such that the transmission factor thereof for writing light having a wavelength of 407 nm is 20%.

## Example 13

The evaluation is made in the same manner as in Example 1 except that the image bearing member 10 is used instead of the image bearing member 1. The background fouling is evaluated for white solid image output after 50,000 image outputs. The result is shown in Table 5 with those of Example 1.

## Example 14

The evaluation is made in the same manner as in Example 1 except that the image bearing member 11 is used instead of the image bearing member 1. The background fouling is evaluated for white solid image output after 50,000 image outputs. The result is shown in Table 5.

## Example 15

The evaluation is made in the same manner as in Example 1 except that the image bearing member 12 is used instead of the image bearing member 1. The background fouling is evaluated for white solid image output after 50,000 image outputs. The result is shown in Table 5.

The background fouling is evaluated with scaling by the number and the size of black spots on the background portion.

The scaling is from 1 to 4, in which "excellent" is rated as E, "good" is rated as G, "fair" is rated as F and "bad" is rated as B.

TABLE 5

|            | Initial                                                 |                                                     | After 50,000 image printing                             |                                                     | Background<br>fouling<br>evaluation |
|------------|---------------------------------------------------------|-----------------------------------------------------|---------------------------------------------------------|-----------------------------------------------------|-------------------------------------|
|            | Surface<br>voltage at<br>non-irradiated<br>portion (-V) | Surface<br>voltage at<br>irradiated<br>portion (-V) | Surface<br>voltage at<br>non-irradiated<br>portion (-V) | Surface<br>voltage at<br>irradiated<br>portion (-V) |                                     |
| Example 1  | 900                                                     | 120                                                 | 900                                                     | 135                                                 | F or G                              |
| Example 13 | 900                                                     | 110                                                 | 900                                                     | 120                                                 | E                                   |
| Example 14 | 900                                                     | 110                                                 | 900                                                     | 120                                                 | E                                   |
| Example 15 | 900                                                     | 110                                                 | 900                                                     | 125                                                 | G                                   |

As seen in Table 5, it is found that, when the average particle diameter in the liquid of application for charge generating layer is not greater than 0.25  $\mu\text{m}$  as in Examples 13 to 15, the surface voltage at the irradiated portion in the initial state of the image bearing member can be reduced and the occurrence of background fouling can be restrained after repetitive use without having an adverse impact on the rise of the irradiated portions.

#### Image Bearing Member Manufacturing Example 13

15 charge transport layer is set to be 23  $\mu\text{m}$  and the liquid of application for protective layer having the following receipt is coated and dried on the charge transport layer to obtain a protective layer having a thickness of 2  $\mu\text{m}$ . The transmission factor of the protective layer formed not on the image bearing member but on polyethylene terephthalate film is measured by spectroscopic photometer at 407 nm. The result of the transmission factor is 98%. The transmission factor of the charge transport layer is 98%.

25

Image bearing member **13** is manufactured in the same manner as in Example 1 except that the layer thickness of the

#### Liquid of Application for Protective Layer

Polycarbonate (TS2050, manufactured by Teijin Chemicals Ltd.)

10 parts

Charge transport material represented by the following chemical structure:

7 parts



Aluminum particulates (specific resistance:  $2.5 \times 10^{12} \Omega \cdot \text{cm}$ , average primary particle

4 parts

diameter: 0.4  $\mu\text{m}$ )

Cyclohexanone

500 parts

Tetrahydrofuran

150 parts

## 129

## Image Bearing Member Manufacturing Example 14

Image bearing member **14** is manufactured in the same manner as in Image Bearing Member Manufacturing Example 13 except that the aluminum particulates in the liquid of application for protective layer in Image Bearing Member Manufacturing Example 13 is changed to the following. The transmission factor of the protective layer for light having a wavelength of 407 nm is 95%.

Titanium oxide particulate (specific resistance:  $1.5 \times 10^{10} \Omega \cdot \text{cm}$ , average primary particle diameter:  $0.5 \mu\text{m}$ ) 4 parts

## Image Bearing Member Manufacturing Example 15

Image bearing member **15** is manufactured in the same manner as in Image Bearing Member Manufacturing Example 13 except that the aluminum particulates in the liquid of application for protective layer in Image Bearing

5

Member Manufacturing Example 13 is changed to the following. The transmission factor of the protective layer for light having a wavelength of 407 nm is 93%.

## 10 Image Bearing Member Manufacturing Example 16

Image bearing member **16** is manufactured in the same manner as in Image Bearing Member Manufacturing Example 13 except that the liquid of application for protective layer in Image Bearing Member Manufacturing Example 13 is changed to the following. The transmission factor of the protective layer for light having a wavelength of 407 nm is 90%.

15

## 20 Liquid of Application for Protective Layer

Charge transport material represented by the following chemical

17 parts

structure: (weight average molecular weight: about 140,000)

Aluminum particulates (specific resistance:  $2.5 \times 10^{12} \Omega \cdot \text{cm}$ , average primary particle

4 parts

diameter:  $0.4 \mu\text{m}$ )

Cyclohexanone

500 parts

Tetrahydrofuran

150 parts

## 131

## Image Bearing Member Manufacturing Example 17

Image bearing member **17** is manufactured in the same manner as in Image Bearing Member Manufacturing Example 13 except that the aluminum particulates in the

## 132

liquid of application for protective layer in Image Bearing Member Manufacturing Example 19 is changed to the following. The transmission factor of the protective layer for light having a wavelength of 407 nm is 38%.

## Liquid of Application for Protective Layer

|                                                                            |           |
|----------------------------------------------------------------------------|-----------|
| Methyltrimethoxysilane                                                     | 100 parts |
| 3% acetic acid                                                             | 20 parts  |
| Charge transport material represented by the following chemical structure: |           |



|                                                                                    |           |
|------------------------------------------------------------------------------------|-----------|
| Anti-oxidant agent (SANOL LS2626, manufactured by Sankyo Unite Industry Co., Ltd.) | 1 part    |
| Curing agent (dibutyl tin acetate)                                                 | 1 part    |
| 2-propanol                                                                         | 200 parts |

Image bearing member **18** is manufactured in the same manner as in Image Bearing Member Manufacturing Example 13 except that the liquid of application for protective layer in Image Bearing Member Manufacturing Example 13 is changed to the following. The transmission factor of the protective layer for light having a wavelength of 407 nm is 38%.

## Liquid of Application for Protective Layer

|                                                                            |           |
|----------------------------------------------------------------------------|-----------|
| Methyltrimethoxysilane                                                     | 100 parts |
| 3% acetic acid                                                             | 20 parts  |
| Charge transport material represented by the following chemical structure: |           |

|                                                                            |          |
|----------------------------------------------------------------------------|----------|
| Charge transport material represented by the following chemical structure: | 35 parts |
|----------------------------------------------------------------------------|----------|



|                                                                                                                                                 |           |
|-------------------------------------------------------------------------------------------------------------------------------------------------|-----------|
| Aluminum particulates (specific resistance: $25 \times 10^{12} \Omega \cdot \text{cm}$ , average primary particle diameter: $0.4 \mu\text{m}$ ) | 15 parts  |
| Anti-oxidant agent (SANOL LS2626, manufactured by Sankyo Unite Industry Co., Ltd.)                                                              | 1 part    |
| Polycarbonate compound (BYK P104, manufactured by Byk Chemie)                                                                                   | 0.4 parts |
| Curing agent (dibutyl tin acetate)                                                                                                              | 1 part    |
| 2-propanol                                                                                                                                      | 200 parts |

## 133

Image Bearing Member Manufacturing Example 19

Image bearing member **18** is manufactured in the same manner as in Image Bearing Member Manufacturing Example 13 except that the liquid of application for protective layer in Image Bearing Member Manufacturing Example 13

## 134

is changed to the following. The transmission factor of the protective layer for light having a wavelength of 407 nm is 74%.

5

Liquid of Application for Protective Layer

Radical polymerizable monomer having at least 3 functional

10 parts

groups which does not have a charge transport structure (trimethylol

propane triacrylate: KAYARAD TAMPTA, manufactured by Nippon Kayaku

Co., Ltd.) (molecular weight: 296, number of functional groups: 3,

molecular weight/number of functional groups: 99)

Radical polymerizable compound having a functional group and

10 parts

a charge transport structure representd by the following chemical  
strucutre: (No. 54 compound illustrated above)

Optical polymerization initiator

1 part

(1-hydroxy-cyclohexyl-phenyl-ketone: ILUGACURE 184, manufactured by

Ciba Specialty Chemicals)

Tetrahydrofuran

100 parts

## 135

The protective layer is cured after 20 minute natural drying after spraying coating by irradiation under the condition of metal halide lamp: 160 W/cm, irradiation intensity: 500 mW/cm<sup>2</sup> and irradiation time: 60 seconds.

## Image Bearing Member Manufacturing Example 20

Image bearing member **20** is manufactured in the same manner as in Image Bearing Member Manufacturing Example 19 except that the radical polymerizable monomer having at least 3 functional groups which does not have a charge transport structure is changed to the following radical polymerizable monomer. The transmission factor of the protective layer for light having a wavelength of 407 nm is 73%.

Radical polymerizable monomer having at least 3 functional groups which does not have a charge transport structure (penta erythritol tetraacrylate, SR-295, manufactured by Sartomer Company Inc.) (molecular weight: 352, number of functional groups: 4, molecular weight/number of functional groups: 88) 10 parts

## Image Bearing Member Manufacturing Example 21

Image bearing member **21** is manufactured in the same manner as in Image Bearing Member Manufacturing Example 19 except that the radical polymerizable monomer having at least 3 functional groups which does not have a charge transport structure is changed to the following radical polymerizable monomer having two functional groups which does not have a charge transport structure. The transmission factor of the protective layer for light having a wavelength of 407 nm is 74%.

Radical polymerizable monomer having two functional groups which does not have a charge transport structure (1,6-hexanediol diacrylate, manufactured by Wako Pure Chemical Industries, Ltd.) (molecular weight: 226, number of functional groups: 2, molecular weight/number of functional groups: 113) 10 parts

## Image Bearing Member Manufacturing Example 22

Image bearing member **22** is manufactured in the same manner as in Image Bearing Member Manufacturing Example 19 except that the radical polymerizable monomer having at least 3 functional groups which does not have a charge transport structure is changed to the following radical polymerizable monomer. The transmission factor of the protective layer is 71%.

## 136

Radical polymerizable monomer having at least 3 functional groups which does not have a charge transport structure (caprolactone modified dipenta erythritol hexaacrylate (KAYARAD DPCA-120, manufactured by Nippon Kayaku Co., Ltd.)(molecular weight: 1,947, number of functional groups: 6, molecular weight/number of functional groups: 325) 10 parts

## Image Bearing Member Manufacturing Example 23

Image bearing member **23** is manufactured in the same manner as in Image Bearing Member Manufacturing Example 19 except that the Radical polymerizable compound having a functional group and a charge transport structure is changed to the radical polymerizable monomer having two functional groups and a charge transport structure represented by the following chemical structure. The transmission factor of the protective layer for light having a wavelength of 407 nm is 3%.



## Image Bearing Member Manufacturing Example 24

Image bearing member **24** is manufactured in the same manner as in Image Bearing Member Manufacturing Example 19 except that the liquid of application for protective layer is changed to the following receipe The transmission factor of the protective layer for light having a wavelength of 407 nm is 72%.

## Liquid of Application for Protective Layer

Radical polymerizable monomer having at least 3 functional

6 parts

groups which does not have a charge transport structure (trimethylol

propane triacrylate: KAYARAD TAMPTA, manufactured by Nippon Kayaku

Co., Ltd.) (molecular weight: 296, number of functional groups: 3,

molecular weight/number of functional groups: 99)

Radical polymerizable compound having a functional group and

14 parts

a charge transport structure representd by the following chemical

strucutre: (No. 54 compound illustrated above)

-continued



Optical polymerization initiator  
(1-hydroxy-cyclohexyl-phenyl-ketone: ILUGACURE 184, manufactured by  
Ciba Specialty Chemicals)  
Tetrahydrofuran

1 part

100 parts

## Image Bearing Member Manufacturing Example 25

Image bearing member **25** is manufactured in the same manner as in Image Bearing Member Manufacturing Example 19 except that the liquid of application for protective

<sup>30</sup> layer is changed to the following receipe The transmission factor of the protective layer for light having a wavelength of 407 nm is 72%.

## Liquid of Application for Protective Layer

Radical polymerizable monomer having at least 3 functional groups which does not have a charge transport structure (trimethylol propane triacrylate: KAYARAD TAMPTA, manufactured by Nippon Kayaku Co., Ltd.) (molecular weight: 296, number of functional groups: 3, molecular weight/number of functional groups: 99)

14 parts

Radical polymerizable compound having a functional group and a charge transport structure representd by the following chemical strucuture: (No. 54 compound illustrated above)

6 parts



139

-continued

Optical polymerization initiator  
(1-hydroxy-cyclohexyl-phenyl-ketone: ILUGACURE 184, manufactured by  
Ciba Specialty Chemicals)  
Tetrahydrofuran

1 part

100 parts

## Image Bearing Member Manufacturing Example 26

Image bearing member **26** is manufactured in the same manner as in Image Bearing Member Manufacturing Example 19 except that the liquid of application for protective layer is changed to the following receipe The transmission factor of the protective layer for light having a wavelength of 407 nm is 74%.

## Liquid of Application for Protective Layer

Radical polymerizable monomer having at least 3 functional groups which does not have a charge transport structure (trimethylol propane triacrylate: KAYARAD TAMPTA, manufactured by Nippon Kayaku Co., Ltd.) (molecular weight: 296, number of functional groups: 3, molecular weight/number of functional groups: 99)  
Radical polymerizable compound having a functional group and a charge transport structure representd by the following chemical strucuture:  
(No. 54 compound illustrated above)

2 parts



Optical polymerization initiator (1-hydroxy-cyclohexyl-phenyl-ketone: ILUGACURE 184, manufactured by  
Ciba Specialty Chemicals)  
Tetrahydrofuran

18 parts

30

35

40

45

50

55

60

65

## Liquid of Application for Protective Layer

10

Radical polymerizable monomer having at least 3 functional groups which does not have a charge transport structure (trimethylol propane triacrylate: KAYARAD TAMPTA, manufactured by Nippon Kayaku Co., Ltd.) (molecular weight: 296, number of functional groups: 3, molecular weight/number of functional groups: 99)

18 parts

Radical polymerizable compound having a functional group and a charge transport structure representd by the following chemical strucuture: (No. 54 compound illustrated above)

2 parts



Optical polymerization initiator (1-hydroxy-cyclohexyl-phenyl-ketone: ILUGACURE 184, manufactured by  
Ciba Specialty Chemicals)  
Tetrahydrofuran

1 part

100 parts

## Example 16

50 The image bearing member **1** is implemented in an image forming apparatus as shown in FIG. 9. The irradiation light source is a semi-conductor laser (image writing by a polygon mirror) emitting light having a wavelength of 407 nm. A scorotron charger is used as the charging device. A transfer belt is used as the transfer device. The process conditions before the test of 70,000 continuous printing of a chart having a writing ratio of 6% are as follows.

Charging device of image bearing member (non-irradiated portion): -900V

60 Developing bias: -650 V (negative/positive development)

Surface voltage at irradiated portion: -120 V

Discharging light: Make homogeneous light having a wavelength of 405 nm by combining a Xenon lamp with a spectroscope and guide the light to the image forming apparatus with optical fiber to irradiate the surface of the image bearing member therewith through slits.

## Image Bearing Member Manufacturing Example 27

Image bearing member **27** is manufactured in the same manner as in Image Bearing Member Manufacturing Example 19 except that the liquid of application for protective layer is changed to the following receipe The transmission factor of the protective layer for light having a wavelength of 407 nm is 73%.

## Evaluation Items

## (1) Surface Voltage

Evaluation is made based on the measurement of the voltage at irradiated portion on the image bearing member before and after the 70,000 image printing.

The voltage is measured after 70,000 image printing while fixing the writing condition (amount of irradiation) to the value of the initial stage.

The voltage at irradiated portion in the development portion is measured for solid printing by the semi-conductor laser after -900 V charging on the image bearing member with a surface voltmeter placed on the developing position shown in FIG. 9. The result is shown in Table 6.

## (2) Background Fouling

The background fouling is evaluated for white solid image output after the 70,000 image outputs (after measuring the surface voltage) at 22° C. and 50% RH. The background fouling is evaluated as the 4 rank scaling mentioned above. The result is shown in Table 6.

written is output). The 1 dot image is observed by an optical microscope and the clearness of the dot contour is evaluated by 4 rank scaling as follows: Excellent represented by E; Good represented by G; Fair represented by F; and Poor represented by P. The result is shown in Table 6.

## (5) Amount of Abrasion

The layer thickness of the image bearing member at the initial state is measured and again measured after all the tests of (1) to (4). The differences (amount of abrasion) between the layer thickness before and after the tests are evaluated. The layer thickness is measured with an interval of 1 cm except for 5 cm from both ends in the longitudinal direction of the image bearing member and the average is determined as the layer thickness.

15

## Examples 17 to 31

The image bearing members 13 to 27 as manufactured above are evaluated under the same conditions as in Example 16. The results are shown in Table 6. The numbers of the image bearing members corresponding to the numbers of Examples are also shown in Table 6.

TABLE 6

| Number<br>of image<br>bearing<br>member | Voltage at irradiated<br>portion (-V) |                                   |                                     |                                    |                                     |                               |
|-----------------------------------------|---------------------------------------|-----------------------------------|-------------------------------------|------------------------------------|-------------------------------------|-------------------------------|
|                                         | Initial                               | After<br>70,000<br>image<br>print | Background<br>fouling<br>evaluation | Cleaning<br>property<br>evaluation | Dot<br>representation<br>evaluation | Amount of<br>abrasion<br>(μm) |
| Example 16                              | 1                                     | 120                               | 145                                 | F                                  | G                                   | E                             |
| Example 17                              | 13                                    | 125                               | 155                                 | E                                  | F or G                              | E or G                        |
| Example 18                              | 14                                    | 130                               | 160                                 | E                                  | F or G                              | G                             |
| Example 19                              | 15                                    | 120                               | 150                                 | G                                  | F or G                              | F or G                        |
| Example 20                              | 16                                    | 130                               | 155                                 | E                                  | F or G                              | G                             |
| Example 21                              | 17                                    | 130                               | 155                                 | E or G                             | G                                   | 3.4                           |
| Example 22                              | 18                                    | 135                               | 160                                 | E                                  | F or G                              | F or G                        |
| Example 23                              | 19                                    | 130                               | 155                                 | E                                  | E                                   | 1.9                           |
| Example 24                              | 20                                    | 130                               | 155                                 | G                                  | E                                   | 1.6                           |
| Example 25                              | 21                                    | 130                               | 155                                 | E                                  | F or G                              | 3.5                           |
| Example 26                              | 22                                    | 130                               | 155                                 | E                                  | E                                   | 1.9                           |
| Example 27                              | 23                                    | 160                               | 185                                 | E                                  | F or G                              | E                             |
| Example 28                              | 24                                    | 125                               | 150                                 | E or G                             | E                                   | 2.1                           |
| Example 29                              | 25                                    | 135                               | 160                                 | E                                  | E                                   | 1.9                           |
| Example 30                              | 26                                    | 120                               | 145                                 | E or G                             | E                                   | 2.4                           |
| Example 31                              | 27                                    | 140                               | 160                                 | E                                  | E                                   | 1.9                           |

## (3) Cleaning Property

After the evaluation of the background fouling, 50 test charts as illustrated in FIG. 15 are continuously printed in the direction from the black solid portion to the white solid portion under the same condition as in Example 1 at a low temperature (10° C.) and a low humidity (15% RH) for evaluating cleaning property. The white solid portion of the 50th image is observed with naked eyes. The evaluation is made with the 4 rank scaling as follows: Excellent (no bad cleaning performance) represented by E; Good (one or two black streaks are slightly observed in the longitudinal direction) represented by G; Fair (three or four black streaks are slightly observed in the longitudinal direction) represented by F; and Poor (clear black streaks are observed) represented by P. The result is shown in Table 6.

## (4) Dot Representation

After the cleaning property evaluation, 1,000 images of the test charts having a writing ratio of 6% are output at a high temperature 30° C.) and a high humidity (90% RH) for 1 dot image evaluation (an image in which an independent dot is

The following is seen in Table 6.

Even when a protective layer is formed, the rise of the residual voltage is prevented by absorption for light having a wavelength of 407 nm by the titanium oxide contained in the intermediate layer.

The anti-abrasion property is improved in cases in which a protective layer is provided as in Examples 17 to 31 in comparison with cases in which a protective layer is not provided as in Example 16.

Among the cases in which the protective layer containing an inorganic pigment (metal oxide) is provided as in Examples 17 to 19, the dot representation is not significantly decreased at a high temperature and a high humidity when the inorganic pigment has a specific resistance of not less than  $10^{10} \Omega \cdot \text{cm}$  as in Examples 18 and 19.

The anti-abrasion property is relatively improved by a protective layer having a cross linking structure in comparison with a protective layer without a cross linking structure. A protective layer formed by curing a radical polymerizable monomer having at least 3 functional groups which does not

## 143

have a charge transport structure and a radical polymerizable compound having a functional group and a charge transport structure can improve the anti-abrasion property as in Examples 20, 23, 26, and 28 to 31.

In addition, the cleaning property can be improved by using a protective layer formed by curing a radical polymerizable monomer having at least 3 functional groups which does not have a charge transport structure and a radical polymerizable compound having a functional group and a charge transport structure.

## Example 32

The voltage at the irradiated portion is measured and the evaluation is made in the same manner as in Example 26 except that a 502 nm LED with a half value width of 15 nm (manufactured by Seiwa Electric Mfg. Co., Ltd.) is used instead. The amount of discharging light is adjusted such that the surface voltage of the image bearing member after discharging is the same as in Example 26. The result is shown in Table 7 accompanied by the result of Example 26. The transmission factors of the charge generating layer and the charge transport layer for writing light for the image bearing member having a wavelength of 407 nm are 20% and 98%, respectively.

## Comparative Example 4

The evaluation is made in the same manner as in Example 32 except that a 440 nm LD (image writing by a polygon mirror) is used instead. The amount of writing light is adjusted such that the surface voltage at the irradiated portion at the initial stage is equal to that of Example 32. The result is shown in Table 7. The transmission factors of the charge generating layer and the charge transport layer for writing light for the image bearing member having a wavelength of 440 nm are 38% and 98%, respectively.

## 144

Example 26 than when discharging light is not absorbed by the intermediate layer as in Example 32.

## Image Bearing Manufacturing Example 28

Image bearing member **28** is manufactured in the same manner as in Image Bearing Member Manufacturing Example 22 except that the layer thickness of the protective layer is changed to 2.2  $\mu\text{m}$ .

## Image Bearing Manufacturing Example 29

Image bearing member **29** is manufactured in the same manner as in Image Bearing Member Manufacturing Example 22 except that the layer thickness of the protective layer is changed to 4.1  $\mu\text{m}$ .

## Example 33

The image bearing member **22** is implemented in an image forming apparatus as shown in FIG. 9. The irradiation light source is a semi-conductor laser (image writing by a polygon mirror) emitting light having a wavelength of 407 nm. A scortron charger is used as the charging device. A transfer belt is used as the transfer device. The following is used as the discharging light source. The process conditions before the test of 70,000 continuous printing of a chart having a writing ratio of 6% are set as follows.

Charging device of image bearing member (non-irradiated portion): -900V

Developing bias: -650 V (negative/positive development)

Surface voltage at irradiated portion: -130 V

Discharging light: Make homogeneous light having a wavelength of 409 nm by combining a Xenon lamp with a spectroscope and guide the light to the image forming apparatus with optical fiber to irradiate the surface of the image bearing member therewith through slits.

TABLE 7

|             | Initial    |             |                |              |                |              | After 70,000 printing |  |
|-------------|------------|-------------|----------------|--------------|----------------|--------------|-----------------------|--|
|             | Writing    | Discharging | Surface        | Surface      | Surface        | Surface      |                       |  |
|             | light      | light       | voltage at     | voltage at   | voltage at     | voltage at   |                       |  |
|             | wavelength | wavelength  | non-irradiated | irradiated   | non-irradiated | irradiated   |                       |  |
|             | (nm)       | (nm)        | portion (-V)   | portion (-V) | portion (-V)   | portion (-V) |                       |  |
| Example 26  | 407        | 405         | 900            | 130          | 900            | 155          |                       |  |
| Example 32  | 407        | 502         | 900            | 130          | 900            | 170          |                       |  |
| Comparative | 440        | 502         | 900            | 130          | 900            | 190          |                       |  |
| Example 4   |            |             |                |              |                |              |                       |  |

As seen in Table 7, when the wavelength of writing light is set to be shorter than 450 nm and the writing light is absorbed by metal oxide (titanium oxide) contained in the intermediate layer as in Example 26, the rise of the voltage at irradiated portions after repetitive use is relatively small in comparison with that in the case in which the writing light is not absorbed by the metal oxide as in Comparative Example 4 even when a protective layer is provided. This effect is greater when discharging light is absorbed by the intermediate layer as in

Evaluation is made based on the measurement of the charging voltage of the image bearing member and the voltage at irradiated portion thereof before and after 70,000 image printing. The voltage is measured after 70,000 image printing while fixing the writing condition (amount of irradiation) to the value of the initial stage.

The surface voltage of the non-irradiated portions and the irradiated portion at the development portion are measured for solid printing by the semi-conductor laser after -900 V

## 145

charging on the image bearing member with a surface voltmeter placed on the developing position shown in FIG. 9. The result is shown in Table 8.

In addition, after measuring the voltage after 70,000 image outputs, the image of the chart shown in FIG. 14 in which the front end half is a stripe image and the rear end half is a halftone image is output and non-uniformity of the image on the halftone portion is observed.

To measure the transmission factor of a protective layer, the protective layers of the image bearing members 28 and 29 are formed under the same conditions as described in the cases of the image bearing members 22 and 23 on an aluminum drum having a diameter of 30 mm around which polyethylene terephthalate film is wound. This material is cut to a suitable size and the spectroscopic transmission factor in the range of from 500 to 300 nm is measured by using a marketed spectral photometer (UV-3100, manufactured by Shimadzu Corporation) while comparing with polyethylene terephthalate on which a liquid for protective layer is not coated. The transmission factor of the charge generating layer for writing light having a wavelength of 407 nm is 20% and the transmission factor of the charge transport layer is 98% for discharging light for the image bearing member.

## Example 34

The evaluation is made in the same manner as in Example 33 except that the image bearing member 28 is replaced with the image bearing member 29. The result is shown in Table 8. The transmission factor of the charge generating layer and the charge transport layer is 20% and 98% for writing light having a wavelength of 407 nm.

## Example 35

The evaluation is made in the same manner as in Example 33 except that the writing light source is changed to a light source of 380 nm LD (image writing by a polygon mirror). The amount of light is adjusted to have the same amount as that in the initial stage of Example 33. The result is shown in Table 8. The transmission factors of the charge generating layer and the charge transport layer for writing light having a wavelength of 380 nm are 20% and 98%, respectively.

## Example 36

The evaluation is made in the same manner as in Example 34 except that the writing light source is changed to a light source of 380 nm LD (image writing by a polygon mirror). The result is shown in Table 8. The transmission factors of the charge generating layer and the charge transport layer for writing light having a wavelength of 380 nm are 20% and 98%, respectively.

TABLE 8

| Wavelength of writing light (nm) | Transmission factor of protective layer for writing light (%) | Surface voltage at irradiated portions (-V) |                           |
|----------------------------------|---------------------------------------------------------------|---------------------------------------------|---------------------------|
|                                  |                                                               | Initial                                     | After 50,000 image output |
| Example 33                       | 407                                                           | 79                                          | 130 155                   |
| Example 34                       | 407                                                           | 72                                          | 130 155                   |
| Example 35                       | 380                                                           | 29                                          | 130 160                   |
| Example 36                       | 380                                                           | 10                                          | 130 160                   |

## 146

As seen in Table 8, when the transmission factor of the protective layer for the discharging light is less than 30%, the effect slightly deteriorates.

In addition, the half tone portion in the output of the chart illustrated in FIG. 16 for Examples 33 and 34 is properly formed but a slight residual image corresponding to the stripe in the half tone is recognized in Examples 35 and 36. The degree of the residual image is worse in Example 36 than in Example 35.

Based on the results, it is found that it is possible to restrain the rise of the residual voltage after repetitive use by the absorption of the discharging light having a wavelength shorter than 410 nm by the titanium oxide contained in the intermediate layer. However, it is also found that, when the transmission factor of the protective layer for the writing light is less than 30%, a slight side effect may appear.

## Image Bearing Member Manufacturing Example 30

Image bearing member 30 is manufactured in the same manner as in Image Bearing Member Manufacturing Example 1 except that the intermediate layer in the Image Bearing Member Manufacturing Example 1 is changed to a layered structure having a charge blocking layer and a moiré prevention layer, and a liquid of application having the following recipe for the charge blocking layer and for the moiré prevention layer are applied and dried such that the layer thickness of the charge blocking layer and of the moiré prevention layer are 1.0  $\mu\text{m}$  and 3.5  $\mu\text{m}$ , respectively.

## Liquid of Application for Charge Blocking Layer

|                                                                                                         |          |
|---------------------------------------------------------------------------------------------------------|----------|
| N-methoxy methylated nylon (FINERESIN FR-101, manufactured by Namariichi Chemical Industrial Co., Ltd.) | 4 parts  |
| Methanol                                                                                                | 70 parts |
| n-butanol                                                                                               | 30 parts |

## Liquid of Application for Moire Layer

|                                                                                                                                                               |            |
|---------------------------------------------------------------------------------------------------------------------------------------------------------------|------------|
| Non-surface treated rutile type titanium oxide having an average particle diameter of 0.25 $\mu\text{m}$ (CR-EL, manufactured by Ishihara Industry Co., Ltd.) | 126 parts  |
| Alkyd resin (BECKOLITE M6401-50-S, manufactured by Dainippon Ink and Chemicals Incorporated, solid portion: 50%)                                              | 33.6 parts |
| Melamine resin (SUPERBECAKMINE L-121-60, manufactured by Dainippon Ink and Chemicals Incorporated, solid portion: 60%)                                        | 18.7 parts |
| 2-butanone                                                                                                                                                    | 100 parts  |

The volume ratio of the inorganic pigment to the binder resin is 1.5/1 in the composition.

## Image Bearing Member Manufacturing Example 31

Image bearing member 31 is manufactured in the same manner as in Image Bearing Member Manufacturing Example 30 except that the layer thickness of the charge blocking layer is changed to 0.3  $\mu\text{m}$ .

## 147

## Image Bearing Member Manufacturing Example 32

Image bearing member **32** is manufactured in the same manner as in Image Bearing Member Manufacturing Example 30 except that the layer thickness of the charge blocking layer is changed to 1.8  $\mu\text{m}$ .

## Image Bearing Member Manufacturing Example 33

Image bearing member **33** is manufactured in the same manner as in Image Bearing Member Manufacturing Example 30 except that the liquid of application for the charge blocking layer is changed to have the following receipt.

## Liquid of Application for Charge Blocking Layer

|                                                                               |          |
|-------------------------------------------------------------------------------|----------|
| Alcohol soluble nylon (AMILAN CM8000, manufactured by Toray Industries, Inc.) | 4 parts  |
| Methanol                                                                      | 70 parts |
| n-butanol                                                                     | 30 parts |

## Image Bearing Member Manufacturing Example 34

Image bearing member **34** is manufactured in the same manner as in Image Bearing Member Manufacturing Example 30 except that the liquid of application for the moiré prevention layer is changed to have the following receipt.

## Liquid of Application for Moire Prevention Layer

|                                                                                                                                                               |            |
|---------------------------------------------------------------------------------------------------------------------------------------------------------------|------------|
| Non-surface treated rutile type Titanium oxide having an average particle diameter of 0.25 $\mu\text{m}$ (CR-EL, manufactured by Ishihara Industry Co., Ltd.) | 252 parts  |
| Alkyd resin (BECKOLITE M6401-50-S, manufactured by Dainippon Ink and Chemicals Incorporated, solid portion: 50%)                                              | 33.6 parts |
| Melamine resin (SUPERBECAKMINE L-121-60, manufactured by Dainippon Ink and Chemicals Incorporated, solid portion: 60%)                                        | 18.7 parts |
| 2-butanone                                                                                                                                                    | 100 parts  |

## 148

The volume ratio of the inorganic pigment to the binder resin is 3/1 in the composition.

The weight ratio of the alkyd resin to the melamine resin is 6/4.

## Image Bearing Member Manufacturing Example 35

Image bearing member **35** is manufactured in the same manner as in Image Bearing Member Manufacturing Example 30 except that the liquid of application for the moiré prevention layer is changed to have the following receipt.

## Liquid of Application for Moire Prevention Layer

|                                                                                                                                                               |            |
|---------------------------------------------------------------------------------------------------------------------------------------------------------------|------------|
| Non-surface treated rutile type titanium oxide having an average particle diameter of 0.25 $\mu\text{m}$ (CR-EL, manufactured by Ishihara Industry Co., Ltd.) | 84 parts   |
| Alkyd resin (BECKOLITE M6401-50-S, manufactured by Dainippon Ink and Chemicals Incorporated, solid portion: 50%)                                              | 33.6 parts |
| Melamine resin (SUPERBECAKMINE L-121-60, manufactured by Dainippon Ink and Chemicals Incorporated, solid portion: 60%)                                        | 18.7 parts |
| 2-butanone                                                                                                                                                    | 100 parts  |

The volume ratio of the inorganic pigment to the binder resin is 1/1 in the composition.

The weight ratio of the alkyd resin to the melamine resin is 6/4.

## Examples 37 to 42

70,000 image continuous printing is performed using the image bearing members 30 to 35 under the same condition as in Example 16. The evaluation is made in the same manner for the same items. The results are shown in Table 9 in comparison with the results of Example 16. The transmission factors of the charge generating layer and the charge transport layer for writing light having a wavelength of 407 nm in each Example are 20% and 98%, respectively.

TABLE 9

| Number<br>of image<br>bearing<br>member | Voltage at irradiated<br>portion (-V) |                                    |                                    |                                     |                                    |                                     | Amount of<br>abrasion<br>( $\mu\text{m}$ ) |
|-----------------------------------------|---------------------------------------|------------------------------------|------------------------------------|-------------------------------------|------------------------------------|-------------------------------------|--------------------------------------------|
|                                         | Initial                               | After<br>70,000<br>image<br>prints |                                    | Background<br>fouling<br>evaluation | Cleaning<br>property<br>evaluation | Dot<br>representation<br>evaluation |                                            |
|                                         |                                       | Initial                            | After<br>70,000<br>image<br>prints | Background<br>fouling<br>evaluation | Cleaning<br>property<br>evaluation | Dot<br>representation<br>evaluation |                                            |
| Example 16                              | 1                                     | 120                                | 145                                | F                                   | G                                  | E                                   | 9.8                                        |
| Example 37                              | 30                                    | 120                                | 150                                | E                                   | G                                  | E                                   | 9.8                                        |
| Example 38                              | 31                                    | 120                                | 145                                | G                                   | G                                  | E                                   | 9.8                                        |
| Example 39                              | 32                                    | 125                                | 155                                | E                                   | G                                  | E                                   | 9.8                                        |
| Example 40                              | 33                                    | 130                                | 165                                | E                                   | G                                  | E                                   | 9.8                                        |
| Example 41                              | 34                                    | 120                                | 145                                | G                                   | G                                  | E                                   | 9.8                                        |
| Example 42                              | 35                                    | 130                                | 155                                | E                                   | G                                  | E                                   | 9.8                                        |

149

As seen in the results shown in Table 9, it is found that the anti-background fouling property is improved by having a structure in which the intermediate layer is formed of a charge blocking layer and a moiré blocking layer.

## Image Bearing Member Manufacturing Example 36

Image bearing member 36 is manufactured in the same manner as in Image Bearing Member Manufacturing Example 1 except that the liquid dispersion 5 is used as the liquid of application for charge generating layer. The layer thickness of the charge generating layer is adjusted such that the transmission factor thereof for writing light having a wavelength of 407 nm is 20%.

## Image Bearing Member Manufacturing Example 37

Image bearing member 37 is manufactured in the same manner as in Image Bearing Member Manufacturing Example 1 except that the liquid dispersion 6 is used as the liquid of application for charge generating layer. The layer thickness of the charge generating layer is adjusted such that the transmission factor thereof for writing light having a wavelength of 407 nm is 20%.

## Image Bearing Member Manufacturing Example 38

Image bearing member 38 is manufactured in the same manner as in Image Bearing Member Manufacturing Example 36 except that the liquid of application for intermediate layer used in Image Bearing Member Manufacturing Example 36 is changed to the following component.

## Liquid of Application for Intermediate Layer

|                                                                                                                        |            |
|------------------------------------------------------------------------------------------------------------------------|------------|
| Surface treated rutile type titanium oxide                                                                             | 112 parts  |
| Alkyd resin (BECKOLITE M6401-50-S, manufactured by Dainippon Ink and Chemicals Incorporated, solid portion: 50%)       | 33.6 parts |
| Melamine resin (SUPERBECAKMINE L-121-60, manufactured by Dainippon Ink and Chemicals Incorporated, solid portion: 60%) | 18.7 parts |
| 2-butanone                                                                                                             | 260 parts  |

The surface treated rutile type titanium oxide is obtained by surface-treating the non-surface treated rutile type titanium oxide used in Image Bearing Member Manufacturing Example 1 with siloxane having 2 weight % based on the weight of the non-surface treated rutile type titanium oxide.

## Image Bearing Member Manufacturing Example 39

Image bearing member 39 is manufactured in the same manner as in Image Bearing Member Manufacturing Example 36 except that the liquid of application for intermediate layer used in Image Bearing Member Manufacturing Example 36 is changed to the following component.

## Liquid of Application for Intermediate Layer

|                                                                                                                  |            |
|------------------------------------------------------------------------------------------------------------------|------------|
| Non-surface treated zinc oxide (SAZEX #2000, manufactured by Sakai Chemical Industry Co., Ltd.)                  | 112 parts  |
| Alkyd resin (BECKOLITE M6401-50-S, manufactured by Dainippon Ink and Chemicals Incorporated, solid portion: 50%) | 33.6 parts |

150

-continued

|                                                                                                                        |            |
|------------------------------------------------------------------------------------------------------------------------|------------|
| Melamine resin (SUPERBECAKMINE L-121-60, manufactured by Dainippon Ink and Chemicals Incorporated, solid portion: 60%) | 18.7 parts |
| 2-butanone                                                                                                             | 260 parts  |

An intermediate layer is formed using the liquid of application mentioned above for intermediate layer on an aluminum board having a thickness of 1 mm in the same manner as described in manufacturing of the image bearing member 39 using the liquid of application for intermediate layer. The spectroscopic reflection spectrum of the intermediate layer is measured by a marketed spectral photometer (UV-3100, manufactured by Shimadzu Corporation). The absorption end (the upper limit of the wavelength of light which can be absorbed therein) of the intermediate layer is obtained from the spectroscopic reflection spectrum. The result of the absorption end of the titanium oxide mentioned above is about 388 nm.

25 An intermediate layer is formed using the liquid of application mentioned above for intermediate layer on an aluminum board having a thickness of 1 mm in the same manner as described in manufacturing of the image bearing member 39 using the liquid of application for intermediate layer. The spectroscopic reflection spectrum of the intermediate layer is measured by a marketed spectral photometer (UV-3100, manufactured by Shimadzu Corporation). The absorption end (the upper limit of the wavelength of light which can be absorbed therein) of the intermediate layer is obtained from the spectroscopic reflection spectrum. The result of the absorption end of the titanium oxide mentioned above is about 388 nm.

30 The Image bearing member 36 is implemented in a process cartridge as illustrated in FIG. 11 which is implemented in an image forming apparatus as shown in FIG. 10. The irradiation light source is a semi-conductor laser (image writing by a polygon mirror) emitting light having a wavelength of 407 nm. A contact type charging roller is used as the charging device. A transfer belt is used as the transfer device. A 380 nm LED, manufactured by Nichia Corporation, is as the discharging light source. The process conditions before the test of 50,000 image continuous printing of a chart in which characters corresponding to about 6% based on the total area of an A4 sheet are uniformly written are set as follows. The transmission factor of the charge generating layer is 20% and the transmission factor of the charge transport layer is 98% for the writing light wavelength (407 nm) for the image bearing member.

35 Charging device of image bearing member (non-irradiated portion): -900V

Developing bias: -650 V (negative/positive development)

40 Surface voltage at irradiated portion: -60 V

45 Evaluation is made based on the measurement of the voltage at irradiated portion on the image bearing member before and after 50,000 image continuous printing. The voltage is measured after 50,000 image printing while fixing the writing condition (amount of irradiation) to the value of the initial stage.

The surface voltage of non-irradiated portions and irradiated portions at the development portion of the image bearing member are measured for solid printing by the semi-conductor laser after -900 V charging on the image bearing member with a surface voltmeter placed on the developing position shown in FIG. 10. The result is shown in Table 10.

50 In addition, color representation is evaluated by outputting ISO/JIS-SCID image N1 (portrait) before and after the 50,000 image continuous printing.

151

## Example 44

The evaluation is made in the same manner as in Example 43 except that a 502 nm LED with a half value width of 15 nm (manufactured by Seiwa Electric Mfg. Co., Ltd.) is used instead. The result is shown in Table 10.

## Comparative Example 5

The evaluation is made in the same manner as in Example 44 except that the writing light source of Example 44 is changed to a light source of 440 nm LD (image writing by a polygon mirror). The amount of light is adjusted to have the same voltage as the surface voltage of the irradiated portion in the initial stage of Example 44. The result is shown in Table 10. The transmission factors of the charge generating layer and the charge transport layer for light having a wavelength of 440 nm for use in the image bearing member is 17% and 98% respectively.

## Example 45

The evaluation is made in the same manner as in Example 43 except that the image bearing member 36 is replaced with

152

irradiated portion in the initial stage of Example 43. The result is shown in Table 10. The transmission factors of the charge generating layer and the charge transport layer for light having a wavelength of 375 nm for use in the image bearing member is 26% and 77%, respectively.

## Comparative Example 6

The evaluation is made in the same manner as in Example 43 except that the image bearing member 36 is replaced with the image bearing member 39. The result is shown in Table 10. The transmission factor of the charge generating layer and the charge transport layer is 20% and 98%, respectively, for writing light having a wavelength of 407 nm for use in the image bearing member.

## Comparative Example 7

The evaluation is made in the same manner as in Comparative Example 5 except that the image bearing member 36 is replaced with the image bearing member 39. The result is shown in Table 10. The transmission factor of the charge generating layer and the charge transport layer is 20% and 98% for writing light having a wavelength of 375 nm for use in the image bearing member.

TABLE 10

|                       | Writing light wavelength (nm) | Discharging light wavelength (nm) | Initial                                        |                                            | After 50,000 printing                          |                                            |
|-----------------------|-------------------------------|-----------------------------------|------------------------------------------------|--------------------------------------------|------------------------------------------------|--------------------------------------------|
|                       |                               |                                   | Surface voltage at non-irradiated portion (-V) | Surface voltage at irradiated portion (-V) | Surface voltage at non-irradiated portion (-V) | Surface voltage at irradiated portion (-V) |
| Example 43            | 407                           | 380                               | 900                                            | 60                                         | 900                                            | 80                                         |
| Example 44            | 407                           | 502                               | 900                                            | 60                                         | 900                                            | 100                                        |
| Comparative Example 5 | 440                           | 502                               | 900                                            | 60                                         | 900                                            | 130                                        |
| Example 45            | 407                           | 380                               | 900                                            | 75                                         | 900                                            | 95                                         |
| Example 46            | 407                           | 380                               | 900                                            | 60                                         | 900                                            | 95                                         |
| Example 47            | 375                           | 380                               | 900                                            | 65                                         | 900                                            | 85                                         |
| Comparative Example 6 | 407                           | 380                               | 900                                            | 65                                         | 900                                            | 120                                        |
| Comparative Example 7 | 440                           | 502                               | 900                                            | 65                                         | 900                                            | 130                                        |

the image bearing member 37. The result is shown in Table 10. The transmission factor of the charge generating layer and the charge transport layer is 18% and 98% for writing light having a wavelength of 407 nm.

## Example 46

The evaluation is made in the same manner as in Example 43 except that the image bearing member 36 is replaced with the image bearing member 38. The result is shown in Table 10. The transmission factor of the charge generating layer and the charge transport layer is 17% and 98% for writing light having a wavelength of 407 nm.

## Example 47

The evaluation is made in the same manner as in Example 43 except that the writing light source of Example 43 is changed to a light source of 375 nm LD (image writing by a polygon mirror) and the image bearing member 36 is replaced with the image bearing member 39. The amount of light is adjusted to have the same voltage as the surface voltage of the

As seen in the result of the test chart, the obtained image in Example 43 after 50,000 image output is almost as same as the image obtained at the initial stage but the obtained images in Comparative Example 5 are slightly off balance in color after 50,000 image output.

When the surface voltage at the irradiated portion in Example 43 is compared with the surface voltage at the irradiated portion in Example 45, the surface voltage at the irradiated portion in Example 43 is low. It is found that asymmetry of the coupler composition of the azo pigments for use in Example 43 contributes to the improvement on the sensitivity.

The effect of reducing the rise of the residual voltage is relatively small in Example 46 in which the surface treated titanium oxide is contained in the intermediate layer in comparison with the case in which the non-surface treated titanium oxide is used as in Example 43.

When the wavelength of writing light is set to be 375 nm and the writing light is absorbed by metal oxide (zinc oxide) contained in the intermediate layer as in Example 47, the rise of the voltage at irradiated portions after repetitive use is relatively small in comparison with those in the cases in

## 153

which the writing light is not absorbed by the metal oxide as in Comparative Examples 6 and 7.

This document claims priority and contains subject matter related to Japanese Patent Applications Nos. 2006-028493, filed on Feb. 6, 2006, 2006-028494, filed on Feb. 6, 2006, 2007-004924, filed on Jan. 12, 2007, and 2007-004925, filed on Jan. 12, 2007, the entire contents of which are incorporated herein by reference.

Having now fully described the invention, it will be apparent to one of ordinary skill in the art that many changes and modifications can be made thereto without departing from the spirit and scope of the invention as set forth therein.

What is claimed as new and desired to be secured by Letters Patent of the United States is:

1. An image forming method comprising:  
charging an image bearing member comprising a substrate, an intermediate layer comprising a charge blocking layer comprising N-methoxy methylated nylon and a moiré prevention layer having a layer thickness of from 2 to 5  $\mu\text{m}$  which comprises a metal oxide and is provided on the charge blocking layer, a photosensitive layer comprising a charge transport layer and a charge generating layer comprising an organic charge generating material;  
writing a latent electrostatic image on the image bearing member by irradiating the image bearing member with light having a wavelength shorter than 450 nm which the metal oxide absorbs so that carriers can be generated; developing the latent electrostatic image with a toner to form a visualized image;  
transferring the visualized image to a recording medium;  
fixing the transferred image on the recording medium; and discharging residual charges on the image bearing member.
2. The image forming method according to claim 1, wherein the discharging device irradiates the image bearing member with light having a wavelength shorter than 450 nm which the metal oxide in the intermediate layer absorbs so that carriers can be generated.
3. The image forming method according to claim 1, comprising a plurality of charging processes and writing processes.
4. An image forming apparatus comprising:  
an image bearing member configured to bear a latent electrostatic image comprising;  
a substrate;  
an intermediate layer comprising a charge blocking layer comprising N-methoxy methylated nylon and a moiré prevention layer having a layer thickness of from 2 to 5  $\mu\text{m}$  which comprises a metal oxide and is provided on the charge blocking layer; and  
a photosensitive layer comprising a charge transport layer and a charge generating layer comprising an organic charge generating material;
5. The image forming apparatus according to claim 4, comprising a charging device configured to charge the image bearing member;
6. The image forming apparatus according to claim 5, comprising a writing device configured to write the latent electrostatic image on the image bearing member by irradiating the image bearing member with light having a wavelength shorter than 450 nm which is absorbed by the metal oxide in the moiré prevention layer to generate carriers; a developing device configured to develop the latent electrostatic image with a toner to form a visualized image;
7. The image forming apparatus according to claim 6, comprising a transfer device configured to transfer the visualized image to a recording medium;
8. The image forming apparatus according to claim 7, comprising a fixing device configured to fix the transferred image on the recording image; and
9. The image forming apparatus according to claim 8, comprising a discharging device configured to optically discharge residual charges on the image bearing member.
10. The image forming apparatus according to claim 4, wherein the metal oxide is a non-surface treated metal oxide.
11. The image forming apparatus according to claim 4, wherein the metal oxide is a rutile type titanium oxide and the writing device irradiates the image bearing member with light having a wavelength shorter than 410 nm.
12. The image forming apparatus according to claim 4, wherein the rutile type titanium oxide is a non-surface treated rutile type titanium oxide.
13. The image forming apparatus according to claim 4, wherein the transmission factor of the charge generating layer for the writing light is from 10 to 25%.
14. The image forming apparatus according to claim 4, wherein the transmission factor of the charge transport layer for the writing light is not less than 30%.
15. The image forming apparatus according to claim 4, wherein a protective layer is provided on the photosensitive layer.
16. The image forming apparatus according to claim 4, wherein the transmission factor of the protective layer for the writing light is not less than 30%.
17. The image forming apparatus according to claim 4, wherein the charge blocking layer comprises an insulating material and has a thickness of from 0.1 to less than 2.0  $\mu\text{m}$ .
18. The image forming apparatus according to claim 4, wherein the moiré prevention layer further comprises a binder resin and a ratio in volume of the metal oxide in the moiré prevention layer to the binder resin is from 1 to 3.
19. The image forming apparatus according to claim 4, wherein the discharging device comprises a light source irradiating the image bearing member with light having a wavelength shorter than 450 nm which the metal oxide in the intermediate layer absorbs so that carriers can be generated.
20. The image forming apparatus according to claim 4, comprising a plurality of image bearing members, charging devices, and writing devices.
21. The image forming apparatus according to claim 4, wherein the image bearing member, the charging device and the writing devices are integrally detachably attached to the image forming apparatus.
22. A process cartridge comprising:  
an image bearing member configured to bear a latent electrostatic image comprising a substrate, a photosensitive layer and an intermediate layer comprising a charge blocking layer comprising N-methoxy methylated nylon and a moiré prevention layer having a layer thickness of from 2 to 5  $\mu\text{m}$  which comprises a metal oxide and is provided on the charge blocking layer;
23. The process cartridge according to claim 22, comprising a charging device configured to charge the image bearing member; and
24. The process cartridge according to claim 23, comprising a writing device configured to write the latent electrostatic image on the image bearing member by irradiating the image bearing member with light having a wavelength shorter than 450 nm which the metal oxide in the moiré prevention layer absorbs so that carriers can be generated.

## 154

a transfer device configured to transfer the visualized image to a recording medium;

a fixing device configured to fix the transferred image on the recording image; and

a discharging device configured to optically discharge residual charges on the image bearing member.

5. The image forming apparatus according to claim 4, wherein the metal oxide is a non-surface treated metal oxide.

10. The image forming apparatus according to claim 4, wherein the metal oxide is a rutile type titanium oxide and the writing device irradiates the image bearing member with light having a wavelength shorter than 410 nm.

15. The image forming apparatus according to claim 6, wherein the rutile type titanium oxide is a non-surface treated rutile type titanium oxide.

20. The image forming apparatus according to claim 4, wherein the transmission factor of the charge generating layer for the writing light is from 10 to 25%.

25. The image forming apparatus according to claim 4, wherein the transmission factor of the charge transport layer for the writing light is not less than 30%.

30. The image forming apparatus according to claim 4, wherein a protective layer is provided on the photosensitive layer.

35. The image forming apparatus according to claim 10, wherein the transmission factor of the protective layer for the writing light is not less than 30%.

40. The image forming apparatus according to claim 4, wherein the charge blocking layer comprises an insulating material and has a thickness of from 0.1 to less than 2.0  $\mu\text{m}$ .

45. The image forming apparatus according to claim 4, wherein the moiré prevention layer further comprises a binder resin and a ratio in volume of the metal oxide in the moiré prevention layer to the binder resin is from 1 to 3.

50. The image forming apparatus according to claim 4, wherein the discharging device comprises a light source irradiating the image bearing member with light having a wavelength shorter than 450 nm which the metal oxide in the intermediate layer absorbs so that carriers can be generated.

55. The image forming apparatus according to claim 4, comprising a plurality of image bearing members, charging devices, and writing devices.

60. The image forming apparatus according to claim 4, wherein the image bearing member, the charging device and the writing devices are integrally detachably attached to the image forming apparatus.

65. A process cartridge comprising:

an image bearing member configured to bear a latent electrostatic image comprising a substrate, a photosensitive layer and an intermediate layer comprising a charge blocking layer comprising N-methoxy methylated nylon and a moiré prevention layer having a layer thickness of from 2 to 5  $\mu\text{m}$  which comprises a metal oxide and is provided on the charge blocking layer;

a charging device configured to charge the image bearing member; and

a writing device configured to write the latent electrostatic image on the image bearing member by irradiating the image bearing member with light having a wavelength shorter than 450 nm which the metal oxide in the moiré prevention layer absorbs so that carriers can be generated.

\* \* \* \* \*